



US009069267B2

(12) **United States Patent**  
**Kaku et al.**

(10) **Patent No.:** **US 9,069,267 B2**  
(45) **Date of Patent:** **Jun. 30, 2015**

(54) **ELECTROPHOTOGRAPHIC PHOTOSENSITIVE MEMBER, PROCESS CARTRIDGE, AND ELECTROPHOTOGRAPHIC APPARATUS**

(71) **Applicant:** **CANON KABUSHIKI KAISHA**,  
Tokyo (JP)

(72) **Inventors:** **Kenichi Kaku**, Newcastle Upon Tyne (GB); **Michiyo Sekiya**, Atami (JP); **Kunihiro Sekido**, Suntou-gun (JP); **Atsushi Okuda**, Yokohama (JP); **Nobuhiro Nakamura**, Mishima (JP); **Yota Ito**, Mishima (JP); **Hiroyuki Tomono**, Numazu (JP); **Yuka Ishiduka**, Suntou-gun (JP)

(73) **Assignee:** **CANON KABUSHIKI KAISHA**,  
Tokyo (JP)

(\*) **Notice:** Subject to any disclaimer, the term of this patent is extended or adjusted under 35 U.S.C. 154(b) by 0 days.

(21) **Appl. No.:** **13/930,368**

(22) **Filed:** **Jun. 28, 2013**

(65) **Prior Publication Data**

US 2014/0004453 A1 Jan. 2, 2014

(30) **Foreign Application Priority Data**

Jun. 29, 2012 (JP) ..... 2012-147158  
Apr. 25, 2013 (JP) ..... 2013-093091  
Jun. 20, 2013 (JP) ..... 2013-130014

(51) **Int. Cl.**  
**G03G 5/05** (2006.01)  
**G03G 5/043** (2006.01)  
(Continued)

(52) **U.S. Cl.**  
CPC ..... **G03G 5/043** (2013.01); **G03G 5/0651** (2013.01); **G03G 5/0607** (2013.01);  
(Continued)

(58) **Field of Classification Search**  
CPC ... G03G 5/055; G03G 5/0605; G03G 5/0607;  
G03G 5/0648; G03G 5/0651; G03G 5/065  
USPC ..... 430/60, 63, 65, 58.25, 58.5, 58.7  
See application file for complete search history.

(56) **References Cited**

**U.S. PATENT DOCUMENTS**

4,442,193 A 4/1984 Chen et al.  
4,562,132 A 12/1985 Ong et al.

(Continued)

**FOREIGN PATENT DOCUMENTS**

EP 2 317 393 A1 5/2011  
JP 1-206349 A 8/1989

(Continued)

**OTHER PUBLICATIONS**

English language machine translation of JP 2004-093801 (Mar. 2004).\*

(Continued)

*Primary Examiner* — Christopher Rodee

(74) **Attorney, Agent, or Firm:** Fitzpatrick, Cella, Harper and Scinto

(57) **ABSTRACT**

An electrophotographic photosensitive member has a laminated body, and a hole transporting layer formed on the laminated body, wherein the laminated body is a laminated body having a conductive support, an electron transporting layer and a charge generating layer. When an impedance is measured by forming a circular-shaped gold electrode having a thickness of 300 nm and a diameter of 10 mm on a surface of the charge generating layer of the laminated body by sputtering, and applying an alternating electric field of 100 mV and 0.1 Hz between the conductive support and the gold electrode, the laminated body of the electrophotographic photosensitive member satisfies the following expression (1):

$$R_{\text{opt}}/R_{\text{dark}} \leq 0.95 \quad (1)$$

**8 Claims, 5 Drawing Sheets**



| (51) Int. Cl. |                                                                                                                                                                                                                                                                        | FOREIGN PATENT DOCUMENTS |    |                             |
|---------------|------------------------------------------------------------------------------------------------------------------------------------------------------------------------------------------------------------------------------------------------------------------------|--------------------------|----|-----------------------------|
|               | <i>G03G 5/06</i>                                                                                                                                                                                                                                                       | (2006.01)                | JP | 5-279582 A 10/1993          |
|               | <i>G03G 5/04</i>                                                                                                                                                                                                                                                       | (2006.01)                | JP | 7-70038 A 3/1995            |
|               | <i>G03G 5/07</i>                                                                                                                                                                                                                                                       | (2006.01)                | JP | 9-151157 A 6/1997           |
|               | <i>G03G 5/14</i>                                                                                                                                                                                                                                                       | (2006.01)                | JP | 11-119458 A 4/1999          |
| (52) U.S. Cl. |                                                                                                                                                                                                                                                                        |                          | JP | 2003-330209 A 11/2003       |
| CPC .....     | <i>G03G 5/0648</i> (2013.01); <i>G03G 5/055</i> (2013.01); <i>G03G 5/0605</i> (2013.01); <i>G03G 5/04</i> (2013.01); <i>G03G 5/0589</i> (2013.01); <i>G03G 5/0592</i> (2013.01); <i>G03G 5/075</i> (2013.01); <i>G03G 5/076</i> (2013.01); <i>G03G 5/142</i> (2013.01) |                          | JP | 2004093801 A * 3/2004 ..... |
|               |                                                                                                                                                                                                                                                                        |                          | JP | 2005-189764 A 7/2005        |
|               |                                                                                                                                                                                                                                                                        |                          | JP | 2006-30698 A 2/2006         |
|               |                                                                                                                                                                                                                                                                        |                          | JP | 2009-505156 A 2/2009        |
|               |                                                                                                                                                                                                                                                                        |                          | JP | 2010-145506 A 7/2010        |
|               |                                                                                                                                                                                                                                                                        |                          | JP | 4594444 B2 12/2010          |
|               |                                                                                                                                                                                                                                                                        |                          | WO | WO 2012/002516 A1 * 1/2012  |

## (56) References Cited

## U.S. PATENT DOCUMENTS

|                 |         |                                 |
|-----------------|---------|---------------------------------|
| 4,992,349 A     | 2/1991  | Chen et al.                     |
| 5,455,135 A     | 10/1995 | Maruyama et al.                 |
| 5,468,583 A     | 11/1995 | Gruenbaum et al.                |
| 5,604,061 A     | 2/1997  | Sekido et al.                   |
| 5,641,599 A *   | 6/1997  | Markovics et al. .... 430/58.25 |
| 5,693,443 A     | 12/1997 | Nakamura et al.                 |
| 5,863,688 A     | 1/1999  | Watanabe et al.                 |
| 6,110,628 A     | 8/2000  | Sekiya et al.                   |
| 6,228,546 B1    | 5/2001  | Kashizaki et al.                |
| 6,372,397 B1    | 4/2002  | Maruyama et al.                 |
| 6,436,597 B2    | 8/2002  | Maruyama et al.                 |
| 6,664,014 B1    | 12/2003 | Kikuchi et al.                  |
| 6,991,881 B2    | 1/2006  | Ogaki et al.                    |
| 6,994,941 B2    | 2/2006  | Tanaka et al.                   |
| 7,001,699 B2    | 2/2006  | Tanaka et al.                   |
| 7,045,261 B2    | 5/2006  | Tanaka et al.                   |
| 7,141,341 B2    | 11/2006 | Sekido et al.                   |
| 7,171,142 B2    | 1/2007  | Kawakami et al.                 |
| 7,378,205 B2    | 5/2008  | Sekiya et al.                   |
| 7,541,124 B2    | 6/2009  | Molaira et al.                  |
| 7,585,604 B2    | 9/2009  | Ogaki et al.                    |
| 7,645,547 B2    | 1/2010  | Okuda et al.                    |
| 7,655,370 B2    | 2/2010  | Kitamura et al.                 |
| 7,702,256 B2    | 4/2010  | Nukada et al.                   |
| 7,910,274 B2    | 3/2011  | Tanaka et al.                   |
| 7,927,774 B2    | 4/2011  | Ogaki et al.                    |
| 8,088,541 B2    | 1/2012  | Tanaka et al.                   |
| 8,343,699 B2    | 1/2013  | Nagasaki et al.                 |
| 8,455,170 B2    | 6/2013  | Nakamura et al.                 |
| 8,465,889 B2    | 6/2013  | Sekido et al.                   |
| 8,481,236 B2    | 7/2013  | Tanaka et al.                   |
| 8,524,430 B2    | 9/2013  | Takagi et al.                   |
| 8,546,050 B2    | 10/2013 | Maruyama et al.                 |
| 2007/0026332 A1 | 2/2007  | Ferrari et al.                  |
| 2008/0280220 A1 | 11/2008 | Chen et al.                     |
| 2010/0062171 A1 | 3/2010  | Kaku et al.                     |
| 2011/0143273 A1 | 6/2011  | Sekido et al.                   |
| 2011/0158683 A1 | 6/2011  | Okuda et al.                    |
| 2012/0033994 A1 | 2/2012  | Tanaka et al.                   |
| 2012/0114375 A1 | 5/2012  | Fujii et al.                    |
| 2012/0230727 A1 | 9/2012  | Sekido et al.                   |
| 2012/0301181 A1 | 11/2012 | Ogaki et al.                    |
| 2012/0301182 A1 | 11/2012 | Anezaki et al.                  |
| 2013/0202326 A1 | 8/2013  | Shida et al.                    |
| 2013/0202327 A1 | 8/2013  | Murai et al.                    |
| 2013/0236823 A1 | 9/2013  | Noguchi et al.                  |
| 2013/0316283 A1 | 11/2013 | Fujii et al.                    |
| 2013/0323632 A1 | 12/2013 | Fujii et al.                    |

## FOREIGN PATENT DOCUMENTS

|    |                     |              |
|----|---------------------|--------------|
| JP | 5-279582 A          | 10/1993      |
| JP | 7-70038 A           | 3/1995       |
| JP | 9-151157 A          | 6/1997       |
| JP | 11-119458 A         | 4/1999       |
| JP | 2003-330209 A       | 11/2003      |
| JP | 2004093801 A *      | 3/2004 ..... |
| JP | 2005-189764 A       | 7/2005       |
| JP | 2006-30698 A        | 2/2006       |
| JP | 2009-505156 A       | 2/2009       |
| JP | 2010-145506 A       | 7/2010       |
| JP | 4594444 B2          | 12/2010      |
| WO | WO 2012/002516 A1 * | 1/2012       |

## OTHER PUBLICATIONS

- Jones, et al., "Cyanonaphthalene Diimide Semiconductors for Air-Stable, Flexible, and Optically Transparent n-Channel Field-Effect Transistors", Chemistry of Materials, vol. 19, No. 11, May 29, 2007, pp. 2703-2705.
- Callahan, et al., "Syntheses of Phencyclone Analogues. Applications for NMR Studies of Hindered Rotations and Magnetic Anisotropy in Crowded Diels-Alder Adducts", Chem. Educator, vol. 6, 2001, pp. 227-234.
- Kato, et al., "Nitration of Phenanthrenequinone", Journal of Synthetic Organic Chemistry, Japan, vol. 15, 1957, pp. 29-32.
- Kato, et al., "Syntheses of Amino-phenanthrenequinones by the Reduction of Nitro Compounds", Journal of Synthetic Organic Chemistry, Japan, vol. 15, 1957, pp. 32-34.
- Yamada, et al., "Synthesis and Properties of Diamino-Substituted Dipyrido [3,2-a:2',3'-c]phenazine", Bulletin of the Chemical Society of Japan, vol. 65, No. 4, 1992, pp. 1006-1011.
- Qian, et al., "4-Amino-1, 8-dicyanonaphthalene derivatives as novel fluorophore and fluorescence switches: efficient synthesis and fluorescence enhancement induced by transition metal ions and protons", Tetrahedron Letters, vol. 43, 2002, pp. 2991-2994.
- Xiao, et al., "Novel highly efficient fluoroionophores with a peri-effect and strong electron-donating receptors: TICT-promoted PET and signaling response to transition metal cations with low background emission", Tetrahedron Letters, vol. 44, 2003, pp. 2087-2091.
- Miyamura, et al., "Polymer Incarcerated Gold Catalyzed Aerobic Oxidation of Hydroquinones and Their Derivatives", Chemistry Letters, vol. 37, No. 3, 2008, pp. 360-361.
- Okada, et al., "Synthesis and Properties of a Novel Electron Transporting Compound, 3,3'-dialkyl-4,4'-bisnaphthylquinone (DBNQ)", PPCI/Japan Hardcopy '98 Papers, 1998, pp. 207-210.
- Jones, et al., "Tuning Orbital Energetics in Arylene Diimide Semiconductors. Materials Design for Ambient Stability of n-Type Charge Transport", J. Am. Chem. Soc., vol. 129, 2007, pp. 15259-15278.
- Yamashita, et al., "Crosslinking Agent Handbook", 1981, pp. 536-605.
- European Search Report dated Oct. 22, 2013 in European Application No. 13174199.3.
- Okuda, et al., U.S. Appl. No. 14/009,723, 371(c) Date: Oct. 3, 2013.
- Okuda, et al., U.S. Appl. No. 14/009,721, 371(c) Date: Oct. 3, 2013.
- Tokimitsu, et al., U.S. Appl. No. 13/913,910, filed Jun. 10, 2013.
- Sekiya, et al., U.S. Appl. No. 13/930,341, filed Jun. 28, 2013.
- Okuda, et al., U.S. Appl. No. 13/930,383, filed Jun. 28, 2013.
- Fujii, et al., U.S. Appl. No. 13/972,688, filed Aug. 21, 2013.

\* cited by examiner

FIG. 1



**FIG. 2****FIG. 3**

FIG. 4



*FIG. 5A**FIG. 5B*

FIG. 6



## 1

**ELECTROPHOTOGRAPHIC  
PHOTOSENSITIVE MEMBER, PROCESS  
CARTIDGE, AND  
ELECTROPHOTOGRAPHIC APPARATUS**

**BACKGROUND OF THE INVENTION**

**1. Field of the Invention**

The present invention relates to an electrophotographic photosensitive member, and a process cartridge and an electrophotographic apparatus having an electrophotographic photosensitive member.

**2. Description of the Related Art**

As electrophotographic photosensitive members used for process cartridges and electrophotographic apparatuses, electrophotographic photosensitive members containing an organic photoconductive substance mainly prevail at present. The electrophotographic photosensitive member generally has a support and a photosensitive layer formed on the support. Then, an undercoating layer is provided between the support and the photosensitive layer in order to suppress the charge injection from the support side to the photosensitive layer (charge generating layer) side and to suppress the generation of image defects such as fogging.

Charge generating substances having a higher sensitivity have recently been used. However, such a problem arises that a charge is liable to be retained in a photosensitive layer due to that the amount of charge generated becomes large along with making higher the sensitivity of the charge generating substance, and the ghost is liable to occur. Specifically, a phenomenon of a so-called positive ghost, in which the density of only portions irradiated with light in the preceding rotation time becomes high, is liable to occur in a printed-out image.

A technology of reducing such a ghost phenomenon is disclosed in which an undercoating layer is made to be a layer (hereinafter, also referred to as an electron transporting layer) having an electron transporting capability by incorporating an electron transporting substance in the undercoating layer. National Publication of International Patent Application No. 2009-505156 discloses a condensed polymer (electron transporting substance) having an aromatic tetracarbonylbisimide skeleton and a crosslinking site, and an electron transporting layer containing a polymer with a crosslinking agent. Japanese Patent Application Laid-Open No. 2003-330209 discloses that a polymer of an electron transporting substance having a non-hydrolyzable polymerizable functional group is incorporated in an undercoating layer. Japanese Patent Application Laid-Open No. 2005-189764 discloses a technology of making the electron mobility of an undercoating layer to be  $10^{-7} \text{ cm}^2/\text{V}\cdot\text{sec}$  or more in order to improve the electron transporting capability.

The demand for the quality of electrophotographic images has recently been raised increasingly, and the allowable range for the early-stage positive ghost and the long-term positive ghost after repeated use has remarkably become severe. As a result of exhaustive studies by the present inventors, it has been found that with respect to the reduction of the positive ghost, technologies disclosed in National Publication of International Patent Application No. 2009-505156 and Japanese Patent Application Laid-Open Nos. 2003-330209 and 2005-189764 still have room for improvement.

**SUMMARY OF THE INVENTION**

It is an object of the present invention to provide an electrophotographic photosensitive member reduced in the posi-

## 2

tive ghost in the early stage and after the long-term repeated use, and a process cartridge and an electrophotographic apparatus having the electrophotographic photosensitive member.

The present invention relates to an electrophotographic photosensitive member including a laminated body, and a hole transporting layer formed on the laminated body, wherein the laminated body has a conductive support, an electron transporting layer formed on the conductive support, and a charge generating layer formed on the electron transporting layer; and the laminated body satisfies the following expression (1):

$$R_{\text{opt}}/R_{\text{dark}} \leq 0.95 \quad (1),$$

where, in the above expression (1),  $R_{\text{opt}}$  represents impedance of the laminated body measured by the steps of: forming, on a surface of the charge generating layer, a circular-shaped gold electrode having a thickness of 300 nm and a diameter of 10 mm by sputtering, and applying, between the conductive support and the circular-shaped gold electrode, an alternating electric field having a voltage of 100 mV and a frequency of 0.1 Hz while irradiating the surface of the charge generating layer with light having intensity of  $30 \mu\text{J}/\text{cm}^2\cdot\text{sec}$ , and measuring the impedance, and  $R_{\text{dark}}$  represents impedance of the laminated body measured by the steps of: forming, on a surface of the charge generating layer, a circular-shaped gold electrode having a thickness of 300 nm and a diameter of 10 mm by sputtering, and applying, between the conductive support and the circular-shaped gold electrode, an alternating electric field having a voltage of 100 mV and a frequency of 0.1 Hz without irradiating the surface of the charge generating layer with light, and measuring the impedance.

The present invention relates also to a process cartridge detachably attachable to a main body of an electrophotographic apparatus, wherein the process cartridge integrally supports: the electrophotographic photosensitive member, and at least one unit selected from the group consisting of a charging unit, a developing unit, a transfer unit and a cleaning unit.

The present invention relates also to an electrophotographic apparatus having the electrophotographic photosensitive member, and a charging unit, a light irradiation unit, a developing unit and a transfer unit.

The present invention can provide an electrophotographic photosensitive member reduced in the positive ghost in the early stage and after the long-term repeated use, and a process cartridge and an electrophotographic apparatus having the electrophotographic photosensitive member.

Further features of the present invention will become apparent from the following description of exemplary embodiments with reference to the attached drawings.

**BRIEF DESCRIPTION OF THE DRAWINGS**

FIG. 1 is a diagram illustrating one example of an outline constitution of a determination apparatus to carry out a determination method according to the present invention.

FIG. 2 is a diagram illustrating typical examples of  $R_{\text{dark}}$  and  $R_{\text{opt}}$  when the determination method according to the present invention is carried out.

FIG. 3 is a diagram illustrating an outline constitution of an electrophotographic apparatus having a process cartridge having an electrophotographic photosensitive member.

FIG. 4 is a diagram to describe an image for ghost evaluation used in ghost image evaluation.

FIG. 5A is a diagram to describe a one-dot keima (similar to knight's move) pattern image.

FIG. 5B is a diagram to describe a one-dot pattern image used after long-term repeated use.

FIG. 6 is a diagram illustrating one example of a layer constitution of the electrophotographic photosensitive member.

#### DESCRIPTION OF THE EMBODIMENTS

Preferred embodiments of the present invention will now be described in detail in accordance with the accompanying drawings.

First, a determination method (hereinafter, referred to as "determination method according to the present invention") for determining whether or not an electrophotographic photosensitive member satisfies the relation of the above expression (1) of the present invention will be described. The temperature and humidity condition when the determination method according to the present invention is carried out may be under the environment of using an electrophotographic apparatus having an electrophotographic photosensitive member. The condition can be under the normal temperature and normal humidity environment (23° C.±3° C., 50%±20% RH). The above measuring method involves using a laminated body having a conductive support, an electron transporting layer and a charge generating layer in this order.

At this time, a hole transporting layer is peeled off an electrophotographic photosensitive member having a laminated body and the hole transporting layer formed on the laminated body to thereby make a laminated body (hereinafter, also referred to as "electrophotographic photosensitive member for determination"), which can be used as a determination object. A method of peeling a hole transporting layer includes a method in which an electrophotographic photosensitive member is immersed in a solvent which dissolves the hole transporting layer and hardly dissolves an electron transporting layer and a charge generating layer, and a method in which the hole transporting layer is ground.

As the solvent which dissolves a hole transporting layer and hardly dissolves an electron transporting layer and a charge generating layer, a solvent used for a coating liquid for the hole transporting layer can be used. The kinds of the solvent will be described later. An electrophotographic photosensitive member is immersed in the solvent for a hole transporting layer to be dissolved in the solvent, and thereafter dried to thereby obtain an electrophotographic photosensitive member for determination. That a hole transporting layer may have been peeled off can be confirmed, for example, by that no resin components of the hole transporting layer cannot be observed by the ATR method (total reflection method) in the FTIR measuring method.

A method of grinding a hole transporting layer involves, for example, using a drum and tape grinding apparatus made by Canon Inc. and using a wrapping tape (C2000, made by Fujifilm Corp.). At this time, the measurement can be carried out at the time when all of the hole transporting layer is removed while the thickness of the hole transporting layer is successively measured so as not to be ground up to a charge generating layer due to excessive grinding of the hole transporting layer and the surface of an electrophotographic photosensitive member is being observed. The case where a thickness of the charge generating layer of 0.10  $\mu\text{m}$  or more is left after the grinding is carried out up to the charge generating layer has been verified to give nearly the same value by the above-mentioned determination method as the case where the grinding is carried out not up to the charge generating layer. Therefore, even if not only a hole transporting layer but also up to a charge generating layer is ground, in the case where

the thickness of the charge generating layer is 0.10  $\mu\text{m}$  or more, the above-mentioned determination method can be used.

FIG. 1 illustrates one example of an outline constitution of a determination apparatus to carry out the determination method according to the present invention. In FIG. 1, reference numeral 101 denotes a part of an electrophotographic photosensitive member for determination (laminated body) obtained by cutting out the electrophotographic photosensitive member for determination into 2 cm (peripheral direction)×4 cm (long axis direction). Reference numeral 102 denotes a circular-shaped gold electrode having a diameter of 10 mm and a thickness of 300 nm formed on a surface of a charge generating layer of the above-mentioned laminated body by sputtering. A method for sputtering a gold electrode is not especially limited, but a Quick Auto Coater (SC-707AT) made by SANYU Electronic Co., Ltd., or the like can be used. The sputtering is carried out until the thickness of a gold electrode becomes 300 nm while a discharge current of 10 mA is maintained with a constitution in which a gold target is arranged over a surface of the charge generating layer, to thereby fabricate the gold electrode. Reference numeral 103 denotes an impedance measuring instrument, and it is illustrated that a lead wire 105 is connected to the gold electrode 102 on the charge generating layer and the conductive support. Reference numeral 104 denotes an apparatus to oscillate laser light (apparatus to carry out light irradiation), and reference numeral 106 denotes irradiation light. As the impedance measuring instrument, for example, a measuring module being a combination of SI-1287-electrochemical-interface, SI-1260-impedance-gain-phase-analyzer and 1296-dielectric-interface, made by Toyo Corp., is used. The impedance ( $R_{\text{dark}}$ ) under the condition of no light irradiation in the present invention is measured by covering the whole apparatus of FIG. 1 with a blackout film to shield indoor light, without light irradiation by the apparatus 104 to oscillate laser light. Then, an alternating electric field of 100 mV is applied between the conductive support of the laminated body and the gold electrode, and the impedance is measured by sweeping the frequency from a high frequency of 1 MHz to a low frequency of 0.1 Hz to thereby acquire an impedance ( $R_{\text{dark}}$ ) at 0.1 Hz. That is, the impedance denotes an impedance measured by applying an alternating electric field of 100 mV and 0.1 Hz between the conductive support of the laminated body and the gold electrode under the condition of no irradiation of a surface of the charge generating layer with light. Then, the impedance ( $R_{\text{opt}}$ ) under the condition of light irradiation is measured as in the above-mentioned case of no light irradiation, except for continuously oscillating irradiation light 106 from the apparatus 104 to oscillate laser light to the electrophotographic photosensitive member for determination 101. With respect to irradiation light when the  $R_{\text{opt}}$  is measured, light of a wavelength suitable for the light absorption property of the charge generating layer is used, and irradiation with the light having an enough intensity to saturate the charge generating layer with light-excited carriers generated from a charge generating substance is carried out. Specifically, with irradiation with light having a wavelength of 400 nm to 800 nm and an irradiation intensity of 30  $\mu\text{J}/\text{cm}^2\text{-sec}$  or more, light-excited carriers can be saturated sufficiently. Examples of the present invention used such an irradiation intensity that the impedance ( $R_{\text{opt}}$ ) under light irradiation is saturated at the lowest value. Specifically, irradiation with laser light having a wavelength of 680 nm and an irradiation intensity of 30  $\mu\text{J}/\text{cm}^2\text{-sec}$  was carried out. As to a time for the light irradiation, the light irradiation with the above irradiation intensity carried out for a period of time of 50

1 second or more can provide sufficient saturation of light-excited carriers, but the measurement of the impedance takes several minutes. The impedance is measured while the light irradiation is carried out at the above irradiation intensity, with the result that light-excited carriers are saturated sufficiently. That is, the impedance denotes an impedance measured by applying an alternating electric field of 100 mV and 0.1 Hz between the conductive support and the gold electrode under the condition of irradiation of the surface of the charge generating layer with light having an irradiation intensity of 30  $\mu\text{J}/\text{cm}^2\text{-sec}$ . Whether or not the electrophotographic photosensitive member satisfies the relation of the above expression (1) can be determined by calculating the ratio of the measured  $R_{\text{dark}}$  and  $R_{\text{opt}}$ .

FIG. 2 illustrates typical examples of  $R_{\text{dark}}$  and  $R_{\text{opt}}$ . In FIG. 2, the frequency dependency of the impedances ( $R_{\text{dark}}$  and  $R_{\text{opt}}$ ) measured by the above method is illustrated. Particularly on the low-frequency side, the change in the impedance becomes large depending on the presence and absence of light irradiation. That is, the ratio of  $R_{\text{opt}}/R_{\text{dark}}$  at 0.1 Hz indicates 0.95 or less.

In the present invention, in order to reduce the positive ghost in the early stage and after repeated use, the ratio of  $R_{\text{opt}}/R_{\text{dark}}$  is 0.95 or less. The present inventors presume the reason that the satisfaction of the relation of the above expression (1) can reduce the positive ghost in the early stage and after repeated use, as follows.

That is, in the case of an electrophotographic photosensitive member provided with an electron transporting layer (undercoating layer), a charge generating layer and a hole transporting layer on a support in this order, in portions on which irradiation light (image-irradiation light) has fallen, out of charges (holes and electrons) generated in the charge generating layer, holes are injected in the hole transporting layer, and electrons are injected in the electron transporting layer and transfer to the support. However, if electrons generated in the charge generating layer by light excitation do not completely move in the electron transporting layer before the following charging, the charge is retained in the charge generating layer, still causing electron movement even during the following charging. The electrons slow in movement are liable to cause the local decrease in the charging capability of portions irradiated with light after the following charging. These phenomena are caused also in the repeated use of an electrophotographic photosensitive member, and the charge retained in the charge generating layer is liable to increase gradually. The charge retained in the charge generating layer makes a cause of generating the positive ghost in the early stage and after repeated use.

Then, if the laminated body satisfies the relation of the above expression (1), the reception and delivery of electrons (electrons derived from light excitation and retained in the charge generating layer) slow in movement at the interface between the electron transporting layer and the charge generating layer is conceivably promoted. That is, in the determination method according to the present invention, if the resistance between the conductive support and the gold electrode does not change depending on the presence and absence of light irradiation in the state that the charge generating layer of the laminated body is saturated with the charge derived from light excitation, it is expressed that the injection of electrons from the charge generating layer to the electron transporting layer is insufficient, and electrons slow in movement are likely to be retained in the charge generating layer. Then, it is conceivable that the tendency corresponds to the case where  $R_{\text{opt}}/R_{\text{dark}}$  is 0.96 or more. By contrast, if the resistance between the conductive support and the gold elec-

trode decreases by light irradiation in the state that the charge generating layer is saturated with electrons (charge derived from light excitation) slow in movement, it is conceivable that the injection of electrons from the charge generating layer to the electron transporting layer is sufficiently carried out, and the retention of electrons slow in movement in the charge generating layer can be reduced.

The state of the retention of electrons slow in movement can be clarified by paying attention to the impedance at low frequencies. Although 0.1 Hz is paid attention to as a low frequency in the evaluation method according to the present invention, it is conceivable that any frequency can express the impedance of electrons slow in movement as long as the frequency is a low frequency lower than 0.1 Hz. In the present invention, the impedance of electrons slow in movement is observed using the impedance at 0.1 Hz. 0.1 Hz is a period of about 10 sec, and a state is conceivably expressed that electrons responding to the electric field in a period of 10 sec are retained in the charge generating layer through repeated use, and the positive ghost is liable to occur.

It is conceivable that if the relation of the expression (1) is satisfied, such a state of good injectability that the retention of electrons slow in movement is reduced is exhibited, and in the repeated use, the retention of electrons in the early stage and after the repeated use in the charging-light irradiation process is reduced to thereby allow the reduction of the positive ghost. As shown in Comparative Examples described later, although electrophotographic photosensitive members of National Publication of International Patent Application No. 2009-505156 and the like have a sufficient conductivity of electron transporting layers, since electrons slow in movement are liable to be retained in charge generating layers,  $R_{\text{opt}}/R_{\text{dark}}$  becomes higher than 0.95, and the positive ghost after repeated use is liable to occur in some cases.

It is also conceivable that a technology of Japanese Patent Application Laid-Open No. 2005-189764 in which the electron mobility of an undercoating layer (electron transporting layer) is made to be  $10^{-7} \text{ cm}^2/\text{V}\cdot\text{sec}$  or more has an object to improve the movement of electrons to a faster movement, and does not solve the cause of the positive ghost due to the retention of electrons slow in movement. Japanese Patent Application Laid-Open No. 2010-145506 discloses that the charge mobility of a hole transporting layer and an electron transporting layer (undercoating layer) are made to be in specific ranges, but does not solve the cause of generating the positive ghost as in Japanese Patent Application Laid-Open No. 2005-189764. Additionally, in these Patent Literatures, the measurement of the electron mobility of an electron transporting layer is carried out by using a constitution in which an electron transporting layer is formed on a charge generating layer, which constitution is reverse to the layer constitution used in an electrophotographic photosensitive member. However, such a measurement cannot be said to be able to sufficiently evaluate the movement of electrons in an electron transporting layer of an electrophotographic photosensitive member.

For example, in the case where an electron transporting layer is made by incorporating an electron transporting substance in an undercoating layer, when coating liquids for a charge generating layer and a hole transporting layer as upper layers are applied to form the charge generating layer and the hole transporting layer, the electron transporting substance elutes in some cases. It is conceivable in this case that even if the electron mobility is measured by making the electron transporting layer and the charge generating layer as reversed layers as described above, since the electron transporting substance elutes in an electrophotographic photosensitive

member, the movement of electrons of the electron transporting layer of the electrophotographic photosensitive member cannot sufficiently be evaluated. Therefore, it is believed that the determination needs to be carried out using an electron transporting layer from which a hole transporting layer has been peeled and a charge generating layer after the charge generating layer and the hole transporting layer are formed on the electron transporting layer.

The electrophotographic photosensitive member according to the present invention has a laminated body, and a hole transporting layer formed on the laminated body, and the laminated body has a conductive support, an electron transporting layer formed on the conductive support, and a charge generating layer formed on the electron transporting layer. FIG. 6 is a diagram illustrating one example of a layer constitution of the electrophotographic photosensitive member. In FIG. 6, reference numeral 21 denotes a conductive support; reference numeral 22 denotes an electron transporting layer; reference numeral 23 denotes a charge generating layer; and reference numeral 24 denotes a hole transporting layer.

As a usual electrophotographic photosensitive member, a cylindrical electrophotographic photosensitive member in which a photosensitive layer (a charge generating layer, a hole transporting layer) are formed on a cylindrical support is broadly used, but an otherwise shaped one such as a belt-shaped or sheet-shaped one may be used.

#### Electron Transporting Layer

The thickness of an electron transporting layer can be 0.1  $\mu\text{m}$  or more and 1.5  $\mu\text{m}$  or less, and is more preferably 0.2  $\mu\text{m}$  or more and 0.7  $\mu\text{m}$  or less.

If the above-mentioned laminated body satisfies the relation of the following expression (2), a larger positive ghost-reduction effect is acquired. Since a lower value of  $R_{\text{opt}}/R_{\text{dark}}$  gives a larger positive ghost-reduction effect, the value suffices if the value is higher than 0.

$$0 < R_{\text{opt}}/R_{\text{dark}} \leq 0.85 \quad \text{expression (2)}$$

The value more preferably satisfies the following expression (3).

$$0.60 \leq R_{\text{opt}}/R_{\text{dark}} \leq 0.85 \quad \text{Expression (3)}$$

In the above expressions (2) and (3),  $R_{\text{opt}}$  represents an impedance measured by forming a circular-shaped gold electrode having a thickness of 300 nm and a diameter of 10 mm on a surface of the charge generating layer of the laminated body by sputtering, applying an alternating electric field of 100 mV and 0.1 Hz between the conductive support and the gold electrode under the condition of irradiation of the surface of the charge generating layer with light having an irradiation intensity of 30  $\mu\text{J}/\text{cm}^2\text{-sec}$ , and measuring the impedance.  $R_{\text{dark}}$  represents an impedance measured by forming a circular-shaped gold electrode having a thickness of 300 nm and a diameter of 10 mm on a surface of the charge generating layer of the laminated body by sputtering, applying an alternating electric field of 100 mV and 0.1 Hz between the conductive support and the gold electrode under the condition of no light irradiation of the surface of the charge generating layer, and measuring the impedance.

Then, the constitution of an electron transporting layer will be described. An electron transporting layer can contain an electron transporting substance or a polymer of an electron transporting substance. The electron transporting layer can further contain a polymer obtained by polymerizing a composition including an electron transporting substance having polymerizable functional groups, a thermoplastic resin having polymerizable functional groups and a crosslinking agent.

#### Electron Transporting Substance

Examples of electron transporting substances include quinone compounds, imide compounds, benzimidazole compounds and cyclopentadienylidene compounds. An electron transporting substance can be an electron transporting substance having polymerizable functional groups. The polymerizable functional group includes a hydroxy group, a thiol group, an amino group, a carboxyl group and a methoxy group.

Hereinafter, specific examples of the electron transporting substance are shown. The electron transporting substance includes compounds represented by one of the following formulae (A1) to (A9).



9

-continued



(A6)



(A7)



(A8)



(A9)

In the formulae (A1) to (A9), R<sup>101</sup> to R<sup>111</sup>, R<sup>201</sup> to R<sup>210</sup>, R<sup>301</sup> to R<sup>308</sup>, R<sup>401</sup> to R<sup>408</sup>, R<sup>501</sup> to R<sup>510</sup>, R<sup>601</sup> to R<sup>606</sup>, R<sup>701</sup> to R<sup>708</sup>, R<sup>801</sup> to R<sup>810</sup> and R<sup>901</sup> to R<sup>908</sup> each independently represent a monovalent group represented by the following formula (A), a hydrogen atom, a cyano group, a nitro group, a halogen atom, an alkoxy carbonyl group, a substituted or unsubstituted alkyl group, a substituted or unsubstituted aryl group or a substituted or unsubstituted heterocyclic group. One of carbon atoms in the main chain of the alkyl group may be replaced by O, S, NH or NR<sup>1001</sup> (R<sup>1001</sup> is an alkyl group). The substituent of the substituted alkyl group includes an alkyl group, an aryl group, an alkoxy carbonyl group and a halogen atom. The substituent of the substituted aryl group and the substituent of the substituted heterocyclic group include a halogen atom, a nitro group, a cyano group, an alkyl group and an alkyl halide group. Z<sup>201</sup>, Z<sup>301</sup>, Z<sup>401</sup> and Z<sup>501</sup> each independently represent a carbon atom, a nitrogen atom or an oxygen atom. In the case where Z<sup>201</sup> is an oxygen atom, R<sup>209</sup> and R<sup>210</sup> are not present, and in the case where Z<sup>201</sup> is a nitrogen atom, R<sup>210</sup> is not present. In the case where Z<sup>301</sup> is an oxygen atom, R<sup>307</sup> and R<sup>308</sup> are not present, and in the case where Z<sup>301</sup> is a nitrogen atom, R<sup>308</sup> is not present. In the case where Z<sup>401</sup> is an oxygen atom, R<sup>407</sup> and R<sup>408</sup> are not present, and in the case where Z<sup>401</sup> is a nitrogen atom, R<sup>408</sup> is not

10

present. In the case where Z<sup>501</sup> is an oxygen atom, R<sup>509</sup> and R<sup>510</sup> are not present, and in the case where Z<sup>501</sup> is a nitrogen atom, R<sup>510</sup> is not present.

5       $\text{---} \alpha \text{---} \beta \text{---} \gamma \text{---}$ 

(A)

In the formula (A), at least one of  $\alpha$ ,  $\beta$  and  $\gamma$  is a group having a substituent, and the substituent is at least one group selected from the group consisting of a hydroxy group, a thiol group, an amino group, a carboxyl group and a methoxy group. 1 and m are each independently 0 or 1, and the sum of 1 and m is 0 to 2.

10       $\alpha$  represents an alkylene group having 1 to 6 atoms in the main chain, an alkylene group having 1 to 6 atoms in the main chain and being substituted with an alkyl group having 1 to 6 carbon atoms, an alkylene group having 1 to 6 atoms in the main chain and being substituted with a benzyl group, an alkylene group having 1 to 6 atoms in the main chain and being substituted with an alkoxy carbonyl group, or an alkylene group having 1 to 6 atoms in the main chain and being substituted with a phenyl group, and these groups may have at least one substituent selected from the group consisting of a hydroxy group, a thiol group, an amino group and a carboxyl group. One of carbon atoms in the main chain of the alkylene group may be replaced by O, S, NH or NR<sup>1002</sup> (R<sup>1002</sup> is an alkyl group).

15       $\beta$  represents a phenylene group, a phenylene group substituted with an alkyl group having 1 to 6 carbon atoms, a nitro group-substituted phenylene group, a halogen group-substituted phenylene group or an alkoxy group-substituted phenylene group, and these groups may have at least one substituent selected from the group consisting of a hydroxy group, a thiol group, an amino group and a carboxyl group.

20       $\gamma$  represents a hydrogen atom, an alkyl group having 1 to 6 atoms in the main chain, or an alkyl group having 1 to 6 atoms in the main chain and being substituted with an alkyl group having 1 to 6 carbon atoms, and these groups may have at least one substituent selected from the group consisting of a hydroxy group, a thiol group, an amino group and a carboxyl group. One of carbon atoms in the main chain of the alkyl group may be replaced by O, S, NH or NR<sup>100</sup> (R<sup>1003</sup> is an alkyl group).

25      Among electron transporting substances represented by one of the above formulae (A-1) to (A-9), electron transporting substances are more preferable which have a polymerizable functional group being a monovalent group represented by the above formula (A) for at least one of R<sup>101</sup> to R<sup>106</sup>, at least one of R<sup>201</sup> to R<sup>210</sup>, at least one of R<sup>301</sup> to R<sup>308</sup>, at least one of R<sup>401</sup> to R<sup>408</sup>, at least one of R<sup>501</sup> to R<sup>510</sup>, at least one of R<sup>601</sup> to R<sup>606</sup>, at least one of R<sup>701</sup> to R<sup>708</sup>, at least one of R<sup>801</sup> to R<sup>810</sup> and at least one of R<sup>901</sup> to R<sup>908</sup>.

30      A polymer can be formed which is obtained by polymerizing a composition containing an electron transporting substance having polymerizable functional groups, a thermoplastic resin having polymerizable functional groups, and a crosslinking agent. A method for forming an electron transporting layer involves forming a coating film of a coating liquid for the electron transporting layer containing a composition including an electron transporting substance having polymerizable functional groups, a thermoplastic resin having polymerizable functional groups and a crosslinking agent, and drying the coating film by heating to polymerize the composition to thereby form the electron transporting layer. Hereinafter, specific examples of electron transporting substances having polymerizable functional groups will be described. The heating temperature when the coating film of a coating liquid for an electron transporting layer is dried by heating can be 100 to 200°C.

## 11

In the Tables, the symbol A' is represented by the same structure as the symbol A, specific examples of the monovariant group are shown in the columns of A and A'.

Hereinafter, specific examples of the electron transporting substance having polymerizable functional groups will be

## 12

described. Specific examples of compounds represented by the above formula (A1) are shown in Table 1-1, Table 1-2, Table 1-3, Table 1-4, Table 1-5 and Table 1-6. In the Tables, the case where  $\gamma$  is “-” indicates a hydrogen atom, and the hydrogen atom for the  $\gamma$  is incorporated into the structure given in the column of  $\alpha$  or  $\beta$ .

TABLE 1-1

| Compound | A                |                  |                  |                  |                                                                                     |                  |                                                                                     |                                                                                       |                                                                                       |
|----------|------------------|------------------|------------------|------------------|-------------------------------------------------------------------------------------|------------------|-------------------------------------------------------------------------------------|---------------------------------------------------------------------------------------|---------------------------------------------------------------------------------------|
| Example  | R <sup>101</sup> | R <sup>102</sup> | R <sup>103</sup> | R <sup>104</sup> | R <sup>105</sup>                                                                    | R <sup>106</sup> | $\alpha$                                                                            | $\beta$                                                                               | $\gamma$                                                                              |
| A101     | H                | H                | H                | H                |    | A                |    | —                                                                                     | —                                                                                     |
| A102     | H                | H                | H                | H                |    | A                |    | —                                                                                     | —                                                                                     |
| A103     | H                | H                | H                | H                |   | A                | —                                                                                   |   |    |
| A104     | H                | H                | H                | H                |  | A                | —                                                                                   |  |  |
| A105     | H                | H                | H                | H                |  | A                | —                                                                                   |  |  |
| A106     | H                | H                | H                | H                |  | A                |  | —                                                                                     | —                                                                                     |
| A107     | H                | H                | H                | H                |  | A                |  | —                                                                                     | —                                                                                     |
| A108     | H                | H                | H                | H                |  | A                |  | —                                                                                     | —                                                                                     |

TABLE 1-1-continued

| Compound | A                |                  |                  |                  |                                                                                     |                  |                                                                                   |                                                                                       |                                                                                     |
|----------|------------------|------------------|------------------|------------------|-------------------------------------------------------------------------------------|------------------|-----------------------------------------------------------------------------------|---------------------------------------------------------------------------------------|-------------------------------------------------------------------------------------|
| Example  | R <sup>101</sup> | R <sup>102</sup> | R <sup>103</sup> | R <sup>104</sup> | R <sup>105</sup>                                                                    | R <sup>106</sup> | α                                                                                 | β                                                                                     | γ                                                                                   |
| A109     | H                | H                | H                | H                |    | A                | —C <sub>5</sub> H <sub>10</sub> —OH                                               | —                                                                                     | —                                                                                   |
| A110     | H                | H                | H                | H                | —C <sub>6</sub> H <sub>13</sub>                                                     | A                |  | —                                                                                     | —                                                                                   |
| A111     | H                | H                | H                | H                |    | A                | —                                                                                 |    |  |
| A112     | H                | H                | H                | H                |   | A                | —                                                                                 |   | —                                                                                   |
| A113     | H                | H                | H                | H                |  | A                | —                                                                                 |  | —                                                                                   |
| A114     | H                | H                | H                | H                |  | A                | —                                                                                 |  | —                                                                                   |
| A115     | H                | H                | H                | H                |  | A                | —                                                                                 |  | —                                                                                   |
| A116     | H                | H                | H                | H                |  | A                | —                                                                                 |  | —                                                                                   |

TABLE 1-2

| Compound Example | R <sup>101</sup>                                                                  | R <sup>102</sup> | R <sup>103</sup> | R <sup>104</sup>                                                                  | R <sup>105</sup>                                                                     | R <sup>106</sup>                                                                      |
|------------------|-----------------------------------------------------------------------------------|------------------|------------------|-----------------------------------------------------------------------------------|--------------------------------------------------------------------------------------|---------------------------------------------------------------------------------------|
| A117             | H                                                                                 | H                | H                | H                                                                                 |    | A                                                                                     |
| A118             | H                                                                                 | H                | H                | H                                                                                 |    | A                                                                                     |
| A119             |  | H                | H                |  |    | A                                                                                     |
| A120             | CN                                                                                | H                | H                | CN                                                                                |   | A                                                                                     |
| A121             | A                                                                                 | H                | H                | H                                                                                 |  |  |
| A122             | H                                                                                 | NO <sub>2</sub>  | H                | NO <sub>2</sub>                                                                   |  | A                                                                                     |
| A123             | H                                                                                 | H                | H                | H                                                                                 |  | A                                                                                     |
| A124             | H                                                                                 | H                | H                | H                                                                                 | A                                                                                    | A                                                                                     |
| A125             | H                                                                                 | H                | H                | H                                                                                 | A                                                                                    | A                                                                                     |
| A126             | H                                                                                 | H                | H                | H                                                                                 | A                                                                                    | A                                                                                     |
| A127             | H                                                                                 | H                | H                | H                                                                                 | A                                                                                    | A                                                                                     |
| A128             | H                                                                                 | H                | H                | H                                                                                 | A                                                                                    | A                                                                                     |
| A129             | H                                                                                 | H                | H                | H                                                                                 | A                                                                                    | A                                                                                     |
| A130             | H                                                                                 | H                | H                | H                                                                                 | A                                                                                    | A                                                                                     |

TABLE 1-2-continued

|          |                                                                                     |                                                                                     |          |                                                                                   |   |
|----------|-------------------------------------------------------------------------------------|-------------------------------------------------------------------------------------|----------|-----------------------------------------------------------------------------------|---|
| A131     | H                                                                                   | H                                                                                   | H        |  | A |
| A132     | H                                                                                   | H                                                                                   | H        |  | A |
| A133     | H                                                                                   | H                                                                                   | H        |  | A |
| Compound | A                                                                                   |                                                                                     |          |                                                                                   |   |
| Example  | $\alpha$                                                                            | $\beta$                                                                             | $\gamma$ |                                                                                   |   |
| A117     | —                                                                                   |   | —        |                                                                                   |   |
| A118     | —                                                                                   |  | —        | $\cdots \text{C}_2\text{H}_2\text{COOH}$                                          |   |
| A119     |  | —                                                                                   |          |                                                                                   |   |
| A120     |  | —                                                                                   |          |                                                                                   |   |
| A121     | —                                                                                   | —                                                                                   | —        | —COOH                                                                             |   |
| A122     |  | —                                                                                   |          |                                                                                   |   |
| A123     |  | —                                                                                   |          |                                                                                   |   |
| A124     |  | —                                                                                   |          |                                                                                   |   |
| A125     | —                                                                                   |  | —        | $\cdots \text{CH}_2\text{OH}$                                                     |   |

TABLE 1-2-continued

|      |                                                                                     |                                                                                   |   |
|------|-------------------------------------------------------------------------------------|-----------------------------------------------------------------------------------|---|
| A126 | —                                                                                   |  | — |
| A127 | —                                                                                   |  | — |
| A128 | —                                                                                   |  | — |
| A129 | —                                                                                   |  | — |
| A130 | —                                                                                   |  | — |
| A131 |   | —                                                                                 | — |
| A132 |  | —                                                                                 | — |
| A133 |  | —                                                                                 | — |

TABLE 1-3

| Compound Example | R <sup>101</sup> | R <sup>102</sup> | R <sup>103</sup> | R <sup>104</sup> | R <sup>105</sup>                                                                    | R <sup>106</sup> |
|------------------|------------------|------------------|------------------|------------------|-------------------------------------------------------------------------------------|------------------|
| A134             | H                | H                | H                | H                |  | A                |
| A135             | H                | H                | H                | H                | A                                                                                   | A                |
| A136             | H                | H                | H                | H                | A                                                                                   | A                |
| A137             | H                | H                | H                | H                | A                                                                                   | A                |
| A138             | H                | H                | H                | H                | A                                                                                   | A                |
| A139             | H                | H                | H                | H                |  | A                |

TABLE 1-3-continued

|          |    |                                                                                     |   |         |                                                                                     |          |
|----------|----|-------------------------------------------------------------------------------------|---|---------|-------------------------------------------------------------------------------------|----------|
| A140     | H  | H                                                                                   | H | H       |    | A        |
| A141     | H  | H                                                                                   | H | H       |    | A        |
| A142     | H  | H                                                                                   | H | H       | A                                                                                   | A        |
| A143     | CN | H                                                                                   | H | CN      |    | A        |
| A144     | H  | H                                                                                   | H | H       | $-\text{C}_2\text{H}_4-\text{O}-\text{C}_2\text{H}_5$                               | A        |
| A145     | H  | H                                                                                   | H | H       |    | A        |
| A146     | H  | H                                                                                   | H | H       | A                                                                                   | A        |
| A147     | H  | H                                                                                   | H | H       |   | A        |
| A148     | H  | H                                                                                   | H | H       |  | A        |
| A149     | H  | H                                                                                   | H | H       |  | A        |
| A150     | H  | H                                                                                   | H | H       |  | A        |
| A151     | H  | H                                                                                   | H | H       | A                                                                                   | A        |
| Compound |    |                                                                                     |   |         | A                                                                                   |          |
| Example  |    | $\alpha$                                                                            |   | $\beta$ |                                                                                     | $\gamma$ |
| A134     |    |  | — | —       | —                                                                                   | —        |
| A135     |    |  | — | —       | —                                                                                   | —        |

TABLE 1-3-continued

|      |                                                                     |   |   |
|------|---------------------------------------------------------------------|---|---|
| A136 |                                                                     | — | — |
| A137 |                                                                     | — | — |
| A138 | —                                                                   |   |   |
| A139 |                                                                     | — | — |
| A140 |                                                                     | — | — |
| A141 |                                                                     | — | — |
| A142 |                                                                     | — | — |
| A143 |                                                                     | — | — |
| A144 |                                                                     | — | — |
| A145 | —C <sub>2</sub> H <sub>4</sub> —O—C <sub>2</sub> H <sub>4</sub> —OH | — | — |
| A146 |                                                                     | — | — |
| A147 |                                                                     | — | — |
| A148 | —C <sub>2</sub> H <sub>4</sub> —O—C <sub>2</sub> H <sub>4</sub> —OH | — | — |
| A149 | —CH <sub>2</sub> CH <sub>2</sub> —                                  |   | — |

TABLE 1-3-continued

|      |   |  |      |                        |
|------|---|--|------|------------------------|
| A150 | — |  | COOH | —                      |
| A151 | — |  | —    | ---CH <sub>2</sub> —OH |

TABLE 1-4

| Compound | Example | R <sup>101</sup> | R <sup>102</sup> | R <sup>103</sup>                    | R <sup>104</sup>                    | R <sup>105</sup> | R <sup>106</sup>       |
|----------|---------|------------------|------------------|-------------------------------------|-------------------------------------|------------------|------------------------|
| A152     | A152    | H                | H                | H                                   | H                                   | A                | A'                     |
| A153     | A153    | H                | H                | H                                   | H                                   | A                | A'                     |
| A154     | A154    | H                | H                | H                                   | H                                   | A                | A'                     |
| A155     | A155    | H                | H                | H                                   | H                                   | A                | A'                     |
| A156     | A156    | H                | H                | H                                   | H                                   | A                | A'                     |
| Compound | Example | A                |                  |                                     | A'                                  |                  |                        |
|          |         | α                | β                | γ                                   | α                                   | β                | γ                      |
| A152     | A152    |                  | —                | —                                   | —                                   |                  | —                      |
| A153     | A153    | —                |                  | —                                   | ---CH <sub>2</sub> —OH              |                  | —                      |
| A154     | A154    | —                |                  | ---C <sub>H<sub>2</sub></sub> —COOH | ---C <sub>H<sub>2</sub></sub> —COOH | —                | —                      |
| A155     | A155    | —                |                  | —                                   |                                     | —                | ---CH <sub>2</sub> —OH |
| A156     | A156    |                  | —                | —                                   |                                     | —                | ---CH <sub>2</sub> —OH |

TABLE 1-5

| Compound | A                |                  |                  |                  |                  |                  |   |   |   |
|----------|------------------|------------------|------------------|------------------|------------------|------------------|---|---|---|
| Example  | R <sup>101</sup> | R <sup>102</sup> | R <sup>103</sup> | R <sup>104</sup> | R <sup>105</sup> | R <sup>106</sup> | α | β | γ |
| A157     | H                | H                | H                | H                | A                | A                |   | — | — |

TABLE 1-5-continued

| Compound | Example | $R^{101}$ | $R^{102}$ | $R^{103}$ | $R^{104}$ | $R^{105}$                                                                           | $R^{106}$ | A                                                                                    |         |          |
|----------|---------|-----------|-----------|-----------|-----------|-------------------------------------------------------------------------------------|-----------|--------------------------------------------------------------------------------------|---------|----------|
|          |         |           |           |           |           |                                                                                     |           | $\alpha$                                                                             | $\beta$ | $\gamma$ |
| A158     |         | H         | H         | H         | H         | A                                                                                   | A         |    | —       | —        |
| A159     |         | H         | H         | H         | H         | A                                                                                   | A         |    | —       | —        |
| A160     |         | H         | H         | H         | H         | $-C_6H_{12}-OH$                                                                     | A         |    | —       | —        |
| A161     |         | H         | H         | H         | H         |   | A         |   | —       | —        |
| A162     |         | H         | H         | H         | H         | A                                                                                   | A         |  | —       | —        |
| A163     |         | H         | H         | H         | H         |  | A         | $-C_2H_4-S-C_2H_4-OH$                                                                | —       | —        |
| A164     |         | H         | H         | H         | H         | A                                                                                   | A         |  | —       | —        |
| A165     |         | H         | H         | H         | H         | A                                                                                   | A         |  | —       | —        |
| A166     |         | H         | H         | H         | H         | $-C_2H_4-O-C_2H_5$                                                                  | A         |  | —       | —        |
| A167     |         | H         | H         | H         | H         | $-C_2H_4-S-C_2H_5$                                                                  | A         |  | —       | —        |

TABLE 1-5-continued

| Compound |                  |                  |                  |                  |                                                                                                                                                                                                                |                  | A                                                                                  |   |   |
|----------|------------------|------------------|------------------|------------------|----------------------------------------------------------------------------------------------------------------------------------------------------------------------------------------------------------------|------------------|------------------------------------------------------------------------------------|---|---|
| Example  | R <sup>101</sup> | R <sup>102</sup> | R <sup>103</sup> | R <sup>104</sup> | R <sup>105</sup>                                                                                                                                                                                               | R <sup>106</sup> | α                                                                                  | β | γ |
| A168     | H                | H                | H                | H                | $\text{---C}_2\text{H}_4\text{---N}(\text{H})\text{---C}_4\text{H}_9$                                                                                                                                          | A                |  | — | — |
| A169     | H                | H                | H                | H                | $\text{---CH}(\text{CH}_3)\text{---H}_2\text{C---C}(\text{H}_2)\text{---C}(\text{H}_2)\text{---N}(\text{H}_2\text{C---CH}_3)\text{---H}_2\text{C---CH}_3$                                                      | A                |  | — | — |
| A170     | H                | H                | H                | H                | $\text{---CH}(\text{CH}_3)\text{---C}(\text{O})\text{---O---C}(\text{H}_2\text{C---CH}_3)\text{---CH}_3\text{---CH}(\text{CH}_3)\text{---C}(\text{O})\text{---O---C}(\text{H}_2\text{C---CH}_3)\text{---CH}_3$ | A                |  | — | — |

TABLE 1-6

| Compound |                  |                  |                  |                  |                  |                  | A                                                                                   |   | A' |                                                                                       |   |   |
|----------|------------------|------------------|------------------|------------------|------------------|------------------|-------------------------------------------------------------------------------------|---|----|---------------------------------------------------------------------------------------|---|---|
| Example  | R <sup>101</sup> | R <sup>102</sup> | R <sup>103</sup> | R <sup>104</sup> | R <sup>105</sup> | R <sup>106</sup> | α                                                                                   | β | γ  | α                                                                                     | β | γ |
| A171     | H                | H                | H                | H                | A                | A'               |  | — | —  |  | — | — |
| A172     | H                | H                | H                | H                | A                | A'               | $\text{---C}_2\text{H}_4\text{---O---C}_2\text{H}_4\text{---OH}$                    | — | —  |  | — | — |
| A173     | H                | H                | H                | H                | A                | A'               | $\text{---C}_6\text{H}_{12}\text{---OH}$                                            | — | —  |  | — | — |
| A174     | H                | H                | H                | H                | A                | A'               | $\text{---C}_3\text{H}_6\text{---N}(\text{H})\text{---C}_2\text{H}_4\text{---OH}$   | — | —  |  | — | — |
| A175     | H                | H                | H                | H                | A                | A'               | $\text{---C}_2\text{H}_4\text{---O---C}_2\text{H}_4\text{---OH}$                    | — | —  |  | — | — |

TABLE 1-6-continued

| Compound<br>Example | R <sup>101</sup> | R <sup>102</sup> | R <sup>103</sup> | R <sup>104</sup> | R <sup>105</sup> | R <sup>106</sup> | A                                                                   |   |   | A' |   |   |
|---------------------|------------------|------------------|------------------|------------------|------------------|------------------|---------------------------------------------------------------------|---|---|----|---|---|
|                     |                  |                  |                  |                  |                  |                  | α                                                                   | β | γ | α  | β | γ |
| A176                | H                | H                | H                | H                | A                | A'               | —C <sub>2</sub> H <sub>4</sub> —O—C <sub>2</sub> H <sub>4</sub> —OH | — | — |    | — | — |
| A177                | H                | H                | H                | H                | A                | A'               | —C <sub>2</sub> H <sub>4</sub> —S—C <sub>2</sub> H <sub>4</sub> —OH | — | — |    | — | — |
| A178                | H                | H                | H                | H                | A                | A'               |                                                                     | — | — |    | — | — |
| A179                | H                | H                | H                | H                | A                | A'               |                                                                     | — | — |    | — | — |
| A180                | H                | H                | H                | H                | A                | A'               |                                                                     | — | — |    | — | — |
| A181                | H                | H                | H                | H                | A                | A'               | —C <sub>2</sub> H <sub>4</sub> —S—C <sub>2</sub> H <sub>4</sub> —OH | — | — |    | — | — |

Specific examples of compounds represented by the above formula (A2) are shown in Table 2-1, Table 2-2 and Table 2-3. In the Tables, the case where  $\gamma$  is “-” indicates a hydrogen atom, and the hydrogen atom for the  $\gamma$  is incorporated into the structure given in the column of  $\alpha$  or  $\beta$ .  
45

TABLE 2-1

| Compound<br>Example | R <sup>201</sup> | R <sup>202</sup> | R <sup>203</sup> | R <sup>204</sup> | R <sup>205</sup> | R <sup>206</sup> | R <sup>207</sup> | R <sup>208</sup> | R <sup>209</sup> | R <sup>210</sup> | Z <sup>201</sup> |
|---------------------|------------------|------------------|------------------|------------------|------------------|------------------|------------------|------------------|------------------|------------------|------------------|
| A201                | H                | H                | A                | H                | H                | H                | H                | H                | —                | —                | O                |
| A202                | H                | H                | A                | H                | H                | H                | H                | H                | —                | —                | O                |
| A204                | H                | H                | A                | H                | H                | H                | H                | H                | —                | —                | O                |
| A205                | H                | H                | A                | H                | H                | H                | H                | H                | —                | —                | O                |
| A206                | H                | H                | A                | H                | H                | H                | H                | H                | —                | —                | O                |
| A207                | H                | H                | H                | H                | H                | H                | H                | H                | A                | —                | N                |
| A208                | H                | H                | H                | H                | H                | H                | H                | H                | A                | —                | N                |
| A209                | H                | H                | H                | H                | H                | H                | H                | H                | A                | —                | N                |
| A210                | H                | H                | H                | H                | H                | H                | H                | H                | A                | —                | N                |
| A211                | CH <sub>3</sub>  | H                | H                | H                | H                | H                | H                | CH <sub>3</sub>  | A                | —                | N                |
| A212                | H                | Cl               | H                | H                | H                | H                | Cl               | H                | A                | —                | N                |
| A213                | H                | H                |                  | H                | H                |                  | H                | H                | A                | —                | N                |

TABLE 2-1-continued

|          |   |   |          |                 |                 |   |   |          |   |   |   |
|----------|---|---|----------|-----------------|-----------------|---|---|----------|---|---|---|
| A214     | H | H |          | H               | H               |   | H | H        | A | — | N |
| A215     | H | H | H        | NO <sub>2</sub> | NO <sub>2</sub> | H | H | H        | A | — | N |
| A216     | H | H | A        | H               | H               | A | H | H        | — | — | O |
| A217     | H | H | A        | H               | H               | A | H | H        | — | — | O |
| Compound |   |   |          | A               |                 |   |   |          |   |   |   |
| Example  |   |   | $\alpha$ |                 | $\beta$         |   |   | $\gamma$ |   |   |   |
| A201     | — |   |          |                 |                 |   | — |          |   |   |   |
| A202     | — |   |          |                 |                 |   | — |          |   |   |   |
| A204     | — |   |          |                 |                 |   | — |          |   |   |   |
| A205     | — |   |          |                 |                 |   | — |          |   |   |   |
| A206     | — |   |          |                 |                 |   | — |          |   |   |   |
| A207     | — |   |          |                 |                 |   |   |          |   |   |   |
| A208     | — |   |          |                 |                 |   | — |          |   |   |   |
| A209     | — |   |          |                 |                 |   | — |          |   |   |   |
| A210     |   |   |          |                 |                 | — |   |          | — |   |   |
| A211     | — |   |          |                 |                 |   |   |          |   |   |   |

TABLE 2-1-continued

|      |   |  |   |
|------|---|--|---|
| A212 | — |  |   |
| A213 | — |  |   |
| A214 | — |  |   |
| A215 | — |  |   |
| A216 | — |  |   |
| A217 | — |  | — |

TABLE 2-2

| Compound Example | R <sup>201</sup> | R <sup>202</sup> | R <sup>203</sup> | R <sup>204</sup> | R <sup>205</sup> | R <sup>206</sup> | R <sup>207</sup> | R <sup>208</sup> | R <sup>209</sup> | R <sup>210</sup> |
|------------------|------------------|------------------|------------------|------------------|------------------|------------------|------------------|------------------|------------------|------------------|
| A218             | H                | H                | A                | H                | H                | A                | H                | H                | —                | —                |
| A219             | H                | H                | A                | H                | H                | A                | H                | H                | —                | —                |
| A220             | H                | H                | A                | H                | H                | A                | H                | H                | —                | —                |
| A221             | H                | H                | A                | H                | H                | A                | H                | H                | —                | —                |
| A222             | H                | H                | A                | H                | H                | A                | H                | H                | —                | —                |
| A223             | H                | H                | A                | H                | H                | A                | H                | H                | —                | —                |
| A224             | H                | A                | H                | H                | H                | H                | A                | H                | —                | —                |
| A225             | H                | H                | A                | H                | H                | A                | H                | H                | CN               | CN               |
| A226             | H                | H                | A                | H                | H                | A                | H                | H                | CN               | CN               |
| A227             | H                | H                | A                | H                | H                | A                | H                | H                | CN               | CN               |
| A228             | H                | H                | A                | H                | H                | A                | H                | H                | CN               | CN               |
| A229             | H                | H                | A                | H                | H                | A                | H                | H                | CN               |                  |
| A230             | H                | H                | A                | H                | H                | A                | H                | H                |                  |                  |
| A231             | H                | H                | H                | H                | H                | H                | H                | H                | A                | A                |
| A232             | H                | NO <sub>2</sub>  | H                | H                | H                | H                | NO <sub>2</sub>  | H                | A                | —                |
| A233             | H                | H                | H                | H                | H                | A                | H                | H                | —                | —                |

TABLE 2-2-continued

| Compound |           | A        |         |                        |
|----------|-----------|----------|---------|------------------------|
| Example  | $Z^{201}$ | $\alpha$ | $\beta$ | $\gamma$               |
| A218     | O         | —        |         | —                      |
| A219     | O         | —        |         | —                      |
| A220     | O         |          | —       | —                      |
| A221     | O         |          | —       | —                      |
| A222     | O         | —        | —       | COOH                   |
| A223     | O         | —        | —       | NH <sub>2</sub>        |
| A224     | O         | —        |         | ---CH <sub>2</sub> —OH |
| A225     | C         | —        |         | ---CH <sub>2</sub> —OH |
| A226     | C         | —        |         | —                      |
| A227     | C         | —        |         | —                      |
| A228     | C         | —        |         | —                      |
| A229     | C         | —        |         | ---CH <sub>2</sub> —OH |
| A230     | C         | —        |         | ---CH <sub>2</sub> —OH |
| A231     | C         | —        | —       | COOH                   |
| A232     | N         | —        |         |                        |
| A233     | O         | —        |         | ---CH <sub>2</sub> —OH |

TABLE 2-3

| Compound Example | R <sup>201</sup> | R <sup>202</sup> | R <sup>203</sup> | R <sup>204</sup> | R <sup>205</sup> | R <sup>206</sup> | R <sup>207</sup> | R <sup>208</sup> | R <sup>209</sup> | R <sup>210</sup> | Z <sup>201</sup> |
|------------------|------------------|------------------|------------------|------------------|------------------|------------------|------------------|------------------|------------------|------------------|------------------|
| A234             | H                | A                | H                | H                | H                | H                | A'               | H                | —                | —                | O                |
| A235             | H                | A                | H                | H                | H                | H                | A'               | H                | —                | —                | O                |
| A236             | H                | A'               | H                | H                | H                | H                | A'               | H                | —                | —                | O                |
| Compound         | A                |                  |                  |                  |                  | A'               |                  |                  |                  |                  |                  |
| Example          | α                | β                | γ                |                  | α                | β                | γ                |                  |                  |                  |                  |
| A234             |                  | —                | —                |                  | —                |                  |                  | —                | —                | —                | O                |
| A235             | —                |                  |                  | —                |                  |                  | —                | —                | —                | —                | —                |
| A236             | —                |                  |                  | —                |                  |                  | —                | —                | —                | —                | —                |

Specific examples of compounds represented by the above formula (A3) are shown in Table 3-1, Table 3-2 and Table 3-3. 30  
In the Tables, the case where γ is “-” indicates a hydrogen atom, and the hydrogen atom for the γ is incorporated into the structure given in the column of α or β.

TABLE 3-1

| Compound Example | R <sup>301</sup> | R <sup>302</sup> | R <sup>303</sup> | R <sup>304</sup> | R <sup>305</sup> | R <sup>306</sup> | R <sup>307</sup> | R <sup>308</sup> |
|------------------|------------------|------------------|------------------|------------------|------------------|------------------|------------------|------------------|
| A301             | H                | A                | H                | H                | H                | H                | —                | —                |
| A302             | H                | A                | H                | H                | H                | H                | —                | —                |
| A303             | H                | A                | H                | H                | H                | H                | —                | —                |
| A304             | H                | A                | H                | H                | H                | H                | —                | —                |
| A305             | H                | A                | H                | H                | H                | H                | —                | —                |
| A306             | H                | H                | H                | H                | H                | H                | A                | —                |
| A307             | H                | H                | H                | H                | H                | H                | A                | —                |
| A308             | H                | H                | H                | H                | H                | H                | A                | —                |
| A309             | CH <sub>3</sub>  | H                | H                | H                | H                | CH <sub>3</sub>  | A                | —                |
| A310             | H                | H                | Cl               | Cl               | H                | H                | A                | —                |
| Compound         | A                |                  |                  |                  |                  |                  |                  |                  |
| Example          | Z <sup>301</sup> | α                | β                | γ                |                  |                  |                  |                  |
| A301             | O                | —                |                  | —                |                  | —                | —                | —                |

TABLE 3-1-continued

|      |   |                                                                                     |                                                                                     |                                           |
|------|---|-------------------------------------------------------------------------------------|-------------------------------------------------------------------------------------|-------------------------------------------|
| A302 | O | —                                                                                   |    | ---CH <sub>2</sub> —OH                    |
| A303 | O | —                                                                                   |    | —                                         |
| A304 | O | —                                                                                   |    | —                                         |
| A305 | O | —                                                                                   |    | —                                         |
| A306 | N | —                                                                                   |    | ---CH <sub>2</sub> ---CH <sub>2</sub> —OH |
| A307 | N | —                                                                                   |   | —                                         |
| A308 | N |  | —                                                                                   | —                                         |
| A309 | N | —                                                                                   |  | ---CH <sub>2</sub> ---CH <sub>2</sub> —OH |
| A310 | N | —                                                                                   |  | ---CH <sub>2</sub> ---CH <sub>2</sub> —OH |
| A311 | N | —                                                                                   |  | ---CH <sub>2</sub> ---CH <sub>2</sub> —OH |
| A312 | N | —                                                                                   |  | ---CH <sub>2</sub> ---CH <sub>2</sub> —OH |
| A313 | N | —                                                                                   |  | ---CH <sub>2</sub> ---CH <sub>2</sub> —OH |

TABLE 3-1-continued

|      |   |   |  |                        |
|------|---|---|--|------------------------|
| A314 | O | — |  | ---CH <sub>2</sub> —OH |
| A315 | O | — |  | —                      |

TABLE 3-2

| Com-<br>ound<br>Exam- | ple | A                |                  |                  |                  |                  |                  |                  |                  |                  |   |                      |                 |
|-----------------------|-----|------------------|------------------|------------------|------------------|------------------|------------------|------------------|------------------|------------------|---|----------------------|-----------------|
|                       |     | R <sup>301</sup> | R <sup>302</sup> | R <sup>303</sup> | R <sup>304</sup> | R <sup>305</sup> | R <sup>306</sup> | R <sup>307</sup> | R <sup>308</sup> | Z <sup>301</sup> | α | β                    | γ               |
| A316                  | H   | A                | H                | H                | A                | H                | —                | —                | O                | —                |   | —                    | —               |
| A317                  | H   | A                | H                | H                | A                | H                | —                | —                | O                | —                |   | —                    | —               |
| A318                  | H   | A                | H                | H                | A                | H                | —                | —                | O                |                  | — | —                    | —               |
| A319                  | H   | A                | H                | H                | A                | H                | —                | —                | O                |                  | — | —                    | —               |
| A320                  | H   | A                | H                | H                | A                | H                | —                | —                | O                | —                | — | —                    | COOH            |
| A321                  | H   | A                | H                | H                | A                | H                | —                | —                | O                | —                | — | —                    | NH <sub>2</sub> |
| A322                  | H   | H                | A                | A                | H                | H                | —                | —                | O                | —                |   | —CH <sub>2</sub> —OH | —               |
| A323                  | H   | A                | H                | H                | A                | H                | CN               | CN               | C                | —                |   | —CH <sub>2</sub> —OH | —               |
| A324                  | H   | A                | H                | H                | A                | H                | CN               | CN               | C                | —                |   | COOH                 | —               |
| A325                  | H   | A                | H                | H                | A                | H                | CN               | CN               | C                | —                |   | —                    | —               |
| A326                  | H   | A                | H                | H                | A                | H                | CN               | CN               | C                | —                |   | —                    | —               |
| A327                  | H   | A                | H                | H                | A                | H                | CN               |                  | C                | —                |   | —CH <sub>2</sub> —OH | —               |
| A328                  | H   | A                | H                | H                | A                | H                |                  |                  | C                | —                |   | —CH <sub>2</sub> —OH | —               |
| A329                  | H   | H                | H                | H                | H                | H                | A                | A                | C                | —                | — | —                    | COOH            |
| A330                  | H   | H                | H                | H                | H                | H                | A                | —                | N                | —                |   |                      | —               |

TABLE 3-3

| Compound Exam- | ple | R <sup>301</sup> | R <sup>302</sup> | R <sup>303</sup> | R <sup>304</sup> | R <sup>305</sup> | R <sup>306</sup> | R <sup>307</sup> | R <sup>308</sup> | Z <sup>301</sup> | A                                                                                 |                                                                                   |                                                                                    | A'                                                                                  |                                                                                     |                                                                                     |
|----------------|-----|------------------|------------------|------------------|------------------|------------------|------------------|------------------|------------------|------------------|-----------------------------------------------------------------------------------|-----------------------------------------------------------------------------------|------------------------------------------------------------------------------------|-------------------------------------------------------------------------------------|-------------------------------------------------------------------------------------|-------------------------------------------------------------------------------------|
|                |     |                  |                  |                  |                  |                  |                  |                  |                  |                  | α                                                                                 | β                                                                                 | γ                                                                                  | α                                                                                   | β                                                                                   | γ                                                                                   |
| A331           | H   | A                | H                | H                | A'               | H                | H                | H                | H                | O                |  | —                                                                                 | —                                                                                  | —                                                                                   |  |  |
| A332           | H   | A'               | H                | H                | A                | H                | H                | H                | H                | O                | —                                                                                 |  |  |  | —                                                                                   | —                                                                                   |
| A333           | H   | A                | H                | H                | A'               | H                | H                | H                | H                | O                | —                                                                                 |  |  |  | —                                                                                   | —                                                                                   |

Specific examples of compounds represented by the above formula (A4) are shown in Table 4-1 and Table 4-2. In the Tables, the case where  $\gamma$  is “-” indicates a hydrogen atom, and the hydrogen atom for the  $\gamma$  is incorporated into the structure given in the column of  $\alpha$  or  $\beta$ .

TABLE 4-1

| Compound Exam- | ple             | A                |                  |                  |                  |                  |                  |                  |                  |                                                                                      |                                                                                       |                                                                                       |                                                                                       |  |
|----------------|-----------------|------------------|------------------|------------------|------------------|------------------|------------------|------------------|------------------|--------------------------------------------------------------------------------------|---------------------------------------------------------------------------------------|---------------------------------------------------------------------------------------|---------------------------------------------------------------------------------------|--|
|                |                 | R <sup>401</sup> | R <sup>402</sup> | R <sup>403</sup> | R <sup>404</sup> | R <sup>405</sup> | R <sup>406</sup> | R <sup>407</sup> | R <sup>408</sup> | Z <sup>401</sup>                                                                     | α                                                                                     | β                                                                                     | γ                                                                                     |  |
| A401           | H               | H                | A                | H                | H                | H                | CN               | CN               | C                | —                                                                                    |  |  |                                                                                       |  |
| A402           | H               | H                | A                | H                | H                | H                | CN               | CN               | C                | —                                                                                    |  |  |                                                                                       |  |
| A403           | H               | H                | A                | H                | H                | H                | CN               | CN               | C                | —                                                                                    |  |  |                                                                                       |  |
| A404           | H               | H                | A                | H                | H                | H                | CN               | CN               | C                | —                                                                                    |  |  |                                                                                       |  |
| A405           | H               | H                | A                | H                | H                | H                | CN               | CN               | C                | —                                                                                    |  |  |                                                                                       |  |
| A406           | H               | H                | H                | H                | H                | H                | A                | —                | N                | —                                                                                    |  |  |                                                                                       |  |
| A407           | H               | H                | H                | H                | H                | H                | A                | —                | N                | —                                                                                    |  |  |                                                                                       |  |
| A408           | H               | H                | H                | H                | H                | H                | A                | —                | N                | —                                                                                    |  |  |                                                                                       |  |
| A409           | H               | H                | H                | H                | H                | H                | A                | —                | N                |  | —                                                                                     | —                                                                                     |                                                                                       |  |
| A410           | CH <sub>3</sub> | H                | H                | H                | H                | H                | CH <sub>3</sub>  | A                | —                | N                                                                                    | —                                                                                     |  |  |  |
| A411           | H               | Cl               | H                | H                | H                | Cl               | H                | A                | —                | N                                                                                    | —                                                                                     |  |  |  |

TABLE 4-1-continued

| Compound Exam- | ple | R <sup>401</sup> | R <sup>402</sup> | R <sup>403</sup>                                                                  | R <sup>404</sup>                                                                  | R <sup>405</sup> | R <sup>406</sup> | R <sup>407</sup> | R <sup>408</sup> | Z <sup>401</sup> | A |                                                                                     |                                                                                     |                                                                                     |
|----------------|-----|------------------|------------------|-----------------------------------------------------------------------------------|-----------------------------------------------------------------------------------|------------------|------------------|------------------|------------------|------------------|---|-------------------------------------------------------------------------------------|-------------------------------------------------------------------------------------|-------------------------------------------------------------------------------------|
|                |     |                  |                  |                                                                                   |                                                                                   |                  |                  |                  |                  |                  | α | β                                                                                   | γ                                                                                   |                                                                                     |
| A412           | H   | H                |                  |  |  | H                | H                | A                | —                | N                | — |  |  |                                                                                     |
| A413           | H   | H                |                  |  |  | H                | H                | A                | —                | N                | — |  |  |                                                                                     |
| A414           | H   | H                |                  | H                                                                                 |                                                                                   | H                | H                | A                | —                | N                | — |  |  |                                                                                     |
| A415           | H   | H                |                  | A                                                                                 |                                                                                   | A                | H                | H                | CN               | CN               | C | —                                                                                   |  |  |

TABLE 4-2

| Compound Exam- | ple | R <sup>401</sup> | R <sup>402</sup> | R <sup>403</sup> | R <sup>404</sup> | R <sup>405</sup> | R <sup>406</sup> | R <sup>407</sup> | R <sup>408</sup>                                                                    | Z <sup>401</sup> | A                                                                                     |                                                                                       |                                                                                       |
|----------------|-----|------------------|------------------|------------------|------------------|------------------|------------------|------------------|-------------------------------------------------------------------------------------|------------------|---------------------------------------------------------------------------------------|---------------------------------------------------------------------------------------|---------------------------------------------------------------------------------------|
|                |     |                  |                  |                  |                  |                  |                  |                  |                                                                                     |                  | α                                                                                     | β                                                                                     | γ                                                                                     |
| A416           | H   | H                |                  | A                | A                | H                | H                | CN               | CN                                                                                  | C                | —                                                                                     |  |  |
| A417           | H   | H                |                  | A                | A                | H                | H                | CN               | CN                                                                                  | C                | —                                                                                     |  |  |
| A418           | H   | H                |                  | A                | A                | H                | H                | CN               | CN                                                                                  | C                | —                                                                                     |  |  |
| A419           | H   | H                |                  | A                | A                | H                | H                | CN               | CN                                                                                  | C                |  | —                                                                                     | —                                                                                     |
| A420           | H   | H                |                  | A                | A                | H                | H                | CN               | CN                                                                                  | C                |  | —                                                                                     | —                                                                                     |
| A421           | H   | H                |                  | A                | A                | H                | H                | CN               | CN                                                                                  | C                | —                                                                                     | —                                                                                     |  |
| A422           | H   | H                |                  | A                | A                | H                | H                | CN               | CN                                                                                  | C                | —                                                                                     | —                                                                                     |  |
| A423           | H   | A                |                  | H                | H                | A                | H                | CN               | CN                                                                                  | C                | —                                                                                     |  |  |
| A423           | H   | H                |                  | A                | A                | H                | H                | —                | —                                                                                   | O                | —                                                                                     |  |  |
| A424           | H   | H                |                  | A                | A                | H                | H                | —                | —                                                                                   | O                | —                                                                                     |  |  |
| A425           | H   | H                |                  | A                | A                | H                | H                | —                | —                                                                                   | O                | —                                                                                     |  |  |
| A426           | H   | H                |                  | A                | A                | H                | H                | —                | —                                                                                   | O                | —                                                                                     |  |  |
| A427           | H   | H                |                  | A                | A                | H                | H                | CN               |  | C                | —                                                                                     |  |  |

TABLE 4-2-continued

| Compound Example | ple | A                |                                                                                   |                  |                  |                  |                                                                                   |                                                                                   |                  |                  |                                                                                     |                                                                                     |                      |
|------------------|-----|------------------|-----------------------------------------------------------------------------------|------------------|------------------|------------------|-----------------------------------------------------------------------------------|-----------------------------------------------------------------------------------|------------------|------------------|-------------------------------------------------------------------------------------|-------------------------------------------------------------------------------------|----------------------|
|                  |     | R <sup>401</sup> | R <sup>402</sup>                                                                  | R <sup>403</sup> | R <sup>404</sup> | R <sup>405</sup> | R <sup>406</sup>                                                                  | R <sup>407</sup>                                                                  | R <sup>408</sup> | Z <sup>401</sup> | α                                                                                   | β                                                                                   | γ                    |
| A428             | H   | H                | A                                                                                 | A                | H                | H                |  |  | C                | —                |  |  | —CH <sub>2</sub> -OH |
| A429             | H   | H                | H                                                                                 | H                | H                | H                | A                                                                                 | A                                                                                 | C                | —                | —                                                                                   | —                                                                                   | COOH                 |
| A430             | H   | H                | H                                                                                 | A                | H                | H                | CN                                                                                | CN                                                                                | C                | —                |  |  | —CH <sub>2</sub>     |
| A431             | H   | H                |  | A                | H                | H                |  | —                                                                                 | N                | —                |  |  | —CH <sub>2</sub>     |

Specific examples of compounds represented by the above formula (A5) are shown in Table 5-1 and Table 5-2. In the Tables, the case where  $\gamma$  is “-” indicates a hydrogen atom, and the hydrogen atom for the  $\gamma$  is incorporated into the structure given in the column of  $\alpha$  or  $\beta$ .

TABLE 5-1

| Compound Example | ple             | A                |                  |                  |                  |                  |                  |                  |                  |                  |                  |                                                                                       |                                                                                       |                                                                                       |                                                                                       |                  |
|------------------|-----------------|------------------|------------------|------------------|------------------|------------------|------------------|------------------|------------------|------------------|------------------|---------------------------------------------------------------------------------------|---------------------------------------------------------------------------------------|---------------------------------------------------------------------------------------|---------------------------------------------------------------------------------------|------------------|
|                  |                 | R <sup>501</sup> | R <sup>502</sup> | R <sup>503</sup> | R <sup>504</sup> | R <sup>505</sup> | R <sup>506</sup> | R <sup>507</sup> | R <sup>508</sup> | R <sup>509</sup> | R <sup>510</sup> | Z <sup>501</sup>                                                                      | α                                                                                     | β                                                                                     | γ                                                                                     |                  |
| A501             | H               | A                | H                | H                | H                | H                | H                | H                | CN               | CN               | C                | —                                                                                     |  |  | —CH <sub>2</sub> -OH                                                                  |                  |
| A502             | H               | A                | H                | H                | H                | H                | H                | H                | CN               | CN               | C                | —                                                                                     |  |  | —CH <sub>2</sub> -OH                                                                  |                  |
| A503             | H               | A                | H                | H                | H                | H                | H                | H                | CN               | CN               | C                | —                                                                                     |  | COOH                                                                                  | —                                                                                     |                  |
| A504             | H               | A                | H                | H                | H                | H                | H                | H                | CN               | CN               | C                | —                                                                                     |  | NH <sub>2</sub>                                                                       | —                                                                                     |                  |
| A505             | H               | A                | H                | H                | H                | H                | H                | H                | CN               | CN               | C                | —                                                                                     |  | SH                                                                                    | —                                                                                     |                  |
| A506             | H               | NO <sub>2</sub>  | H                | H                | NO <sub>2</sub>  | H                | NO <sub>2</sub>  | H                | A                | —                | N                | —                                                                                     |  |  | —CH <sub>2</sub>                                                                      |                  |
| A507             | H               | H                | H                | H                | H                | H                | H                | H                | A                | —                | N                | —                                                                                     |  | COOH                                                                                  | —                                                                                     |                  |
| A508             | H               | H                | H                | H                | H                | H                | H                | H                | A                | —                | N                | —                                                                                     |  | SH                                                                                    | —                                                                                     |                  |
| A509             | H               | H                | H                | H                | H                | H                | H                | H                | A                | —                | N                |  |  | —                                                                                     |                                                                                       |                  |
| A510             | CH <sub>3</sub> | H                | H                | H                | H                | H                | H                | H                | CH <sub>3</sub>  | A                | —                | N                                                                                     | —                                                                                     |  |  | —CH <sub>2</sub> |

TABLE 5-1-continued

| Compound<br>Ex-<br>am- | ple | A                                                                                 |                  |                  |                  |                  |                                                                                   |                  |                  |                  |                  |                  |                                                                                     |                                                                                     |
|------------------------|-----|-----------------------------------------------------------------------------------|------------------|------------------|------------------|------------------|-----------------------------------------------------------------------------------|------------------|------------------|------------------|------------------|------------------|-------------------------------------------------------------------------------------|-------------------------------------------------------------------------------------|
|                        |     | R <sup>501</sup>                                                                  | R <sup>502</sup> | R <sup>503</sup> | R <sup>504</sup> | R <sup>505</sup> | R <sup>506</sup>                                                                  | R <sup>507</sup> | R <sup>508</sup> | R <sup>509</sup> | R <sup>510</sup> | Z <sup>501</sup> | α                                                                                   | β                                                                                   |
| A511                   | H   | H                                                                                 | Cl               | H                | H                | Cl               | H                                                                                 | H                | A                | —                | N                | —                |  |  |
| A512                   | H   |  | H                | H                | H                | H                |  | H                | A                | —                | N                | —                |  |  |
| A513                   | H   |  | H                | H                | H                | H                |  | H                | A                | —                | N                | —                |  |  |
| A514                   | H   | NO <sub>2</sub>                                                                   | H                | H                | NO <sub>2</sub>  | H                | NO <sub>2</sub>                                                                   | H                | A                | —                | N                | —                |  |  |
| A515                   | H   | A                                                                                 | H                | H                | H                | H                | A                                                                                 | H                | CN               | CN               | C                | —                |  |  |
| A516                   | H   | A                                                                                 | H                | H                | H                | H                | A                                                                                 | H                | CN               | CN               | C                | —                |  | —                                                                                   |

TABLE 5-2

| Compound<br>Ex-<br>am- | ple | A                |                  |                  |                  |                  |                  |                  |                  |                  |                  |                                                                                       |                                                                                       |                                                                                       |
|------------------------|-----|------------------|------------------|------------------|------------------|------------------|------------------|------------------|------------------|------------------|------------------|---------------------------------------------------------------------------------------|---------------------------------------------------------------------------------------|---------------------------------------------------------------------------------------|
|                        |     | R <sup>501</sup> | R <sup>502</sup> | R <sup>503</sup> | R <sup>504</sup> | R <sup>505</sup> | R <sup>506</sup> | R <sup>507</sup> | R <sup>508</sup> | R <sup>509</sup> | R <sup>510</sup> | Z <sup>501</sup>                                                                      | α                                                                                     | β                                                                                     |
| A517                   | H   | A                | H                | H                | H                | H                | A                | H                | CN               | CN               | C                | —                                                                                     |  | —                                                                                     |
| A518                   | H   | A                | H                | H                | H                | H                | A                | H                | CN               | CN               | C                | —                                                                                     |  | —                                                                                     |
| A519                   | H   | A                | H                | H                | H                | H                | A                | H                | CN               | CN               | C                |  | —                                                                                     | —                                                                                     |
| A520                   | H   | A                | H                | H                | H                | H                | A                | H                | CN               | CN               | C                |  | —                                                                                     | —                                                                                     |
| A521                   | H   | A                | H                | H                | H                | H                | A                | H                | CN               | CN               | C                | —                                                                                     | —                                                                                     | COOH                                                                                  |
| A522                   | H   | A                | H                | H                | H                | H                | A                | H                | CN               | CN               | C                | —                                                                                     | —                                                                                     | NH <sub>2</sub>                                                                       |
| A523                   | H   | H                | A                | H                | H                | A                | H                | H                | CN               | CN               | C                | —                                                                                     |  |  |
| A524                   | H   | A                | H                | H                | H                | H                | A                | H                | —                | —                | O                | —                                                                                     |  |  |
| A525                   | H   | A                | H                | H                | H                | H                | A                | H                | —                | —                | O                | —                                                                                     |  | —                                                                                     |
| A526                   | H   | A                | H                | H                | H                | H                | A                | H                | —                | —                | O                | —                                                                                     |  | —                                                                                     |

TABLE 5-2-continued

| Compound<br>Ex-<br>am- | ple | A                |                  |                  |                  |                  |                  |                  |                  |                  |                  |                  |   |                       |
|------------------------|-----|------------------|------------------|------------------|------------------|------------------|------------------|------------------|------------------|------------------|------------------|------------------|---|-----------------------|
|                        |     | R <sup>501</sup> | R <sup>502</sup> | R <sup>503</sup> | R <sup>504</sup> | R <sup>505</sup> | R <sup>506</sup> | R <sup>507</sup> | R <sup>508</sup> | R <sup>509</sup> | R <sup>510</sup> | Z <sup>501</sup> | α | β                     |
| A527                   | H   | A                | H                | H                | H                | H                | A                | H                | —                | —                | O                | —                |   | —                     |
| A528                   | H   | A                | H                | H                | H                | H                | A                | H                | CN               |                  | C                | —                |   | --CH <sub>2</sub> —OH |
| A529                   | H   | A                | H                | H                | H                | H                | A                | H                |                  |                  | C                | —                |   | --CH <sub>2</sub> —OH |
| A530                   | H   | H                | H                | H                | H                | H                | H                | H                | A                | A                | C                | —                | — | COOH                  |
| A531                   | H   | A                | H                | H                | H                | H                | A                | H                | CN               | CN               | C                | —                |   | --CH <sub>2</sub> —OH |
| A532                   | H   | A                | H                | H                | H                | H                | —                | —                |                  | —                | N                | —                |   | --CH <sub>2</sub> —OH |

Specific examples of compounds represented by the above formula (A6) are shown in Table 6. In the Table, the case where γ is “-” indicates a hydrogen atom, and the hydrogen atom for the γ is incorporated into the structure given in the column of α or β.

TABLE 6

| Compound | Example | A                |                  |                  |                  |                  |                  |   |   |                       |   |   |   |
|----------|---------|------------------|------------------|------------------|------------------|------------------|------------------|---|---|-----------------------|---|---|---|
|          |         | R <sup>601</sup> | R <sup>602</sup> | R <sup>603</sup> | R <sup>604</sup> | R <sup>605</sup> | R <sup>606</sup> | α | β | γ                     | — | — | — |
| A601     | A       | H                | H                | H                | H                | H                | H                | — |   | --CH <sub>2</sub> —OH | — | — | — |
| A602     | A       | H                | H                | H                | H                | H                | H                | — |   | --CH <sub>2</sub> —OH | — | — | — |
| A603     | A       | H                | H                | H                | H                | H                | H                | — |   | —                     | — | — | — |
| A604     | A       | H                | H                | H                | H                | H                | H                | — |   | —                     | — | — | — |
| A605     | A       | H                | H                | H                | H                | H                | H                | — |   | —                     | — | — | — |
| A606     | A       | H                | H                | H                | H                | H                | H                |   | — | —                     | — | — |   |

TABLE 6-continued

| Compound | Example         |           |           |           |           |           |           | A        |         |                 |
|----------|-----------------|-----------|-----------|-----------|-----------|-----------|-----------|----------|---------|-----------------|
|          |                 | $R^{601}$ | $R^{602}$ | $R^{603}$ | $R^{604}$ | $R^{605}$ | $R^{606}$ | $\alpha$ | $\beta$ | $\gamma$        |
| A607     | A               | H         | H         | H         | H         | H         | H         |          | —       | —               |
| A608     | A               | H         | H         | H         | H         | H         | H         | —        | —       | COOH            |
| A609     | A               | H         | H         | H         | H         | H         | H         | —        | —       | NH <sub>2</sub> |
| A610     | A               | CN        | H         | H         | H         | H         | H         | —        | —       | NH <sub>2</sub> |
| A611     | CN              | CN        | A         | H         | H         | H         | H         | —        | —       | NH <sub>2</sub> |
| A612     | A               | H         | H         | H         | H         | H         | H         | —        | —       | OH              |
| A613     | H               | H         | A         | H         | H         | H         | H         | —        | —       | OH              |
| A614     | CH <sub>3</sub> | H         | A         | H         | H         | H         | H         | —        | —       | OH              |
| A615     | H               | H         | A         | H         | H         | A         | —         | —        | —       | OH              |
| A616     | A               | A         | H         | H         | H         | H         | —         |          |         |                 |
| A617     | A               | A         | H         | H         | H         | H         |           | —        | —       | —               |
| A618     | A               | A         | H         | H         | H         | H         |           | —        | —       | —               |
| A619     | A               | A         | H         | H         | H         | H         | —         | —        | —       | COOH            |

Specific examples of compounds represented by the above formula (A7) are shown in Table 7-1, Table 7-2 and Table 7-3. In the Tables, the case where  $\gamma$  is “-” indicates a hydrogen atom, and the hydrogen atom for the  $\gamma$  is incorporated into the structure given in the column of  $\alpha$  or  $\beta$ . <sup>35</sup>

TABLE 7-1

| Com-<br>ound<br>Exam-<br>ple |   | A         |           |           |           |           |           |           |                 |          |         |          |
|------------------------------|---|-----------|-----------|-----------|-----------|-----------|-----------|-----------|-----------------|----------|---------|----------|
|                              |   | $R^{701}$ | $R^{702}$ | $R^{703}$ | $R^{704}$ | $R^{705}$ | $R^{706}$ | $R^{707}$ | $R^{708}$       | $\alpha$ | $\beta$ | $\gamma$ |
| A701                         | A | H         | H         | H         | H         | H         | H         | H         | H               | —        |         |          |
| A702                         | A | H         | H         | H         | H         | H         | H         | H         | H               | —        |         |          |
| A703                         | A | H         | H         | H         | H         | H         | H         | H         | NO <sub>2</sub> | —        |         |          |
| A704                         | A | H         | H         | H         | H         | H         | H         | H         | H               | —        |         | COOH     |

TABLE 7-1-continued

| Com-<br>ound<br>Exam-<br>ple | R <sup>701</sup> | R <sup>702</sup> | R <sup>703</sup> | R <sup>704</sup> | R <sup>705</sup> | R <sup>706</sup> | R <sup>707</sup> | R <sup>708</sup> | A |   |                       |
|------------------------------|------------------|------------------|------------------|------------------|------------------|------------------|------------------|------------------|---|---|-----------------------|
|                              |                  |                  |                  |                  |                  |                  |                  |                  | α | β | γ                     |
| A705                         | A                | H                | H                | H                | H                | H                | H                | H                | — |   | —                     |
| A706                         | A                | H                | H                | H                | H                | H                | H                | H                | — |   | —                     |
| A707                         | A                | H                | H                | H                | H                | H                | H                | H                |   | — | —                     |
| A708                         | A                | H                | H                | H                | H                | H                | H                | H                | — | — | COOH                  |
| A709                         | A                | H                | H                | H                |                  | H                | H                | H                | — | — | COOH                  |
| A710                         | A                | H                | H                | H                | A                | H                | H                | H                | — |   | ---CH <sub>2</sub> OH |
| A711                         | A                | H                | H                | H                | A                | H                | H                | H                | — |   | ---CH <sub>2</sub> OH |
| A712                         | A                | H                | H                | NO <sub>2</sub>  | A                | H                | H                | NO <sub>2</sub>  | — |   | ---CH <sub>2</sub> OH |
| A713                         | A                | H                | F                | H                | A                | H                | F                | H                | — |   | ---CH <sub>2</sub> OH |
| A714                         | A                | H                | H                | H                | A                | H                | H                | H                | — |   | —                     |
| A715                         | A                | H                | H                | H                | A                | H                | H                | H                | — |   | —                     |

TABLE 7-2

| Compound Exam- | ple | A         |           |           |           |           |           |           |           | $\alpha$ | $\beta$                      | $\gamma$ |
|----------------|-----|-----------|-----------|-----------|-----------|-----------|-----------|-----------|-----------|----------|------------------------------|----------|
|                |     | $R^{701}$ | $R^{702}$ | $R^{703}$ | $R^{704}$ | $R^{705}$ | $R^{706}$ | $R^{707}$ | $R^{708}$ |          |                              |          |
| A716           | A   | H         | H         | H         | A         | H         | H         | H         | H         | —        |                              | —        |
| A717           | A   | H         | H         | H         | A         | H         | H         | H         | —         |          | —                            | —        |
| A718           | A   | H         | H         | H         | A         | H         | H         | H         | —         | —        | —                            | COOH     |
| A719           | H   | A         | H         | H         | H         | A         | H         | H         | —         | —        | —                            | COOH     |
| A720           | A   | H         | H         | H         | A         | F         | H         | H         | —         | —        | —                            | COOH     |
| A721           | A   | H         | H         | $CH_3$    | $CH_3$    | H         | H         | H         | —         | —        | —                            | COOH     |
| A722           | A   | H         | H         | $C_4H_9$  | $C_4H_9$  | H         | H         | H         | —         | —        | —                            | COOH     |
| A723           | A   | H         | H         |           |           | H         | H         | H         | —         | —        | —                            | COOH     |
| A724           | A   | H         | H         | $CH_3$    | $CH_3$    | H         | H         | H         | —         |          | $\text{---CH}_2\text{---OH}$ | —        |
| A725           | A   | H         | H         | $C_4H_9$  | $C_4H_9$  | H         | H         | H         | —         |          | $\text{---CH}_2\text{---OH}$ | —        |
| A726           | A   | H         | H         |           |           | H         | H         | H         | —         |          | $\text{---CH}_2\text{---OH}$ | —        |
| A727           | A   | H         | H         | $C_4H_9$  | $C_4H_9$  | H         | H         | H         | —         |          | —                            | —        |
| A728           | A   | H         | H         | $C_4H_9$  | $C_4H_9$  | H         | H         | H         | —         |          | —                            | —        |
| A729           | A   | H         | H         | $C_4H_9$  | $C_4H_9$  | H         | H         | H         | —         |          | —                            | —        |

TABLE 7-3

| Compound Exam- | ple | A         |           |           |           |           |           |           |           | A'       |         |                                         |                                         |         |                              |
|----------------|-----|-----------|-----------|-----------|-----------|-----------|-----------|-----------|-----------|----------|---------|-----------------------------------------|-----------------------------------------|---------|------------------------------|
|                |     | $R^{701}$ | $R^{702}$ | $R^{703}$ | $R^{704}$ | $R^{705}$ | $R^{706}$ | $R^{707}$ | $R^{708}$ | $\alpha$ | $\beta$ | $\gamma$                                | $\alpha$                                | $\beta$ | $\gamma$                     |
| A730           | A   | H         | H         | H         | H         | A'        | H         | H         | H         |          | —       | —                                       | —                                       |         | $\text{---CH}_2\text{---OH}$ |
| A731           | A   | H         | H         | H         | H         | A'        | H         | H         | H         | —        |         | $\text{---CH}_2\text{---OH}$            | $\text{---CH}_2\text{---OH}$            | —       | —                            |
| A733           | A   | H         | H         | H         | H         | A'        | H         | H         | H         | —        |         | $\text{---C}_2\text{H}_2\text{---COOH}$ | $\text{---C}_2\text{H}_2\text{---COOH}$ | —       | —                            |

Specific examples of compounds represented by the above formula (A8) are shown in Table 8-1, Table 8-2 and Table 8-3. In the Tables, the case where  $\gamma$  is “-” indicates a hydrogen atom, and the hydrogen atom for the  $\gamma$  is incorporated into the structure given in the column of  $\alpha$  or  $\beta$ .

TABLE 8-1

| Compound Exam- | ple | A                |                  |                  |                  |                  |                  |                  |                                                                                     |                  |                                                                                       |                                                                                       |                                                                                       |
|----------------|-----|------------------|------------------|------------------|------------------|------------------|------------------|------------------|-------------------------------------------------------------------------------------|------------------|---------------------------------------------------------------------------------------|---------------------------------------------------------------------------------------|---------------------------------------------------------------------------------------|
|                |     | R <sup>801</sup> | R <sup>802</sup> | R <sup>803</sup> | R <sup>804</sup> | R <sup>805</sup> | R <sup>806</sup> | R <sup>807</sup> | R <sup>808</sup>                                                                    | R <sup>809</sup> | R <sup>810</sup>                                                                      | α                                                                                     | β                                                                                     |
| A801           | H   | H                | H                | H                | H                | H                | H                | H                |    | A                |    | —                                                                                     | —                                                                                     |
| A802           | H   | H                | H                | H                | H                | H                | H                | H                |    | A                |    | —                                                                                     | —                                                                                     |
| A803           | H   | H                | H                | H                | H                | H                | H                | H                |    | A                | —                                                                                     |    |    |
| A804           | H   | H                | H                | H                | H                | H                | H                | H                |    | A                | —                                                                                     |    | --CH <sub>2</sub> -OH                                                                 |
| A805           | H   | H                | H                | H                | H                | H                | H                | H                |   | A                | —                                                                                     |    | --CH <sub>2</sub> -OH                                                                 |
| A806           | H   | H                | H                | H                | H                | H                | H                | H                |  | A                |  | —                                                                                     | —                                                                                     |
| A807           | H   | H                | H                | H                | H                | H                | H                | H                |  | A                |  | —                                                                                     | —                                                                                     |
| A808           | H   | H                | H                | H                | H                | H                | H                | H                |  | A                |  | —                                                                                     | —                                                                                     |
| A809           | H   | H                | H                | H                | H                | H                | H                | H                |  | A                | —C <sub>5</sub> H <sub>10</sub> -OH                                                   | —                                                                                     | —                                                                                     |
| A810           | H   | H                | H                | H                | H                | H                | H                | H                | —C <sub>6</sub> H <sub>13</sub>                                                     | A                |  | —                                                                                     | —                                                                                     |
| A811           | H   | H                | H                | H                | H                | H                | H                | H                |  | A                | —                                                                                     |  |  |
| A812           | H   | H                | H                | H                | H                | H                | H                | H                |  | A                | —                                                                                     |  | —                                                                                     |
| A813           | H   | H                | H                | H                | H                | H                | H                | H                |  | A                | —                                                                                     |  | —                                                                                     |

TABLE 8-1-continued

| Compound Exam- | ple |                  |                  |                  |                  |                  |                  |                  |                  |                  |                  | A |   |   |
|----------------|-----|------------------|------------------|------------------|------------------|------------------|------------------|------------------|------------------|------------------|------------------|---|---|---|
|                |     | R <sup>801</sup> | R <sup>802</sup> | R <sup>803</sup> | R <sup>804</sup> | R <sup>805</sup> | R <sup>806</sup> | R <sup>807</sup> | R <sup>808</sup> | R <sup>809</sup> | R <sup>810</sup> | α | β | γ |
| A814           | H   | H                | H                | H                | H                | H                | H                | H                |                  | A                | —                |   | — | — |
| A815           | H   | H                | H                | H                | H                | H                | H                | H                |                  | A                | —                |   | — | — |

TABLE 8-2

| Compound Exam- | ple |                  |                  |                  |                  |                  |                  |                  |                  |                  |                  | A |   |       |
|----------------|-----|------------------|------------------|------------------|------------------|------------------|------------------|------------------|------------------|------------------|------------------|---|---|-------|
|                |     | R <sup>801</sup> | R <sup>802</sup> | R <sup>803</sup> | R <sup>804</sup> | R <sup>805</sup> | R <sup>806</sup> | R <sup>807</sup> | R <sup>808</sup> | R <sup>809</sup> | R <sup>810</sup> | α | β | γ     |
| A816           | H   | H                | H                | H                | H                | H                | H                | H                |                  | A                | —                |   | — | —     |
| A817           | H   | H                | H                | H                | H                | H                | H                | H                |                  | A                | —                |   | — | —     |
| A818           | H   | H                | H                | H                | H                | H                | H                | H                |                  | A                | —                |   |   | —     |
| A819           | H   | CN               | H                | H                | H                | H                | CN               | H                |                  | A                |                  |   | — | —     |
| A820           | H   |                  | H                | H                | H                | H                |                  | H                |                  | A                |                  |   | — | —     |
| A821           | H   | A                | H                | H                | H                | H                | H                | H                |                  |                  | —                | — | — | —COOH |
| A822           | H   | Cl               | Cl               | H                | H                | Cl               | Cl               | H                |                  | A                |                  |   | — | —     |
| A823           | H   | H                | H                | H                | H                | H                | H                | H                |                  | A                |                  |   | — | —     |

TABLE 8-2-continued

| Compound<br>Ex-<br>am-<br>ple | A                |                                                                                     |                  |                  |                  |                  |                                                                                     |                  |                                                                                     |                  | α                                                                                   | β                                                                                     | γ                                                                                     |
|-------------------------------|------------------|-------------------------------------------------------------------------------------|------------------|------------------|------------------|------------------|-------------------------------------------------------------------------------------|------------------|-------------------------------------------------------------------------------------|------------------|-------------------------------------------------------------------------------------|---------------------------------------------------------------------------------------|---------------------------------------------------------------------------------------|
|                               | R <sup>801</sup> | R <sup>802</sup>                                                                    | R <sup>803</sup> | R <sup>804</sup> | R <sup>805</sup> | R <sup>806</sup> | R <sup>807</sup>                                                                    | R <sup>808</sup> | R <sup>809</sup>                                                                    | R <sup>810</sup> | α                                                                                   | β                                                                                     | γ                                                                                     |
| A824                          | H                | H                                                                                   | H                | H                | H                | H                | H                                                                                   | H                | A                                                                                   | A                |  | —                                                                                     | —                                                                                     |
| A825                          | H                | H                                                                                   | H                | H                | H                | H                | H                                                                                   | H                | A                                                                                   | A                | —                                                                                   |    |    |
| A826                          | H                | H                                                                                   | H                | H                | H                | H                | H                                                                                   | H                | A                                                                                   | A                | —                                                                                   |    | —                                                                                     |
| A827                          | H                | H                                                                                   | H                | H                | H                | H                | H                                                                                   | H                | A                                                                                   | A                | —                                                                                   |    | —                                                                                     |
| A828                          | H                | H                                                                                   | H                | H                | H                | H                | H                                                                                   | H                | A                                                                                   | A                | —                                                                                   |    | —                                                                                     |
| A829                          | H                | H                                                                                   | H                | H                | H                | H                | H                                                                                   | H                | A                                                                                   | A                | —                                                                                   |    | —                                                                                     |
| A830                          | H                | H                                                                                   | H                | H                | H                | H                | H                                                                                   | H                | A                                                                                   | A                | —                                                                                   |   | —                                                                                     |
| A831                          | H                |  | H                | H                | H                | H                |  | H                |  | A                | —                                                                                   |  |  |

TABLE 8-3

| Compound<br>Ex-<br>am-<br>ple | A                |                  |                  |                  |                  |                  |                  |                  |                  |                  |
|-------------------------------|------------------|------------------|------------------|------------------|------------------|------------------|------------------|------------------|------------------|------------------|
|                               | R <sup>801</sup> | R <sup>802</sup> | R <sup>803</sup> | R <sup>804</sup> | R <sup>805</sup> | R <sup>806</sup> | R <sup>807</sup> | R <sup>808</sup> | R <sup>809</sup> | R <sup>810</sup> |
| A832                          | H                | H                | H                | H                | H                | H                | H                | H                | A                | A'               |
| A833                          | H                | H                | H                | H                | H                | H                | H                | H                | A                | A'               |
| A834                          | H                | H                | H                | H                | H                | H                | H                | H                | A                | A'               |
| A835                          | H                | H                | H                | H                | H                | H                | H                | H                | A                | A'               |

  

| Compound<br>Ex-<br>am-<br>ple | A                                                                                   |                                                                                     |                         |                         |                                                                                     |   | A' |   |   |   |
|-------------------------------|-------------------------------------------------------------------------------------|-------------------------------------------------------------------------------------|-------------------------|-------------------------|-------------------------------------------------------------------------------------|---|----|---|---|---|
|                               | α                                                                                   | β                                                                                   | γ                       | α                       | β                                                                                   | γ | α  | β | γ | α |
| A832                          |  | —                                                                                   | —                       | —                       |  | — | —  | — | — | — |
| A833                          | —                                                                                   |  | ----CH <sub>2</sub> -OH | ----CH <sub>2</sub> -OH |  | — | —  | — | — | — |

TABLE 8-3-continued

|      |   |  |                                      |                                      |                         |   |
|------|---|--|--------------------------------------|--------------------------------------|-------------------------|---|
| A834 | — |  | ----C <sub>H<sub>2</sub></sub> —COOH | ----C <sub>H<sub>2</sub></sub> —COOH | —                       | — |
| A835 | — |  | —                                    |                                      | ----CH <sub>2</sub> —OH | — |

Specific examples of compounds represented by the above formula (A9) are shown in Table 9-1 and Table 9-2. In the Tables, the case where  $\gamma$  is “-” indicates a hydrogen atom, and the hydrogen atom for the  $\gamma$  is incorporated into the structure given in the column of  $\alpha$  or  $\beta$ .

15

TABLE 9-1

| Com-<br>pound<br>Exam-<br>ple | A                |                  |                  |                  |                  |                  |                  |                  |                                     |         |                     |                     |
|-------------------------------|------------------|------------------|------------------|------------------|------------------|------------------|------------------|------------------|-------------------------------------|---------|---------------------|---------------------|
|                               | R <sup>901</sup> | R <sup>902</sup> | R <sup>903</sup> | R <sup>904</sup> | R <sup>905</sup> | R <sup>906</sup> | R <sup>907</sup> | R <sup>908</sup> | $\alpha$                            | $\beta$ | $\gamma$            |                     |
| A901                          | A                | H                | H                | H                | H                | H                | H                | H                | —CH <sub>2</sub> —OH                | —       | —                   |                     |
| A902                          | A                | H                | H                | H                | H                | H                | H                | H                | —(CH <sub>2</sub> ) <sub>2</sub> OH | —       | —                   |                     |
| A903                          | A                | H                | H                | H                |                  | H                | H                | H                | —(CH <sub>2</sub> ) <sub>2</sub> OH | —       | —                   |                     |
| A904                          | A                |                  | H                | H                |                  | H                | H                | H                | —(CH <sub>2</sub> ) <sub>2</sub> OH | —       | —                   |                     |
| A905                          | A                | NO <sub>2</sub>  | H                | H                | H                | NO <sub>2</sub>  | H                | H                | —(CH <sub>2</sub> ) <sub>2</sub> OH | —       | —                   |                     |
| A906                          | A                | H                | H                | H                | H                | A                | H                | H                | —(CH <sub>2</sub> ) <sub>2</sub> OH | —       | —                   |                     |
| A907                          | A                | H                | H                | H                | A                | H                | H                | H                | —(CH <sub>2</sub> ) <sub>2</sub> OH | —       | —                   |                     |
| A908                          | A                | H                | H                | H                | A                | H                | H                | H                | —                                   |         | —                   |                     |
| A909                          | A                | H                | H                | A                | H                | H                | H                | H                | —(CH <sub>2</sub> ) <sub>2</sub> OH | —       | —                   |                     |
| A910                          | A                | H                | H                | A                | H                | H                | H                | H                | —                                   |         | —                   |                     |
| A911                          | H                | H                | H                | H                | H                | H                | H                | A                | —CH <sub>2</sub> —OH                | —       | —                   |                     |
| A912                          | H                | H                | H                | H                | H                | H                | H                | A                | —(CH <sub>2</sub> ) <sub>2</sub> OH | —       | —                   |                     |
| A913                          | H                | NO <sub>2</sub>  | H                | H                | H                | NO <sub>2</sub>  | H                | A                | —(CH <sub>2</sub> ) <sub>2</sub> OH | —       | —                   |                     |
| A914                          | H                | H                | H                | H                | H                | H                | H                | A                | —                                   |         | —                   |                     |
| A915                          | H                | H                | H                | H                | H                | H                | H                | A                | —                                   |         | H <sub>2</sub> C—OH | ----CH <sub>2</sub> |

TABLE 9-1-continued

| Com-<br>ound<br>Exam-<br>ple | A                |                  |                  |                  |                  |                  |                  |                  |                                     |                                                                                     |                                                                                      |
|------------------------------|------------------|------------------|------------------|------------------|------------------|------------------|------------------|------------------|-------------------------------------|-------------------------------------------------------------------------------------|--------------------------------------------------------------------------------------|
|                              | R <sup>901</sup> | R <sup>902</sup> | R <sup>903</sup> | R <sup>904</sup> | R <sup>905</sup> | R <sup>906</sup> | R <sup>907</sup> | R <sup>908</sup> | α                                   | β                                                                                   | γ                                                                                    |
| A916                         | H                | H                | H                | H                | H                | H                | H                | A                | —                                   |   | —                                                                                    |
| A917                         | H                | H                | H                | H                | H                | H                | H                | A                | —                                   |   | —                                                                                    |
| A918                         | H                | H                | H                | H                | H                | H                | H                | A                | —                                   |   | —                                                                                    |
| A919                         | H                | CN               | H                | H                | H                | H                | CN               | A                | —                                   |   | —                                                                                    |
| A920                         | A                | A                | H                | H                | H                | H                | H                | H                | —(CH <sub>2</sub> ) <sub>2</sub> OH | —                                                                                   | —                                                                                    |
| A921                         | A                | A                | H                | NO <sub>2</sub>  | H                | H                | NO <sub>2</sub>  | H                | —(CH <sub>2</sub> ) <sub>2</sub> OH | —                                                                                   | —                                                                                    |
| A922                         | H                | A                | A                | H                | H                | H                | H                | H                | —                                   | —                                                                                   | OH                                                                                   |
| A923                         | H                | H                | A                | H                | H                | H                | H                | H                | —(CH <sub>2</sub> ) <sub>6</sub> OH | —                                                                                   | —                                                                                    |
| A924                         | H                | H                | A                | H                | H                | H                | H                | A                | —                                   |  |  |

TABLE 9-2

| Com-<br>ound<br>Exam-<br>ple | A                |                  |                  |                  |                  |                  |                  |                  |                                     |   | A' |                                                                                       |   |
|------------------------------|------------------|------------------|------------------|------------------|------------------|------------------|------------------|------------------|-------------------------------------|---|----|---------------------------------------------------------------------------------------|---|
|                              | R <sup>901</sup> | R <sup>902</sup> | R <sup>903</sup> | R <sup>904</sup> | R <sup>905</sup> | R <sup>906</sup> | R <sup>907</sup> | R <sup>908</sup> | α                                   | β | γ  | α                                                                                     | β |
| A925                         | A                | H                | H                | H                | A'               | H                | H                | H                | —(CH <sub>2</sub> ) <sub>2</sub> OH | — | —  |  | — |
| A926                         | A                | H                | H                | A'               | H                | H                | H                | H                | —(CH <sub>2</sub> ) <sub>2</sub> OH | — | —  |  | — |
| A927                         | H                | A'               | H                | H                | H                | H                | H                | A                | —(CH <sub>2</sub> ) <sub>6</sub> OH | — | —  |  | — |

A derivative (derivative of an electron transporting substance) having a structure of (A1) can be synthesized by a well-known synthesis method described, for example, in U.S. Pat. Nos. 4,442,193, 4,992,349 and 5,468,583 and Chemistry of Materials, Vol. 19, No. 11, 2703-2705 (2007). The derivative can also be synthesized by a reaction of a naphthalene-tetracarboxylic dianhydride and a monoamine derivative, which are commercially available from Tokyo Chemical Industry Co., Ltd., Sigma-Aldrich Japan Co., Ltd. and Johnson Matthey Japan Inc.

A compound represented by (A1) has polymerizable functional groups (a hydroxy group, a thiol group, an amino group, a carboxyl group and a methoxy group) polymerizable with a crosslinking agent. A method for incorporating these polymerizable functional groups in a derivative having an

(A1) structure includes a method of directly incorporating the polymerizable functional groups in the derivative having an (A1) structure, and a method of incorporating structures having the polymerizable functional groups or functional groups capable of becoming precursors of polymerizable functional groups in the derivative having an (A1) structure. Examples of the latter method include, based on a halide of a naphthylimide derivative, a method of incorporating a functional group-containing aryl group for example, by using a cross coupling reaction using a palladium catalyst and a base, a method of incorporating a functional group-containing alkyl group by using a cross coupling reaction using an FeCl<sub>3</sub> catalyst and a base and a method of incorporating a hydroxy-alkyl group and a carboxyl group by making an epoxy compound or CO<sub>2</sub> to act after lithiation. There is a method of using

a naphthalenetetracarboxylic dianhydride derivative or a monoamine derivative having the polymerizable functional groups or functional groups capable of becoming precursors of polymerizable functional groups as a raw material for synthesis of the naphthylimide derivative.

Derivatives having an (A2) structure are commercially available, for example, from Tokyo Chemical Industry Co., Ltd., Sigma-Aldrich Japan Co., Ltd. and Johnson Matthey Japan Inc. The derivatives can also be synthesized based on a phenanthrene derivative or a phenanthroline derivative by synthesis methods described in Chem. Educator No. 6, 227-234 (2001), Journal of Synthetic Organic Chemistry, Japan, vol. 15, 29-32 (1957) and Journal of Synthetic Organic Chemistry, Japan, vol. 15, 32-34 (1957). A dicyanomethylene group can also be incorporated by a reaction with malononitrile.

A compound represented by (A2) has polymerizable functional groups (a hydroxy group, a thiol group, an amino group, a carboxyl group and a methoxy group) polymerizable with a crosslinking agent. A method for incorporating these polymerizable functional groups in a derivative having an (A2) structure includes a method of directly incorporating the polymerizable functional groups in the derivative having an (A2) structure, and a method of incorporating structures having the polymerizable functional groups or functional groups capable of becoming precursors of polymerizable functional groups in the derivative having an (A2) structure. Examples of the latter method include, based on a halide of phenanthrenequinone, a method of incorporating a functional group-containing aryl group by using a cross coupling reaction using a palladium catalyst and a base, a method of incorporating a functional group-containing alkyl group by using a cross coupling reaction using an  $FeCl_3$  catalyst and a base and a method of incorporating a hydroxyl group and a carboxyl group by making an epoxy compound or  $CO_2$  to act after lithiation.

Derivatives having an (A3) structure are commercially available from Tokyo Chemical Industry Co., Ltd., Sigma-Aldrich Japan Co., Ltd. and Johnson Matthey Japan Inc. The derivatives can also be synthesized based on a phenanthrene derivative or a phenanthroline derivative by a synthesis method described in Bull. Chem. Soc., Jpn., Vol. 65, 1006-1011 (1992). A dicyanomethylene group can also be incorporated by a reaction with malononitrile.

A compound represented by (A3) has polymerizable functional groups (a hydroxy group, a thiol group, an amino group, a carboxyl group and a methoxy group) polymerizable with a crosslinking agent. A method for incorporating these polymerizable functional groups in a derivative having the structure of the above formula (A3) includes a method of directly incorporating the polymerizable functional groups in the derivative having the structure of formula (A3), and a method of incorporating structures having the polymerizable functional groups or functional groups capable of becoming precursors of polymerizable functional groups in the derivative having the structure of formula (A3). Examples of the latter method include, based on a halide of phenanthroline-quinone, a method of incorporating a functional group-containing aryl group by using a cross coupling reaction using a palladium catalyst and a base, a method of incorporating a functional group-containing alkyl group by using a cross coupling reaction using an  $FeCl_3$  catalyst and a base and a method of incorporating a hydroxyl group and a carboxyl group by making an epoxy compound or  $CO_2$  to act after lithiation.

Derivatives having an (A4) structure are commercially available, for example, from Tokyo Chemical Industry Co.,

Ltd., Sigma-Aldrich Japan Co., Ltd. and Johnson Matthey Japan Inc. The derivatives can also be synthesized based on an acenaphthenequinone derivative by synthesis methods described in Tetrahedron Letters, 43 (16), 2991-2994 (2002) and Tetrahedron Letters, 44 (10), 2087-2091 (2003). A dicyanomethylene group can also be incorporated by a reaction with malononitrile.

A compound represented by the formula (A4) has polymerizable functional groups (a hydroxy group, a thiol group, an amino group, a carboxyl group and a methoxy group) polymerizable with a crosslinking agent. A method for incorporating these polymerizable functional groups in a derivative having an (A4) structure includes a method of directly incorporating the polymerizable functional groups in the derivative having an (A4) structure, and a method of incorporating structures having the polymerizable functional groups or functional groups capable of becoming precursors of polymerizable functional groups in the derivative having an (A4) structure. Examples of the latter method include, based on a halide of acenaphthenequinone, a method of incorporating a functional group-containing aryl group for example, by using a cross coupling reaction using a palladium catalyst and a base, a method of incorporating a functional group-containing alkyl group by using a cross coupling reaction using an  $FeCl_3$  catalyst and a base and a method of incorporating a hydroxyl group and a carboxyl group by making an epoxy compound or  $CO_2$  to act after lithiation.

Derivatives having an (A5) structure are commercially available, for example, from Tokyo Chemical Industry Co., Ltd., Sigma-Aldrich Japan Co., Ltd. and Johnson Matthey Japan Inc. The derivatives can also be synthesized using a fluorenone derivative and malononitrile by a synthesis method described in U.S. Pat. No. 4,562,132. The derivatives can also be synthesized using a fluorenone derivative and an aniline derivative by synthesis methods described in Japanese Patent Application Laid-Open Nos. H05-279582 and H07-70038.

A compound represented by the formula (A5) has polymerizable functional groups (a hydroxy group, a thiol group, an amino group, a carboxyl group and a methoxy group) polymerizable with a crosslinking agent. A method for incorporating these polymerizable functional groups in a derivative having an (A5) structure includes a method of directly incorporating the polymerizable functional groups in the derivative having an (A5) structure, and a method of incorporating structures having the polymerizable functional groups or functional groups capable of becoming precursors of polymerizable functional groups in the derivative having an (A5) structure. Examples of the latter method include, based on a halide of fluorenone, a method of incorporating a functional group-containing aryl group for example, by using a cross coupling reaction using a palladium catalyst and a base, a method of incorporating a functional group-containing alkyl group by using a cross coupling reaction using an  $FeCl_3$  catalyst and a base and a method of incorporating a hydroxyl group and a carboxyl group by making an epoxy compound or  $CO_2$  to act after lithiation.

Derivatives having an (A6) structure can be synthesized by synthesis methods described in, for example, Chemistry Letters, 37(3), 360-361 (2008) and Japanese Patent Application Laid-Open No. H09-151157. The derivatives are commercially available from Tokyo Chemical Industry Co., Ltd., Sigma-Aldrich Japan Co., Ltd. and Johnson Matthey Japan Inc.

A compound represented by the formula (A6) has polymerizable functional groups (a hydroxy group, a thiol group, an amino group, a carboxyl group and a methoxy group)

polymerizable with a crosslinking agent. A method for incorporating these polymerizable functional groups in a derivative having an (A6) structure includes a method of directly incorporating the polymerizable functional groups in a naphthoquinone derivative, and a method of incorporating structures having the polymerizable functional groups or functional groups capable of becoming precursors of polymerizable functional groups in a naphthoquinone derivative. Examples of the latter method include, based on a halide of naphthoquinone, a method of incorporating a functional group-containing aryl group for example, by using a cross coupling reaction using a palladium catalyst and a base, a method of incorporating a functional group-containing alkyl group by using a cross coupling reaction using an  $\text{FeCl}_3$  catalyst and a base and a method of incorporating a hydroxyl group and a carboxyl group by making an epoxy compound or  $\text{CO}_2$  to act after lithiation.

Derivatives having an (A7) structure can be synthesized by synthesis methods described in Japanese Patent Application Laid-Open No. H01-206349 and Proceedings of PPCI/Japan Hard Copy '98, Proceedings, p. 207 (1998). The derivatives can be synthesized, for example, using phenol derivatives commercially available from Tokyo Chemical Industry Co., Ltd., or Sigma-Aldrich Japan Co., Ltd., as a raw material.

A compound represented by (A7) has polymerizable functional groups (a hydroxy group, a thiol group, an amino group, a carboxyl group and a methoxy group) polymerizable with a crosslinking agent. A method for incorporating these polymerizable functional groups in a derivative having an (A7) structure includes a method of incorporating structures having the polymerizable functional groups or functional groups capable of becoming precursors of polymerizable functional groups. Examples of the method include, based on a halide of diphenoquinone, a method of incorporating a functional group-containing aryl group for example, by using a cross coupling reaction using a palladium catalyst and a base, a method of incorporating a functional group-containing alkyl group by using a cross coupling reaction using an  $\text{FeCl}_3$  catalyst and a base and a method of incorporating a hydroxyl group and a carboxyl group by making an epoxy compound or  $\text{CO}_2$  to act after lithiation.

Derivatives having an (A8) structure can be synthesized by a well-known synthesis method described in, for example, Journal of the American Chemical Society, Vol. 129, No. 49, 15259-78 (2007). The derivatives can also be synthesized by a reaction of perylenetetracarboxylic dianhydride and a monoamine derivative commercially available from Tokyo Chemical Industry Co., Ltd., Sigma-Aldrich Japan Co., Ltd. and Johnson Matthey Japan Inc.

A compound represented by the formula (A8) has polymerizable functional groups (a hydroxy group, a thiol group, an amino group, a carboxyl group and a methoxy group) polymerizable with a crosslinking agent. A method for incorporating these polymerizable functional groups in a derivative having an (A8) structure includes a method of directly incorporating the polymerizable functional groups in the derivative having an (A8) structure, and a method of incorporating structures having the polymerizable functional groups or functional groups capable of becoming precursors of polymerizable functional groups in the derivative having an (A8) structure. Examples of the latter method include, based on a halide of a peryleneimide derivative, a method of using a cross coupling reaction using a palladium catalyst and a base and a method of using a cross coupling reaction using an  $\text{FeCl}_3$  catalyst and a base. There is a method of using perylenetetracarboxylic dianhydride derivative or a monoamine derivative having the polymerizable functional groups or

functional groups capable of becoming precursors of polymerizable functional groups as a raw material for synthesis of the peryleneimide derivative.

Derivatives having an (A9) structure are commercially available, for example, from Tokyo Chemical Industry Co., Ltd., Sigma-Aldrich Japan Co., Ltd. and Johnson Matthey Japan Inc.

A compound represented by the formula (A9) has polymerizable functional groups (a hydroxy group, a thiol group, an amino group, a carboxyl group and a methoxy group) polymerizable with a crosslinking agent. A method for incorporating these polymerizable functional groups in a derivative having an (A9) structure includes a method of incorporating structures having the polymerizable functional groups or functional groups capable of becoming precursors of polymerizable functional groups, in an anthraquinone derivative commercially available. Examples of the method include, based on a halide of anthraquinone, a method of incorporating a functional group-containing aryl group for example, by using a cross coupling reaction using a palladium catalyst and a base, a method of incorporating a functional group-containing alkyl group by using a cross coupling reaction using an  $\text{FeCl}_3$  catalyst and a base and a method of incorporating a hydroxyl group and a carboxyl group by making an epoxy compound or  $\text{CO}_2$  to act after lithiation.

#### Crosslinking Agent

Then, a crosslinking agent will be described. As a crosslinking agent, a compound can be used which polymerizes with or crosslinks with an electron transporting substance having polymerizable functional groups and a thermoplastic resin having polymerizable functional groups. Specifically, compounds described in "Crosslinking Agent Handbook", edited by Shinzo Yamashita, Tosuke Kaneko, published by Taiseisha Ltd. (1981) (in Japanese), and the like can be used.

Crosslinking agents used for an electron transporting layer can be isocyanate compounds and amine compounds. The crosslinking agents are more preferably crosslinking agents (isocyanate compounds, amine compounds) having 3 to 6 groups of an isocyanate group, a blocked isocyanate group or a monovalent group represented by  $-\text{CH}_2-\text{OR}^1$  from the viewpoint of providing a uniform layer of a polymer.

As the isocyanate compound, an isocyanate compound having a molecular weight in the range of 200 to 1,300 can be used. An isocyanate compound having 3 to 6 isocyanate groups or blocked isocyanate groups can further be used. Examples of the isocyanate compound include isocyanate modifications, biuret modifications, allophanate modifications and trimethylolpropane or pentaerythritol adduct modifications of triisocyanatobenzene, triisocyanatomethylbenzene, triphenylmethane triisocyanate, lysine triisocyanate, and additionally, diisocyanates such as tolylene diisocyanate, hexamethylene diisocyanate, dicyclohexylmethane diisocyanate, naphthalene diisocyanate, diphenylmethane diisocyanate, isophorone diisocyanate, xylylene diisocyanate, 2,2,4-trimethylhexamethylene diisocyanate, methyl-2,6-diisocyanate hexanoate and norbornane diisocyanate. Above all, the modified isocyanate and the modified adducts are more preferable.

A blocked isocyanate group is a group having a structure of  $-\text{NHCX}^1$  ( $X^1$  is a blocking group).  $X^1$  may be any blocking group as long as  $X^1$  can be incorporated to an isocyanate group, but is more preferably a group represented by one of the following formulae (H1) to (H7).

75



(H1)

76  
-continued

(H5)



(H2)

15



(H6)



(H3)

25



(H7)



(H4)

35 Hereinafter, specific examples of isocyanate compounds will be described.



(B1)



(B2)



(B3)



(B4)



-continued

(B5)



(B6)



(B7)



(B8)



(B9)



(B10)



(B11)



79



80

-continued

(B12)



(B13)

(B14)



(B15)

(B16)



(B17)



81



82

-continued  
(B18)

(B19)

(B20)



(B21)



The amine compound can be at least one selected from the group consisting of compounds represented by the following formula (C1), oligomers of compounds represented by the following formula (C1), compounds represented by the following formula (C2), oligomers of compounds represented by the following formula (C2), compounds represented by the following formula (C3), oligomers of compounds represented by the following formula (C3), compounds represented by the following formula (C4), oligomers of compounds represented by the following formula (C4), compounds represented by the following formula (C5), and oligomers of compounds represented by the following formula (C5).



-continued

(C3)



In the formulae (C1) to (C5), R<sup>11</sup> to R<sup>26</sup>, R<sup>22</sup> to R<sup>25</sup>, R<sup>31</sup> to R<sup>34</sup>, R<sup>41</sup> to R<sup>44</sup> and R<sup>51</sup> to R<sup>54</sup> each independently represent a hydrogen atom, a hydroxy group, an acyl group or a monovalent group represented by —CH<sub>2</sub>—OR<sup>1</sup>; at least one of R<sup>11</sup> to R<sup>26</sup>, at least one of R<sup>22</sup> to R<sup>25</sup>, at least one of R<sup>31</sup> to R<sup>34</sup>, at least one of R<sup>41</sup> to R<sup>44</sup>, and at least one of R<sup>51</sup> to R<sup>54</sup> are a monovalent group represented by —CH<sub>2</sub>—OR<sup>1</sup>; R<sup>1</sup> represents a hydrogen atom or an alkyl group having 1 to 10 carbon atoms; the alkyl group can be a methyl group, an ethyl group, a propyl group (n-propyl group, iso-propyl group) or a butyl group (n-butyl group, iso-butyl group, tert-butyl group) from

83

the viewpoint of the polymerizability; R<sup>21</sup> represents an aryl group, an alkyl group-substituted aryl group, a cycloalkyl group or an alkyl group-substituted cycloalkyl group.

Hereinafter, specific examples of compounds represented by one of formulae (C1) to (C5) will be described. Oligomers (multimers) of compounds represented by one of formulae (C1) to (C5) may be contained. Compounds (monomers) represented by one of formulae (C1) to (C5) can be contained in 10% by mass or more in the total mass of the amine compounds from the viewpoint of providing a uniform layer of a polymer. The degree of polymerization of the above-mentioned multimer can be 2 or more and 100 or less. The above-mentioned multimer and monomer may be used as a mixture of two or more.

Examples of compounds represented by the above formula (C1) usually commercially available include Supermelami No. 90 (made by NOF Corp.), Superbekamine(R) TD-139-60, L-105-60, L127-60, L110-60, J-820-60 and G-821-(made by DIC Corporation), Yuban 2020 (made by Mitsui Chemicals Inc.), Sumitex Resin M-3 (made by Sumitomo Chemical Co., Ltd.), and Nikalac MW-30, MW-390 and MX-750LM (Nihon Carbide Industries, Co., Inc.). Examples of compounds represented by the above formula (C2) usually commercially available include Superbekamine(R) L-148-55, 13-535, L-145-60 and TD-126 (made by Dainippon Ink and Chemicals, Inc.), and Nikalac BL-60 and BX-4000 (Nihon Carbide Industries, Co., Inc.). Examples of compounds represented by the above formula (C3) usually commercially available include Nikalac MX-280 (Nihon Carbide Industries, Co., Inc.). Examples of compounds represented by the above formula (C4) usually commercially available include Nikalac MX-270 (Nihon Carbide Industries, Co., Inc.). Examples of compounds represented by the above formula (C5) usually commercially available include Nikalac MX-290 (Nihon Carbide Industries, Co., Inc.).

Hereinafter, specific examples of compounds of the formula (C1) will be described.



84  
-continued

(C1-4)



(C1-5)



(C1-6)



(C1-7)



(C1-8)



(C1-9)



**85**  
-continued

(C1-10)



5



10



(C1-11) 15

20



(C1-12)

30

Hereinafter, specific examples of compounds of the formula (C2) will be described.

40



(C2-1)

45



(C2-2)

60



65

**86**  
-continued

(C2-3)



(C2-4)



(C2-5)



(C2-7)



(C2-8)



**87**

-continued



(C2-9)

(C2-10)

(C2-11)

(C2-12)

(C2-13)

(C2-14)

(C2-15)

(C2-16)

(C2-17)

(C2-18)

**88**

-continued



(C2-14)

(C2-15)

(C2-16)

(C2-17)

(C2-18)

Hereinafter, specific examples of compounds of the formula (C3) will be described.

89



Hereinafter, specific examples of compounds of the formula (C4) will be described.

90  
-continued

(C3-1) 5 H<sub>3</sub>COH<sub>2</sub>C—N—C(=O)—C(=O)N—CH<sub>2</sub>OCH<sub>3</sub>

10

(C3-2) 15 n-Bu—OH<sub>2</sub>C—N—C(=O)—C(=O)N—CH<sub>2</sub>OCH<sub>3</sub>

(C3-3) 20 H<sub>3</sub>COH<sub>2</sub>C—N—C(=O)—C(=O)N—CH<sub>2</sub>O—n-Bu

25

(C3-4) 30 n-Bu—OH<sub>2</sub>C—N—C(=O)—C(=O)N—CH<sub>2</sub>O—n-Bu

35

(C3-5) 40 H<sub>3</sub>COH<sub>2</sub>C—N—C(=O)—N—H



(C3-6) 45 H<sub>3</sub>COH<sub>2</sub>C—N—C(=O)—C(=O)N—CH<sub>2</sub>OH

50

(C4-6) 55 H<sub>3</sub>COH<sub>2</sub>C—N—C(=O)—C(=O)N—CH<sub>2</sub>OH

(C4-1) 60 H<sub>3</sub>COH<sub>2</sub>C—N—C(=O)—C(=O)N—CH<sub>2</sub>OH

65

(C5-1) 65 H<sub>3</sub>COH<sub>2</sub>C—N—C(=O)—C(=O)N—CH<sub>2</sub>OH



Hereinafter, specific examples of compounds of the formula (C5) will be described.



91

-continued



## Resin

Then, the thermoplastic resin having polymerizable functional groups will be described. The thermoplastic resin having polymerizable functional groups can be a thermoplastic resin having a structural unit represented by the following formula (D).



In the formula (D),  $R^{61}$  represents a hydrogen atom or an alkyl group;  $Y^1$  represents a single bond, an alkylene group or

92

a phenylene group; and  $W^1$  represents a hydroxy group, a thiol group, an amino group, a carboxyl group or a methoxy group.

A resin (hereinafter, also referred to as a resin D) having a structural unit represented by the formula (D) can be obtained by polymerizing, for example, a monomer commercially available from Sigma-Aldrich Japan Co., Ltd. and Tokyo Chemical Industry Co., Ltd. and having a polymerizable functional group (a hydroxy group, a thiol group, an amino group, a carboxyl group and a methoxy group).

The resins are usually commercially available. Examples of resins commercially available include polyether polyol-based resins such as AQD-457 and AQD-473 made by Nippon Polyurethane Industry Co., Ltd., and Sunnix GP-400, GP-700 and the like made by Sanyo Chemical Industries, Ltd., polyester polyol-based resins such as Phthalkid W2343 made by Hitachi Chemical Co., Ltd., Watersol S-118 and CD-520 and Beckolite M-6402-50 and M-6201-401M made by DIC Corporation, Haridip WH-1188 made by Harima Chemicals Group, Inc. and ES3604, ES6538 and the like made by Japan UPICA Co., Ltd., polyacryl polyol-based resins such as Burnock WE-300 and WE-304 made by DIC Corporation, polyvinylalcohol-based resins such as Kuraray Poval PVA-203 made by Kuraray Co., Ltd., polyvinyl acetal-based resins such as BX-1, BM-1, KS-1 and KS-5 made by Sekisui Chemical Co., Ltd., polyamide-based resins such as Toresin FS-350 made by Nagase ChemteX Corp., carboxyl group-containing resins such as Aqualic made by Nippon Shokubai Co., Ltd. and Finelex SG2000 made by Namariichi Co., Ltd., polyamine resins such as Rackamide made by DIC Corporation, and polythiol resins such as QE-340M made by Toray Industries, Inc. Above all, polyvinyl acetal-based resins, polyester polyol-based resins and the like are more preferable from the viewpoint of the polymerizability and the uniformity of an electron transporting layer.

The weight-average molecular weight ( $M_w$ ) of a resin D can be in the range of 5,000 to 400,000, and is more preferably in the range of 5,000 to 300,000. Examples of a method for quantifying a polymerizable functional group in the resin include the titration of a carboxyl group using potassium hydroxide, the titration of an amino group using sodium nitrite, the titration of a hydroxy group using acetic anhydride and potassium hydroxide, the titration of a thiol group using 5,5'-dithiobis(2-nitrobenzoic acid), and a calibration curve method using IR spectra of samples in which the incorporation ratio of a polymerizable functional group is varied.

In Table 10 hereinafter, specific examples of the resin D will be described.

TABLE 10

| R61 | Y | W           | Structure           | Mol Number per 1 g | Molecular  |                 |
|-----|---|-------------|---------------------|--------------------|------------|-----------------|
|     |   |             | of Functional Group | Another Site       | Weight     |                 |
| D1  | H | single bond | OH                  | 3.3 mmol           | butyral    | $1 \times 10^5$ |
| D2  | H | single bond | OH                  | 3.3 mmol           | butyral    | $4 \times 10^4$ |
| D3  | H | single bond | OH                  | 3.3 mmol           | butyral    | $2 \times 10^4$ |
| D4  | H | single bond | OH                  | 1.0 mmol           | polyolefin | $1 \times 10^5$ |
| D5  | H | single bond | OH                  | 3.0 mmol           | ester      | $8 \times 10^4$ |
| D6  | H | single bond | OH                  | 2.5 mmol           | Polyether  | $5 \times 10^4$ |
| D7  | H | single bond | OH                  | 2.8 mmol           | cellulose  | $3 \times 10^4$ |
| D8  | H | single bond | COOH                | 3.5 mmol           | polyolefin | $6 \times 10^4$ |
| D9  | H | single bond | NH <sub>2</sub>     | 1.2 mmol           | Polyamide  | $2 \times 10^5$ |
| D10 | H | single bond | SH                  | 1.3 mmol           | Polyolefin | $9 \times 10^3$ |
| D11 | H | phenylene   | OH                  | 2.8 mmol           | Polyolefin | $4 \times 10^3$ |
| D12 | H | single bond | OH                  | 3.0 mmol           | butyral    | $7 \times 10^4$ |
| D13 | H | single bond | OH                  | 2.9 mmol           | Polyester  | $2 \times 10^4$ |
| D14 | H | single bond | OH                  | 2.5 mmol           | Polyester  | $6 \times 10^3$ |
| D15 | H | single bond | OH                  | 2.7 mmol           | Polyester  | $8 \times 10^4$ |

TABLE 10-continued

| Structure |                               |             | Mol Number per 1 g  |              | Molecular  |                   |
|-----------|-------------------------------|-------------|---------------------|--------------|------------|-------------------|
| R61       | Y                             | W           | of Functional Group | Another Site | Weight     |                   |
| D16       | H                             | single bond | COOH                | 1.4 mmol     | polyolefin | $2 \times 10^5$   |
| D17       | H                             | single bond | COOH                | 2.2 mmol     | polyester  | $9 \times 10^3$   |
| D18       | H                             | single bond | COOH                | 2.8 mmol     | polyester  | $8 \times 10^2$   |
| D19       | CH <sub>3</sub>               | alkylene    | OH                  | 1.5 mmol     | polyester  | $2 \times 10^4$   |
| D20       | C <sub>2</sub> H <sub>5</sub> | alkylene    | OH                  | 2.1 mmol     | polyester  | $1 \times 10^4$   |
| D21       | C <sub>2</sub> H <sub>5</sub> | alkylene    | OH                  | 3.0 mmol     | polyester  | $5 \times 10^4$   |
| D22       | H                             | single bond | OCH <sub>3</sub>    | 2.8 mmol     | polyolefin | $7 \times 10^3$   |
| D23       | H                             | single bond | OH                  | 3.3 mmol     | butyral    | $2.7 \times 10^5$ |
| D24       | H                             | single bond | OH                  | 3.3 mmol     | butyral    | $4 \times 10^5$   |
| D25       | H                             | single bond | OH                  | 2.5 mmol     | acetal     | $4 \times 10^5$   |

15

An electron transporting substance having polymerizable functional groups can be 30% by mass or more and 70% by mass or less with respect to the total mass of a composition including the electron transporting substance having polymerizable functional groups, a crosslinking agent and a resin having polymerizable functional groups.

#### Conductive Support

As an conductive support (also referred to as a support), for example, supports made of a metal or an alloy of aluminum, nickel, copper, gold, iron or the like can be used. The support includes supports in which a metal thin film of aluminum, silver, gold or the like is formed on an insulating support of a polyester resin, a polycarbonate resin, a polyimide resin, a glass or the like, and supports in which a conductive material thin film of indium oxide, tin oxide or the like is formed.

The surface of a support may be subjected to a treatment such as an electrochemical treatment such as anodic oxidation, a wet honing treatment, a blast treatment and a cutting treatment, in order to improve electric properties and suppress interference fringes.

A conductive layer may be provided between a support and an undercoating layer described later. The conductive layer is obtained by forming a coating film of a coating liquid for a conductive layer in which a conductive particle is dispersed in a resin, on the support, and drying the coating film. Examples of the conductive particle include carbon black, acetylene black, metal powders such as aluminum, nickel, iron, nichrome, copper, zinc and silver, and metal oxide powders such as conductive tin oxide and ITO.

Examples of the resin include polyester resins, polycarbonate resins, polyvinyl butyral resins, acrylic resins, silicone resin, epoxy resins, melamine resins, urethane resins, phenol resins and alkyd resins.

Examples of a solvent of a coating liquid for a conductive layer include etheric solvents, alcoholic solvents, ketonic solvents and aromatic hydrocarbon solvents. The thickness of a conductive layer can be 0.2  $\mu\text{m}$  or more and 40  $\mu\text{m}$  or less, is more preferably 1  $\mu\text{m}$  or more and 35  $\mu\text{m}$  or less, and still more preferably 5  $\mu\text{m}$  or more and 30  $\mu\text{m}$  or less.

#### Charge Generating Layer

A charge generating layer is provided on an undercoating layer (electron transporting layer).

A charge generating substance includes azo pigments, perylene pigments, anthraquinone derivatives, anthroanthrone derivatives, dibenzopyrenequinone derivatives, pyranthrone derivatives, violanthrone derivatives, isoviolanthrone derivatives, indigo derivatives, thioindigo derivatives, phthalocyanine pigments such as metal phthalocyanines and non-metal phthalocyanines, and bisbenzimidazole derivatives. Above all, at least one of azo pigments and phthalocyanine pigments can be used. Among phthalocyanine pigments, oxytitanium

phthalocyanine, chlorogallium phthalocyanine and hydroxygallium phthalocyanine can be used.

Examples of a binder resin used for a charge generating layer include polymers and copolymers of vinyl compounds such as styrene, vinyl acetate, vinyl chloride, acrylic ester, methacrylic ester, vinylidene fluoride and trifluoroethylene, polyvinyl alcohol resins, polyvinyl acetal resins, polycarbonate resins, polyester resins, polysulfone resins, polyphenylene oxide resins, polyurethane resins, cellulosic resins, phenol resins, melamine resins, silicon resins and epoxy resins. Above all, polyester resins, polycarbonate resins and polyvinyl acetal resins can be used, and polyvinyl acetal is more preferable.

In a charge generating layer, the ratio (charge generating substance/binder resin) of a charge generating substance and a binder resin can be in the range of 10/1 to 1/10, and is more preferably in the range of 5/1 to 1/5. A solvent used for a coating liquid for a charge generating layer includes alcoholic solvents, sulfoxide-based solvents, ketonic solvents, etheric solvents, esteric solvents and aromatic hydrocarbon solvents. The thickness of a charge generating layer can be 0.05  $\mu\text{m}$  or more and 5  $\mu\text{m}$  or less.

#### Hole Transporting Layer

A hole transporting layer is provided on a charge generating layer. Examples of a hole transporting substance include polycyclic aromatic compounds, heterocyclic compounds, hydrazone compounds, styryl compounds, benzidine compounds, and triarylamine compounds, triphenylamine, and polymers having a group derived from these compounds in the main chain or side chain. Above all, triarylamine compounds, benzidine compounds and styryl compounds can be used.

Examples of a binder resin used for a hole transporting layer include polyester resins, polycarbonate resins, polymethacrylic ester resins, polyarylate resins, polysulfone resins and polystyrene resins. Above all, polycarbonate resins and polyarylate resins can be used. With respect to the molecular weight thereof, the weight-average molecular weight (Mw) can be in the range of 10,000 to 300,000.

In a hole transporting layer, the ratio (hole transporting substance/binder resin) of a hole transporting substance and a binder resin can be 10/5 to 5/10, and is more preferably 10/8 to 6/10. The thickness of a hole transporting layer can be 3  $\mu\text{m}$  or more and 40  $\mu\text{m}$  or less. The thickness is more preferably 5  $\mu\text{m}$  or more and 16  $\mu\text{m}$  or less from the viewpoint of the thickness of the electron transporting layer. A solvent used for a coating liquid for a hole transporting layer includes alcoholic solvents, sulfoxide-based solvents, ketonic solvents, etheric solvents, esteric solvents and aromatic hydrocarbon solvents.

Another layer such as a second undercoating layer which does not contain a polymer according to the present invention may be provided between a support and the electron transporting layer and between the electron transporting layer and a charge generating layer.

A surface protecting layer may be provided on a hole transporting layer. The surface protecting layer contains a conductive particle or a charge transporting substance and a binder resin. The surface protecting layer may further contain additives such as a lubricant. The binder resin itself of the protecting layer may have conductivity and charge transportability; in this case, the protecting layer does not need to contain a conductive particle and a charge transporting substance other than the binder resin. The binder resin of the protecting layer may be a thermoplastic resin, and may be a curable resin capable of being polymerized by heat, light, radiation (electron beams) or the like.

A method for forming each layer such as an electron transporting layer, a charge generating layer and a hole transporting layer constituting an electrophotographic photosensitive member can be a method in which a coating liquid obtained by dissolving and/or dispersing a material constituting the each layer in a solvent is applied, and the obtained coating film is dried and/or cured. Examples of a method of applying the coating liquid include an immersion coating method, a spray coating method, a curtain coating method and a spin coating method. Above all, an immersion coating method can be used from the viewpoint of efficiency and productivity.

#### Process Cartridge and Electrophotographic Apparatus

FIG. 3 illustrates an outline constitution of an electrophotographic apparatus having a process cartridge having an electrophotographic photosensitive member.

In FIG. 3, reference numeral 1 denotes a cylindrical electrophotographic photosensitive member, which is rotationally driven at a predetermined peripheral speed in the arrow direction around a shaft 2 as a center. A surface (peripheral surface) of the rotationally driven electrophotographic photosensitive member 1 is uniformly charged at a predetermined positive or negative potential by a charging unit 3 (primary charging unit: charging roller or the like). Then, the surface is subjected to irradiation light (image-exposure light) 4 from a light irradiation unit (exposure unit, not illustrated) such as slit light irradiation or laser beam scanning light irradiation. Electrostatic latent images corresponding to objective images are successively formed on the surface of the electrophotographic photosensitive member 1 in such a manner.

The electrostatic latent images formed on the surface of the electrophotographic photosensitive member 1 are developed with a toner contained in a developer of a developing unit 5 to thereby make toner images. Then, the toner images formed and carried on the surface of the electrophotographic photosensitive member 1 are successively transferred to a transfer material (paper or the like) P by a transferring bias from a transfer unit (transfer roller or the like) 6. The transfer material P is delivered from a transfer material feed unit (not illustrated) and fed to between the electrophotographic photosensitive member 1 and the transfer unit 6 (to a contacting part) synchronously with the rotation of the electrophotographic photosensitive member 1.

The transfer material P having the transferred toner images is separated from the surface of the electrophotographic photosensitive member 1, introduced to a fixing unit 8 to be subjected to image fixation, and printed out as an image-formed matter (print, copy) outside the apparatus.

The surface of the electrophotographic photosensitive member 1 after the toner image transfer is subjected to removal of the untransferred developer (toner) by a cleaning

unit (cleaning blade or the like) 7 to be thereby cleaned. Then, the surface is subjected to a charge-neutralizing treatment with irradiation light (not illustrated) from a light irradiation unit (exposure unit, not illustrated), and thereafter used repeatedly for image formation. As illustrated in FIG. 3, in the case where the charging unit 3 is a contacting charging unit using a charging roller or the like, the light irradiation is not necessarily needed.

A plurality of some constituting elements out of constituting elements including the electrophotographic photosensitive member 1, the charging unit 3, the developing unit 5, the transfer unit 6 and the cleaning unit 7 described above may be selected and accommodated in a container and integrally constituted as a process cartridge; and the process cartridge 15 may be constituted detachably from an electrophotographic apparatus body of a copying machine, a laser beam printer or the like. In FIG. 3, the electrophotographic photosensitive member 1, the charging unit 3, the developing unit 5 and the cleaning unit 7 are integrally supported and made as a cartridge 20 to thereby make a process cartridge 9 attachable to and detachable from an electrophotographic apparatus body by using a guiding unit 10 such as rails of the electrophotographic apparatus body.

#### EXAMPLES

Then, the manufacture and evaluation of electrophotographic photosensitive members will be described. "Parts" in Examples indicate "parts by mass."

##### Example 1

An aluminum cylinder (JIS-A3003, an aluminum alloy) of 260.5 mm in length and 30 mm in diameter was made to be a support (conductive support).

Then, 50 parts of a titanium oxide particle coated with an oxygen-deficient tin oxide (powder resistivity: 120  $\Omega\cdot\text{cm}$ , coverage factor of tin oxide: 40%), 40 parts of a phenol resin (Plyophen J-325, made by DIC Corporation, resin solid content: 60%), and 50 parts of methoxypropanol as a solvent (dispersion solvent) were placed in a sand mill using a glass bead of 0.8 mm in diameter, and subjected to a dispersion treatment for 3 hours to thereby prepare a dispersion liquid. After the dispersion, 0.01 part of a silicone oil SH28PA (made by Dow Corning Toray Co., Ltd.) and a silicone microparticle (Tospearl 120CA) as an organic resin particle were added to the dispersion liquid, and stirred to thereby prepare a coating liquid for a conductive layer. The content of the silicone microparticle was a sum of the solid content thereof and 5% by mass of (the total mass of the titanium oxide particle and the phenol resin). The coating liquid for a conductive layer was immersion coated on the support, and the obtained coating film was dried and heat polymerized for 30 min at 150°C. to thereby form a conductive layer having a thickness of 16  $\mu\text{m}$ .

The average particle diameter of the titanium oxide particle coated with an oxygen-deficient tin oxide in the coating liquid for a conductive layer was measured by a centrifugal precipitation method using tetrahydrofuran as a dispersion medium at a rotation frequency of 5,000 rpm by using a particle size distribution analyzer (trade name: CAPA700) made by HORIBA Ltd. As a result, the average particle diameter was 0.31  $\mu\text{m}$ .

Then, 4 parts of the electron transporting substance (A101), 7.3 parts of the crosslinking agent (B1: blocking group (H1)=5.1:2.2 (mass ratio)), 0.9 part of the resin (D1) and 0.05 part of dioctyltin laurate as a catalyst were dissolved

in a mixed solvent of 100 parts of dimethylacetamide and 100 parts of methyl ethyl ketone to thereby prepare a coating liquid for an electron transporting layer. The coating liquid for an electron transporting layer was immersion coated on the conductive layer, and the obtained coating film was heated for 40 min at 160° C. to be polymerized to thereby form an electron transporting layer (undercoating layer) having a thickness of 0.53  $\mu$ m.

The content of the electron transporting substance with respect to the total mass of the electron transporting substance, the crosslinking agent and the resin was 33% by mass.

Then, 10 parts of a hydroxylgallium phthalocyanine crystal (charge generating substance) having a crystal form exhibiting strong peaks at Bragg angles ( $20\pm0.2^\circ$ ) of  $7.5^\circ$ ,  $9.9^\circ$ ,  $12.5^\circ$ ,  $16.3^\circ$ ,  $18.6^\circ$ ,  $25.1^\circ$  and  $28.3^\circ$  in CuK $\alpha$  characteristic X-ray diffractometry, 0.1 part of a compound represented by the following formula (17), 5 parts of a polyvinyl butyral resin (trade name: Eslec BX-1, made by Sekisui Chemical Co., Ltd.) and 250 parts of cyclohexanone were placed in a sand mill using a glass bead of 0.8 mm in diameter, and subjected to a dispersion treatment for 1.5 hours. Then, 250 parts of ethyl acetate was added thereto to thereby prepare a coating liquid for a charge generating layer.



(9-1)



(9-2)



The coating liquid for a charge generating layer was immersion coated on the electron transporting layer, and the obtained coating film was dried for 10 min at 100° C. to thereby form a charge generating layer having a thickness of 0.15  $\mu\text{m}$ . A laminated body having the conductive support, the conductive layer, the electron transporting layer, and the charge generating layer was formed in such a manner.

Then, 4 parts of each of a triarylamine compound represented by the following formula (9-1) and a benzidine compound represented by the following formula (9-2) and 10 parts of a polyarylate resin having a repeating structural unit represented by the following formula (10-1) and a repeating structural unit represented by the following formula (10-2) in a proportion of 5/5, and having a weight-average molecular weight (Mw) of 100,000 were dissolved in a mixed solvent of 40 parts of dimethoxymethane and 60 parts of chlorobenzene to thereby prepare a coating liquid for a hole transporting layer. The coating liquid for a hole transporting layer was immersion coated on the charge generating layer, and the obtained coating film was dried for 40 min at 120° C. to thereby form a hole transporting layer having a thickness of 15  $\mu$ m.

98

5

10

20

45

14

13

-continued

(10-1)



1



(10-2)

In such a manner, an electrophotographic photosensitive member having the laminated body and the hole transporting layer for evaluating the positive ghost was manufactured. Further as in the above, one more electrophotographic photosensitive member was manufactured, and made as an electrophotographic photosensitive member for determination.

## (Determination Test)

The electrophotographic photosensitive member for determination described above was immersed for 5 min under the application of an ultrasonic wave in a mixed solvent of 40 parts of dimethoxymethane and 60 parts of chlorobenzene to peel the hole transporting layer, and thereafter, the resultant was dried for 10 min at 100° C. to thereby fabricate a laminated body having the support, the electron transporting layer and the charge generating layer, and the laminated body was made as an electrophotographic photosensitive member for determination. The surface thereof was confirmed to have no components of the hole transporting layer by using an FTIR-ATR method.

Then, a measurement portion was cut out in 2 cm (peripheral direction of the electrophotographic photosensitive member)×4 cm (long axis direction thereof) from the electrophotographic photosensitive member for determination, and a circular-shaped gold electrode having a thickness of 300 nm and a diameter of 10 mm was fabricated on the charge generating layer by the above-mentioned sputtering.

Then, the electrophotographic photosensitive member for determination was allowed to stand for 24 hours in an environment of a temperature of 25° C. and a humidity of 50% RH, and thereafter, a sample was fabricated which was constituted of the support, the conductive layer, the electron transporting layer, the charge generating layer and the gold electrode with the above-mentioned determination method. First, the whole sample was covered with a blackout film; and the impedance ( $R_{dark}$ ) when an alternating electric field of 100 mV and 0.1 Hz was applied between the conductive support and the gold electrode was measured by sweeping the frequency from 1 MHz to 0.1 Hz and under the condition of no light irradiation of the surface of the charge generating layer. The impedance ( $R_{opt}$ ) when an alternating electric field of 100 mV and 0.1 Hz was applied between the conductive support and the gold electrode was further measured under the condition that the surface of the charge generating layer was irradiated with light having an irradiation intensity of 30  $\mu$ J/cm<sup>2</sup>·sec in the state that laser light having a wavelength of 680 nm was oscillated and the charge generating layer and the gold electrode side of the sample were irradiated with the light so that the irradiation intensity became 30  $\mu$ J/cm<sup>2</sup>·sec.  $R_{opt}/R_{dark}$  was calculated from the acquired  $R_{dark}$  and  $R_{opt}$ . The measurement results are shown in Table 11.

## (Evaluation of the Positive Ghost)

The manufactured electrophotographic photosensitive member for evaluating the positive ghost was mounted on a remodeled machine (primary charging: roller contacting DC charging, process speed: 120 mm/sec, laser light irradiation), a power source of whose pre-light irradiation unit was cut off, of a laser beam printer (trade name: LBP-2510) made by Canon Corp., and the evaluations of the early-stage printed-out image (early-stage ghost) and the positive ghost in the repeated use were carried out. Details are as follows.

## 1. Early-Stage Ghost

A process cartridge for a cyan color of the laser beam printer was remodeled, and a potential probe (model: 6000B-8, made by Trek Japan KK) was mounted on a development position; and the manufactured electrophotographic photosensitive member was mounted, and the potential of the center portion of the electrophotographic photosensitive member was measured under an environment of a temperature of 23° C. and a humidity of 50% RH by using a surface electrometer (model: 344, made by Trek Japan KK). The charging voltage and the irradiation light intensity were adjusted so that the dark area potential ( $V_d$ ) of the surface potential of the elec-

trophotographic photosensitive member became -600 V and the light area potential ( $V_l$ ) thereof became -200 V.

Then, the electrophotographic photosensitive member was mounted on the process cartridge for a cyan color of the laser beam printer, and the process cartridge was mounted on a process cartridge station for cyan, and images were printed out. Images were continuously printed out in the order of one sheet of a solid white image, 5 sheets of an image for ghost evaluation, one sheet of a solid black image and 5 sheets of an image for ghost evaluation.

The image for ghost evaluation, as illustrated in FIG. 4, had a "white image" printed out in the lead part thereof in which square "solid images" were printed, and had a "halftone image of a one-dot keima pattern" illustrated in FIG. 5A, fabricated after the lead part. In FIG. 4, "ghost" parts were parts where ghosts caused by the "solid images" may have emerged.

The evaluation of the positive ghost was carried out by measuring the density difference between the image density of the halftone image of a one-dot keima pattern described above and the image density of a ghost part. 10 points of the density differences were measured in one sheet of an image for ghost evaluation by a spectrodensitometer (trade name: X-Rite 504/508, made by X-Rite Inc.). This operation was carried out for all of 10 sheets of the image for ghost evaluation, and the average of 100 points in total was calculated. The results are shown in Table 11. It is found that a higher density of a ghost part caused a stronger positive ghost. It is meant that a smaller Macbeth density difference more suppressed the positive ghost. A ghost image density difference (Macbeth density difference) of 0.05 or more gave a level thereof having a visually obvious difference, and a ghost image density difference of less than 0.05 gave a level thereof having no visually obvious difference.

## 2. Long-Term Ghost

Continuous 1,000-sheets image printing-out was carried out using halftone images of a one-dot pattern illustrated in FIG. 5B described above with the adjusted charging voltage and the adjusted irradiation light intensity being fixed to those determined in the evaluation of "1. Early-stage ghost" described above. Within 2 min after the image printing-out of 1,000th sheet, image printing-out was carried out as illustrated in FIG. 4 as in the case of the early-stage ghost, and the positive ghost evaluation (image density evaluation using a spectrodensitometer) after the 1,000-sheets image printing-out was carried out. The results are shown in Table 11.

## Examples 2 to 5

Electrophotographic photosensitive members were manufactured and evaluated as in Example 1, except for altering the thickness of an electron transporting layer from 0.53  $\mu$ m to 0.38  $\mu$ m (Examples 2), 0.25  $\mu$ m (Examples 3), 0.20  $\mu$ m (Examples 4) and 0.15  $\mu$ m (Examples 5) as shown in Table 11.

The results are shown in Table 11.

## Example 6

An electrophotographic photosensitive member was manufactured and evaluated as in Example 1, except for forming an electron transporting layer as follows. The results are shown in Table 11.

4 parts of the electron transporting substance (A101), 5.5 parts of the isocyanate compound (B1: blocking group (H1)=5.1:2.2 (mass ratio)), 0.3 part of the resin (D1) and 0.05 part of dioctyltin laurate as a catalyst were dissolved in a mixed solvent of 100 parts of dimethylacetamide and 100 parts of

**101**

methyl ethyl ketone to thereby prepare a coating liquid for an electron transporting layer. The coating liquid for an electron transporting layer was immersion coated on the conductive layer, and the obtained coating film was heated for 40 min at 160° C. to be polymerized to thereby form an electron transporting layer having a thickness of 0.61  $\mu\text{m}$ .

## Examples 7 to 12

Electrophotographic photosensitive members were manufactured and evaluated as in Example 6, except for altering the thickness of the electron transporting layer from 0.61  $\mu\text{m}$  to those shown in Table 11. The results are shown in Table 11.

## Example 13

An electrophotographic photosensitive member was manufactured and evaluated as in Example 1, except for forming an electron transporting layer as follows. The results are shown in Table 11.

5 parts of the electron transporting substance (A-101), 2.3 parts of the amine compound (C<sub>1</sub>-3), 3.3 parts of the resin (D1) and 0.1 part of dodecylbenzenesulfonic acid as a catalyst were dissolved in a mixed solvent of 100 parts of dimethyl-lacetoamide and 100 parts of methyl ethyl ketone to thereby prepare a coating liquid for an electron transporting layer. The coating liquid for an electron transporting layer was immersion coated on the conductive layer, and the obtained coating film was heated for 40 min at 160° C. to be polymerized to thereby form an electron transporting layer having a thickness of 0.51  $\mu\text{m}$ .

## Examples 14 to 17

Electrophotographic photosensitive members were manufactured and evaluated as in Example 13, except for altering the thickness of the electron transporting layer from 0.51  $\mu\text{m}$  to those shown in Table 11. The results are shown in Table 11.

## Example 18

An electrophotographic photosensitive member was manufactured and evaluated as in Example 1, except for forming an electron transporting layer as follows. The results are shown in Table 11.

5 parts of the electron transporting substance (A-101), 1.75 parts of the amine compound (C<sub>1</sub>-3), 2 parts of the resin (D1) and 0.1 part of dodecylbenzenesulfonic acid as a catalyst were dissolved in a mixed solvent of 100 parts of dimethyl-lacetoamide and 100 parts of methyl ethyl ketone to thereby prepare a coating liquid for an electron transporting layer. The coating liquid for an electron transporting layer was immersion coated on the conductive layer, and the obtained coating film was heated for 40 min at 160° C. to be polymerized to thereby form an electron transporting layer having a thickness of 0.70  $\mu\text{m}$ .

## Examples 19 to 24

Electrophotographic photosensitive members were manufactured and evaluated as in Example 18, except for altering the thickness of the electron transporting layer from 0.70  $\mu\text{m}$  to those shown in Table 11. The results are shown in Table 11.

## Examples 25 to 45

Electrophotographic photosensitive members were manufactured and evaluated as in Example 6, except for altering the

**102**

electron transporting substance of Example 6 from (A-101) to electron transporting substances shown in Table 11, and altering the thickness of the electron transporting layer to those shown in Table 11. The results are shown in Table 11.

## Examples 46 to 66

Electrophotographic photosensitive members were manufactured and evaluated as in Example 18, except for altering the electron transporting substance of Example 18 from (A-101) to electron transporting substances shown in Table 11, and altering the thickness of the electron transporting layer to those shown in Table 11. The results are shown in Table 11.

## Examples 67 to 72

Electrophotographic photosensitive members were manufactured and evaluated as in Example 8, except for altering the crosslinking agent (B1: blocking group (H1)=5.1:2.2 (mass ratio)) of Example 8 to crosslinking agents shown in Table 11. The results are shown in Tables 11 and 12.

## Examples 73 and 74

Electrophotographic photosensitive members were manufactured and evaluated as in Example 21, except for altering the crosslinking agent (C<sub>1</sub>-3) of Example 21 to crosslinking agents shown in Table 11. The results are shown in Table 12.

## Example 75

An electrophotographic photosensitive member was manufactured and evaluated as in Example 1, except for forming an electron transporting layer as follows. The results are shown in Table 12.

4 parts of the electron transporting substance (A-101), 4 parts of the amine compound (C<sub>1</sub>-9), 1.5 parts of the resin (D1) and 0.2 part of dodecylbenzenesulfonic acid as a catalyst were dissolved in a mixed solvent of 100 parts of dimethyl-lacetoamide and 100 parts of methyl ethyl ketone to thereby prepare a coating liquid for an electron transporting layer. The coating liquid for an electron transporting layer was immersion coated on the conductive layer, and the obtained coating film was heated for 40 min at 160° C. to be polymerized to thereby form an electron transporting layer having a thickness of 0.35  $\mu\text{m}$ .

## Examples 76 and 77

Electrophotographic photosensitive members were manufactured and evaluated as in Example 75, except for altering the crosslinking agent (C<sub>1</sub>-9) of Example 75 to crosslinking agents shown in Table 12. The results are shown in Table 12.

## Examples 78 to 81

Electrophotographic photosensitive members were manufactured and evaluated as in Example 9, except for altering the resin (D1) of Example 9 to resins shown in Table 12. The results are shown in Table 12.

## Example 82

An electrophotographic photosensitive member was manufactured and evaluated as in Example 1, except for forming an electron transporting layer as follows. The results are shown in Table 12.

## 103

6 parts of the electron transporting substance (A-124), 2.1 parts of the amine compound (C<sub>1</sub>-3), 1.2 parts of the resin (D1) and 0.1 part of dodecylbenzenesulfonic acid as a catalyst were dissolved in a mixed solvent of 100 parts of dimethyl-lacetoamide and 100 parts of methyl ethyl ketone to thereby prepare a coating liquid for an electron transporting layer. The coating liquid for an electron transporting layer was immersion coated on the conductive layer, and the obtained coating film was heated for 40 min at 160° C. to be polymerized to thereby form an electron transporting layer having a thickness of 0.45 μm.

## Examples 83 and 84

Electrophotographic photosensitive members were manufactured and evaluated as in Example 82, except for altering the electron transporting substance of Example 82 from (A-124) to electron transporting substances shown in Table 12. The results are shown in Table 12.

## Example 85

An electrophotographic photosensitive member was manufactured and evaluated as in Example 1, except for forming an electron transporting layer as follows. The results are shown in Table 12.

6 parts of the electron transporting substance (A-125), 2.1 parts of the amine compound (C<sub>1</sub>-3), 0.5 part of the resin (D1) and 0.1 part of dodecylbenzenesulfonic acid as a catalyst were dissolved in a mixed solvent of 100 parts of dimethyl-lacetoamide and 100 parts of methyl ethyl ketone to thereby prepare a coating liquid for an electron transporting layer. The coating liquid for an electron transporting layer was immersion coated on the conductive layer, and the obtained coating film was heated for 40 min at 160° C. to thereby form an electron transporting layer having a thickness of 0.49 μm.

## Example 86

An electrophotographic photosensitive member was manufactured and evaluated as in Example 1, except for forming an electron transporting layer as follows. The results are shown in Table 12.

6.5 parts of the electron transporting substance (A-125), 2.1 parts of the amine compound (C<sub>1</sub>-3), 0.4 part of the resin (D1) and 0.1 part of dodecylbenzenesulfonic acid as a catalyst were dissolved in a mixed solvent of 100 parts of dimethyl-lacetoamide and 100 parts of methyl ethyl ketone to thereby prepare a coating liquid for an electron transporting layer. The coating liquid for an electron transporting layer was immersion coated on the conductive layer, and the obtained coating film was heated for 40 min at 160° C. to be polymerized to thereby form an electron transporting layer having a thickness of 0.49 μm.

## Example 87 to 89

An electrophotographic photosensitive member was manufactured and evaluated as in Example 85, except for altering the thickness of the electron transporting layer from 0.49 μm to those shown in Table 12. The results are shown in Table 12.

## Example 90

An electrophotographic photosensitive member was manufactured and evaluated as in Example 1, except for forming an electron transporting layer as follows. The results are shown in Table 12.

## 104

3.6 parts of the electron transporting substance (A101), 7 parts of the isocyanate compound (B1: blocking group (H1)=5.1:2.2 (mass ratio)), 1.3 parts of the resin (D1) and 0.05 part of dioctyltin laurate as a catalyst were dissolved in a mixed solvent of 100 parts of dimethyl-lacetoamide and 100 parts of methyl ethyl ketone to thereby prepare a coating liquid for an electron transporting layer. The coating liquid for an electron transporting layer was immersion coated on the conductive layer, and the obtained coating film was heated for 40 min at 160° C. to be polymerized to thereby form an electron transporting layer having a thickness of 0.53 μm.

## Example 91

An electrophotographic photosensitive member was manufactured and evaluated as in Example 1, except for altering the thickness of the charge generating layer from 0.53 μm to 0.15 μm. The results are shown in Table 12.

## Example 92

An electrophotographic photosensitive member was manufactured and evaluated as in Example 1, except for forming a charge generating layer as follows. The results are shown in Table 12.

10 parts of oxytitanium phthalocyanine exhibiting strong peaks at Bragg angles (20±0.2°) of 9.0°, 14.2°, 23.9° and 27.1° in CuK $\alpha$  X-ray diffractometry was used, and 166 parts of a solution was prepared in which a polyvinyl butyral resin (trade name: Eslec BX-1, made by Sekisui Chemical Co., Ltd.) was dissolved in a mixed solvent of cyclohexanone:water=97:3 to make a 5% by mass solution. The solution and 150 parts of the mixed solvent of cyclohexanone:water=97:3 were together dispersed for 4 hours in a sand mill apparatus using 400 parts of a glass bead of 1 mmφ, and thereafter, 210 parts of the mixed solvent of cyclohexanone:water=97:3 and 260 parts of cyclohexanone were added thereto to thereby prepare a coating liquid for a charge generating layer. The coating liquid for a charge generating layer was immersion coated on the electron transporting layer, and the obtained coating film was dried for 10 min at 80° C. to thereby form a charge generating layer having a thickness of 0.20 μm.

## Example 93

An electrophotographic photosensitive member was manufactured and evaluated as in Example 1, except for forming charge generating layer as follows. The results are shown in Table 12.

20 parts of a bisazo pigment represented by the following structural formula (II) and 10 parts of a polyvinyl butyral resin (trade name: Eslec BX-1, made by Sekisui Chemical Co., Ltd.) were mixed and dispersed in 150 parts of tetrahydrofuran to thereby prepare a coating liquid for a charge generating layer. Then, the coating liquid was immersion coated on the electron transporting layer, and the obtained coating film was dried at 110° C. for 30 min to thereby form a charge generating layer having a thickness of 0.30 μm.

105



106



## Example 94

An electrophotographic photosensitive member was manufactured and evaluated as in Example 1, except for altering the benzidine compound represented by the above formula (9-2) of Example 1 to a styryl compound (hole transporting substance) represented by the following formula (9-3). The results are shown in Table 13.



## Examples 95 and 96

Electrophotographic photosensitive members were manufactured and evaluated as in Example 1, except for altering the thickness of the hole transporting layer from 15  $\mu\text{m}$  to 10  $\mu\text{m}$  (Example 95) and 25  $\mu\text{m}$  (Example 96). The results are shown in Table 13.

## Example 97

An aluminum cylinder (JIS-A3003, an aluminum alloy) of 260.5 mm in length and 30 mm in diameter was made to be a support (conductive support).

Then, 214 parts of a titanium oxide ( $\text{TiO}_2$ ) particle coated with an oxygen-deficient tin oxide ( $\text{SnO}_2$ ) as a metal oxide particle, 132 parts of a phenol resin (trade name: Plyophen J-325) as a binder resin, and 98 parts of 1-methoxy-2-propanol as a solvent were placed in a sand mill using 450 parts of a glass bead of 0.8 mm in diameter, and subjected to a dispersion treatment under the conditions of a rotation frequency of 2,000 rpm, a dispersion treatment time of 4.5 hours

and a set temperature of a cooling water of 18° C. to thereby obtain a dispersion liquid. The glass bead was removed from the dispersion liquid by a mesh (mesh opening: 150  $\mu\text{m}$ ). A silicone resin particle (trade name: Tospearl 120, made by Momentive Performance Materials Inc., average particle diameter: 2  $\mu\text{m}$ ) as a surface-roughening material was added to the dispersion liquid after the removal of the glass bead so as to become 10% by mass with respect to the total mass of the metal oxide particle and the binder resin in the dispersion liquid; and a silicone oil (trade name: SH28PA, made by Dow Corning Toray Co., Ltd.) as a leveling agent was added to the dispersion liquid so as to become 0.01% by mass with respect to the total mass of the metal oxide particle and the binder resin in the dispersion liquid; and the resultant mixture was stirred to thereby prepare a coating liquid for a conductive layer. The coating liquid for a conductive layer was immersion coated on a support, and the obtained coating film was dried and heat cured for 30 min at 150° C. to thereby form a conductive layer having a thickness of 30  $\mu\text{m}$ .

Then, 6.2 parts of the electron transporting substance (A157), 8.0 parts of the crosslinking agent (B1: blocking group (H5)=5.1:2.9 (mass ratio)), 1.1 parts of the resin (D25) and 0.05 part of zinc(II) hexanote as a catalyst were dissolved in a mixed solvent of 100 parts of dimethylacetamide and 100 parts of methyl ethyl ketone to thereby prepare a coating liquid for an electron transporting layer. The coating liquid for an electron transporting layer was immersion coated on the conductive layer, and the obtained coating film was heated for 40 min at 160° C. to be polymerized to thereby form an electron transporting layer (undercoating layer) having a thickness of 0.53  $\mu\text{m}$ . The content of the electron transporting substance with respect to the total mass of the electron transporting substance, the crosslinking agent and the resin was 34% by mass.

Then, a charge generating layer having a thickness of 0.15  $\mu\text{m}$  was formed as in Example 1.

9 parts of the triarylamine compound represented by the above structural formula (9-1), 1 part of a benzidine compound (hole transporting substance) represented by the following structural formula (18), 3 parts of a polyester resin E (weight-average molecular weight: 90,000) having a repeating structural unit represented by the following formula (24), and a repeating structural unit represented by the following formula (26) and a repeating structural unit represented by the following formula (25) in a ratio of 7:3, and 7 parts of a polyester resin F (weight-average molecular weight: 120,

107

000) having a repeating structural unit represented by the following formula (27) and a repeating structural unit represented by the following formula (28) in a ratio of 5: were dissolved in a mixed solvent of 30 parts of dimethoxymethane and 50 parts of orthoxylene to thereby prepare a coating liquid for a hole transporting layer. Here, the content of the repeating structural unit represented by the following formula (24) in the polyester resin E was 10% by mass, and the content of the repeating structural units represented by the following formulae (25) and (26) therein was 90% by mass.



(18)



(24)



(25)



(26)



(27)



(28)

The coating liquid for a hole transporting layer was immersion coated on the charge generating layer, and dried for 1 hour at 120° C. to thereby form a hole transporting layer having a thickness of 16 µm. The formed hole transporting layer was confirmed to have a domain structure in which a matrix containing the hole transporting substance and the polyester resin F contained the polyester resin E.

The evaluation was carried out as in Example 1. The results are shown in Table 13.

#### Example 98

An electrophotographic photosensitive member was manufactured as in Example 1, except for forming a hole transporting layer as follows. The results are shown in Table 13.

9 parts of the triarylamine compound represented by the above structural formula (9-1), 1 part of the benzidine com-

108

pound represented by the above structural formula (18), 10 parts of a polycarbonate resin G (weight-average molecular weight: 70,000) having a repeating structural unit represented by the following formula (29), and 0.3 part of a polycarbonate resin H (weight-average molecular weight: 40,000) having a repeating structural unit represented by the following formula (29), a repeating structural unit represented by the following formula (30) and a structure of at least one terminal represented by the following formula (31) were dissolved in a mixed solvent of 30 parts of dimethoxymethane and 50 parts



(29)

of orthoxylene to thereby prepare a coating liquid for a hole transporting layer. Here, the total mass of the structures represented by the following formulae (30) and (31) in the polycarbonate resin H was 30% by mass. The coating liquid for a hole transporting layer was immersion coated on the charge generating layer, and dried for 1 hour at 120° C. to thereby form a hole transporting layer having a thickness of 16 µm.

55

50

55

50

55

50

55

50

55

50

109

-continued

(30)



## Example 99

An electrophotographic photosensitive member was manufactured and evaluated as in Example 98, except for altering 10 parts of the polycarbonate resin G (weight-average molecular weight: 70,000) in the coating liquid for a hole transporting layer of Example 98 to 10 parts of the polyester resin F (weight-average molecular weight: 120,000). The results are shown in Table 13.

## Example 100

An electrophotographic photosensitive member was manufactured and evaluated as in Example 97, except for forming a conductive layer as follows. The results are shown in Table 13.

207 parts of a titanium oxide ( $TiO_2$ ) particle coated with a tin oxide ( $SnO_2$ ) doped with phosphorus (P) as a metal oxide particle, 144 parts of a phenol resin (trade name: Plyophen J-325) as a binder resin, and 98 parts of 1-methoxy-2-propanol as a solvent were placed in a sand mill using 450 parts of a glass bead of 0.8 mm in diameter, and subjected to a dispersion treatment under the conditions of a rotation frequency of 2,000 rpm, a dispersion treatment time of 4.5 hours and a set temperature of a cooling water of 18° C. to thereby obtain a dispersion liquid. The glass bead was removed from the dispersion liquid by a mesh (mesh opening: 150  $\mu m$ ).

A silicone resin particle (trade name: Tospearl 120) as a surface-roughening material was added to the dispersion liquid after the removal of the glass bead so as to become 15% by mass with respect to the total mass of the metal oxide particle and the binder resin in the dispersion liquid; and a silicone oil (trade name: SH28PA) as a leveling agent was added to the dispersion liquid so as to become 0.01% by mass with respect to the total mass of the metal oxide particle and the binder resin in the dispersion liquid; and the resultant mixture was stirred to thereby prepare a coating liquid for a conductive layer. The coating liquid for a conductive layer was immersion coated on a support, and the obtained coating film was dried and heat cured for 30 min at 150° C. to thereby form a conductive layer having a thickness of 30  $\mu m$ .

## Examples 101 to 119

Electrophotographic photosensitive members were manufactured and evaluated as in Example 97, except for altering the electron transporting substance of Example 97 from

110

(A157) to electron transporting substances shown in Table 13. The results are shown in Table 13.

## Comparative Example 1

An electrophotographic photosensitive member was manufactured and evaluated as in Example 1, except for forming an electron transporting layer as follows. The results are shown in Table 12.

2.4 parts of the electron transporting substance (A101), 4.2 parts of the isocyanate compound (B1: blocking group (H1)= 5.1:2.2 (mass ratio)), 5.4 parts of the resin (D1) and 0.05 part of dioctyltin laurate as a catalyst were dissolved in a mixed solvent of 100 parts of dimethylacetamide and 100 parts of methyl ethyl ketone to thereby prepare a coating liquid for an electron transporting layer. The coating liquid for an electron transporting layer was immersion coated on the conductive layer, and the obtained coating film was heated for 40 min at 160° C. to be polymerized to thereby form an electron transporting layer having a thickness of 0.53  $\mu m$ .

## Comparative Example 2

An electrophotographic photosensitive member was manufactured and evaluated as in Example 1, except for forming an electron transporting layer as follows. The results are shown in Table 12.

3.2 parts of the electron transporting substance (A101), 5 parts of the isocyanate compound (B1: blocking group (H1)= 5.1:2.2 (mass ratio)), 4.2 parts of the resin (D1) and 0.05 part of dioctyltin laurate as a catalyst were dissolved in a mixed solvent of 100 parts of dimethylacetamide and 100 parts of methyl ethyl ketone to thereby prepare a coating liquid for an electron transporting layer. The coating liquid for an electron transporting layer was immersion coated on the conductive layer, and the obtained coating film was heated for 40 min at 160° C. to be polymerized to thereby form an electron transporting layer having a thickness of 0.53  $\mu m$ .

## Comparative Examples 3 and 4

Electrophotographic photosensitive members were manufactured and evaluated as in Comparative Example 2, except for altering the thickness of the electron transporting layer from 0.53  $\mu m$  to 0.40  $\mu m$  and 0.32  $\mu m$ . The results are shown in Table 12.

## Comparative Examples 5 to 8

Electrophotographic photosensitive members were manufactured and evaluated as in Example 1, except for altering the thickness of the electron transporting layer from 0.53  $\mu m$  to 0.78  $\mu m$ , 1.03  $\mu m$ , 1.25  $\mu m$  and 1.48  $\mu m$ . The results are shown in Table 12.

## Comparative Example 9

An electrophotographic photosensitive member was manufactured and evaluated as in Example 1, except for forming an electron transporting layer as follows. The results are shown in Table 12.

4 parts of the electron transporting substance (A225), 3 parts of hexamethylene diisocyanate and 4 parts of the resin (D1) were dissolved in a mixed solvent of 100 parts of dimethylacetamide and 100 parts of methyl ethyl ketone to thereby prepare a coating liquid for an electron transporting layer. The coating liquid for an electron transporting layer

## 111

was immersion coated on the conductive layer, and the obtained coating film was heated for 40 min at 160° C. to be polymerized to thereby form an electron transporting layer having a thickness of 1.00  $\mu\text{m}$ .

## Comparative Example 10

An electrophotographic photosensitive member was manufactured and evaluated as in Example 1, except for forming an electron transporting layer as follows. The results are shown in Table 12.

5 parts of the electron transporting substance (A124), 2.5 parts of 2,4-toluene diisocyanate and 2.5 parts of a poly(p-hydroxystyrene) (trade name: Malkalinker, made by Maruzen Petrochemical Co., Ltd.) were dissolved in a mixed solvent of 100 parts of dimethylacetamide and 100 parts of methyl ethyl ketone to thereby prepare a coating liquid for an electron transporting layer. The coating liquid for an electron transporting layer was immersion coated on the conductive

layer, and the obtained coating film was heated for 40 min at 160° C. to be polymerized to thereby form an electron transporting layer having a thickness of 0.40  $\mu\text{m}$ .

5

## 112

## Comparative Example 11

An electrophotographic photosensitive member was manufactured and evaluated as in Example 1, except for forming an electron transporting layer as follows. The results are shown in Table 12.

7 parts of the electron transporting substance (A124), 2 parts of 2,4-toluene diisocyanate and 1 part of a poly(p-hydroxystyrene) were dissolved in a mixed solvent of 100 parts of dimethylacetamide and 100 parts of methyl ethyl ketone to thereby prepare a coating liquid for an electron transporting layer. The coating liquid for an electron transporting layer was immersion coated on the conductive layer, and the obtained coating film was heated for 40 min at 160° C. to be polymerized to thereby form an electron transporting layer having a thickness of 0.40  $\mu\text{m}$ .

TABLE 11

| Example | Electron Transporting Substance | Crosslinking Agent | Resin | Ratio of Electron Transporting Substance | Thickness of Undercoating Layer | R <sub>opt</sub> /R <sub>dark</sub> | Early-Stage Ghost | Ghost After 1,000 Sheets | Difference Between the Ghosts |
|---------|---------------------------------|--------------------|-------|------------------------------------------|---------------------------------|-------------------------------------|-------------------|--------------------------|-------------------------------|
| 1       | A101                            | B1:H1              | D1    | 33%                                      | 0.53                            | 0.85                                | 0.03              | 0.03                     | 0.00                          |
| 2       | A101                            | B1:H1              | D1    | 33%                                      | 0.38                            | 0.85                                | 0.03              | 0.03                     | 0.00                          |
| 3       | A101                            | B1:H1              | D1    | 33%                                      | 0.25                            | 0.85                                | 0.03              | 0.03                     | 0.00                          |
| 4       | A101                            | B1:H1              | D1    | 33%                                      | 0.20                            | 0.85                                | 0.03              | 0.03                     | 0.00                          |
| 5       | A101                            | B1:H1              | D1    | 33%                                      | 0.15                            | 0.95                                | 0.04              | 0.05                     | 0.01                          |
| 6       | A101                            | B1:H1              | D1    | 41%                                      | 0.61                            | 0.75                                | 0.02              | 0.02                     | 0.00                          |
| 7       | A101                            | B1:H1              | D1    | 41%                                      | 0.52                            | 0.75                                | 0.02              | 0.02                     | 0.00                          |
| 8       | A101                            | B1:H1              | D1    | 41%                                      | 0.40                            | 0.85                                | 0.03              | 0.03                     | 0.00                          |
| 9       | A101                            | B1:H1              | D1    | 41%                                      | 0.26                            | 0.85                                | 0.03              | 0.03                     | 0.00                          |
| 10      | A101                            | B1:H1              | D1    | 41%                                      | 0.70                            | 0.85                                | 0.03              | 0.03                     | 0.00                          |
| 11      | A101                            | B1:H1              | D1    | 41%                                      | 0.90                            | 0.90                                | 0.04              | 0.05                     | 0.01                          |
| 12      | A101                            | B1:H1              | D1    | 41%                                      | 1.10                            | 0.95                                | 0.04              | 0.05                     | 0.01                          |
| 13      | A101                            | C1-3               | D1    | 47%                                      | 0.51                            | 0.75                                | 0.02              | 0.02                     | 0.00                          |
| 14      | A101                            | C1-3               | D1    | 47%                                      | 0.45                            | 0.75                                | 0.01              | 0.01                     | 0.00                          |
| 15      | A101                            | C1-3               | D1    | 47%                                      | 0.34                            | 0.75                                | 0.02              | 0.02                     | 0.00                          |
| 16      | A101                            | C1-3               | D1    | 47%                                      | 0.70                            | 0.85                                | 0.02              | 0.02                     | 0.00                          |
| 17      | A101                            | C1-3               | D1    | 47%                                      | 0.91                            | 0.93                                | 0.03              | 0.04                     | 0.01                          |
| 18      | A101                            | C1-3               | D1    | 57%                                      | 0.70                            | 0.85                                | 0.03              | 0.03                     | 0.00                          |
| 19      | A101                            | C1-3               | D1    | 57%                                      | 0.58                            | 0.75                                | 0.02              | 0.02                     | 0.00                          |
| 20      | A101                            | C1-3               | D1    | 57%                                      | 0.50                            | 0.75                                | 0.02              | 0.02                     | 0.00                          |
| 21      | A101                            | C1-3               | D1    | 57%                                      | 0.35                            | 0.85                                | 0.03              | 0.03                     | 0.00                          |
| 22      | A101                            | C1-3               | D1    | 57%                                      | 0.92                            | 0.90                                | 0.03              | 0.04                     | 0.01                          |
| 23      | A101                            | C1-3               | D1    | 57%                                      | 1.11                            | 0.93                                | 0.03              | 0.04                     | 0.01                          |
| 24      | A101                            | C1-3               | D1    | 57%                                      | 1.32                            | 0.95                                | 0.04              | 0.05                     | 0.01                          |
| 25      | A106                            | B1:H1              | D1    | 41%                                      | 0.52                            | 0.75                                | 0.02              | 0.02                     | 0.00                          |
| 26      | A125                            | B1:H1              | D1    | 41%                                      | 0.52                            | 0.75                                | 0.02              | 0.02                     | 0.00                          |
| 27      | A125                            | B1:H1              | D1    | 41%                                      | 0.20                            | 0.75                                | 0.02              | 0.02                     | 0.00                          |
| 28      | A125                            | B1:H1              | D1    | 41%                                      | 0.70                            | 0.75                                | 0.02              | 0.02                     | 0.00                          |
| 29      | A136                            | B1:H1              | D1    | 41%                                      | 0.51                            | 0.75                                | 0.02              | 0.02                     | 0.00                          |
| 30      | A136                            | B1:H1              | D1    | 41%                                      | 0.21                            | 0.75                                | 0.02              | 0.02                     | 0.00                          |
| 31      | A136                            | B1:H1              | D1    | 41%                                      | 0.69                            | 0.75                                | 0.02              | 0.02                     | 0.00                          |
| 32      | A116                            | B1:H1              | D1    | 41%                                      | 0.52                            | 0.85                                | 0.03              | 0.03                     | 0.00                          |
| 33      | A119                            | B1:H1              | D1    | 41%                                      | 0.52                            | 0.85                                | 0.03              | 0.03                     | 0.00                          |
| 34      | A120                            | B1:H1              | D1    | 41%                                      | 0.52                            | 0.85                                | 0.03              | 0.03                     | 0.00                          |
| 35      | A124                            | B1:H1              | D1    | 41%                                      | 0.52                            | 0.85                                | 0.03              | 0.03                     | 0.00                          |
| 36      | A130                            | B1:H1              | D1    | 41%                                      | 0.52                            | 0.95                                | 0.04              | 0.05                     | 0.01                          |
| 37      | A156                            | B1:H1              | D1    | 41%                                      | 0.52                            | 0.95                                | 0.04              | 0.05                     | 0.01                          |
| 38      | A214                            | B1:H1              | D1    | 41%                                      | 0.52                            | 0.95                                | 0.04              | 0.05                     | 0.01                          |
| 39      | A310                            | B1:H1              | D1    | 41%                                      | 0.52                            | 0.95                                | 0.04              | 0.05                     | 0.01                          |
| 40      | A423                            | B1:H1              | D1    | 41%                                      | 0.52                            | 0.95                                | 0.04              | 0.05                     | 0.01                          |
| 41      | A523                            | B1:H1              | D1    | 41%                                      | 0.52                            | 0.95                                | 0.04              | 0.05                     | 0.01                          |
| 42      | A618                            | B1:H1              | D1    | 41%                                      | 0.52                            | 0.95                                | 0.04              | 0.05                     | 0.01                          |
| 43      | A731                            | B1:H1              | D1    | 41%                                      | 0.52                            | 0.95                                | 0.04              | 0.05                     | 0.01                          |
| 44      | A819                            | B1:H1              | D1    | 41%                                      | 0.52                            | 0.95                                | 0.04              | 0.05                     | 0.01                          |
| 45      | A919                            | B1:H1              | D1    | 41%                                      | 0.52                            | 0.95                                | 0.04              | 0.05                     | 0.01                          |
| 46      | A106                            | C1-3               | D1    | 57%                                      | 0.48                            | 0.65                                | 0.01              | 0.01                     | 0.00                          |
| 47      | A113                            | C1-3               | D1    | 57%                                      | 0.48                            | 0.65                                | 0.01              | 0.01                     | 0.00                          |
| 48      | A116                            | C1-3               | D1    | 57%                                      | 0.48                            | 0.65                                | 0.01              | 0.01                     | 0.00                          |
| 49      | A120                            | C1-3               | D1    | 57%                                      | 0.48                            | 0.65                                | 0.01              | 0.01                     | 0.00                          |
| 50      | A124                            | C1-3               | D1    | 57%                                      | 0.48                            | 0.65                                | 0.01              | 0.01                     | 0.00                          |

TABLE 11-continued

| Example | Electron Transporting Substance | Crosslinking Agent | Resin | Ratio of Electron Transporting Substance | Thickness of Undercoating Layer | R <sub>opt</sub> /R <sub>dark</sub> | Early-Stage Ghost | Ghost After 1,000 Sheets | Difference Between the Ghosts |
|---------|---------------------------------|--------------------|-------|------------------------------------------|---------------------------------|-------------------------------------|-------------------|--------------------------|-------------------------------|
| 51      | A136                            | C1-3               | D1    | 57%                                      | 0.48                            | 0.65                                | 0.01              | 0.01                     | 0.00                          |
| 52      | A136                            | C1-3               | D1    | 57%                                      | 0.15                            | 0.85                                | 0.02              | 0.02                     | 0.00                          |
| 53      | A136                            | C1-3               | D1    | 57%                                      | 0.65                            | 0.60                                | 0.01              | 0.01                     | 0.00                          |
| 54      | A136                            | C1-3               | D1    | 57%                                      | 0.75                            | 0.65                                | 0.01              | 0.01                     | 0.00                          |

TABLE 12

| Example                | Electron Transporting Substance | Crosslinking Agent         | Resin | Ratio of Electron Transporting Substance | Thickness of Undercoating Layer | R <sub>opt</sub> /R <sub>dark</sub> | Early-Stage Ghost | Ghost After 1,000 Sheets | Difference Between the Ghosts |
|------------------------|---------------------------------|----------------------------|-------|------------------------------------------|---------------------------------|-------------------------------------|-------------------|--------------------------|-------------------------------|
| 55                     | A136                            | C1-3                       | D1    | 57%                                      | 0.90                            | 0.75                                | 0.02              | 0.02                     | 0.00                          |
| 56                     | A136                            | C1-3                       | D1    | 57%                                      | 1.12                            | 0.77                                | 0.02              | 0.02                     | 0.00                          |
| 57                     | A136                            | C1-3                       | D1    | 57%                                      | 1.30                            | 0.80                                | 0.02              | 0.02                     | 0.00                          |
| 58                     | A201                            | C1-3                       | D1    | 57%                                      | 1.30                            | 0.85                                | 0.03              | 0.03                     | 0.00                          |
| 59                     | A306                            | C1-3                       | D1    | 57%                                      | 1.30                            | 0.85                                | 0.03              | 0.03                     | 0.00                          |
| 60                     | A306                            | C1-3                       | D1    | 57%                                      | 1.30                            | 0.75                                | 0.02              | 0.02                     | 0.00                          |
| 61                     | A404                            | C1-3                       | D1    | 57%                                      | 1.30                            | 0.75                                | 0.02              | 0.02                     | 0.00                          |
| 62                     | A510                            | C1-3                       | D1    | 57%                                      | 1.30                            | 0.75                                | 0.02              | 0.02                     | 0.00                          |
| 63                     | A602                            | C1-3                       | D1    | 57%                                      | 1.30                            | 0.85                                | 0.03              | 0.03                     | 0.00                          |
| 64                     | A709                            | C1-3                       | D1    | 57%                                      | 1.30                            | 0.85                                | 0.03              | 0.03                     | 0.00                          |
| 65                     | A807                            | C1-3                       | D1    | 57%                                      | 1.30                            | 0.75                                | 0.02              | 0.02                     | 0.00                          |
| 66                     | A902                            | C1-3                       | D1    | 57%                                      | 1.30                            | 0.75                                | 0.02              | 0.02                     | 0.00                          |
| 67                     | A101                            | B1:H2                      | D1    | 41%                                      | 0.40                            | 0.85                                | 0.03              | 0.03                     | 0.00                          |
| 68                     | A101                            | B1:H3                      | D1    | 41%                                      | 0.40                            | 0.85                                | 0.03              | 0.03                     | 0.00                          |
| 69                     | A101                            | B4:H1                      | D1    | 41%                                      | 0.40                            | 0.85                                | 0.03              | 0.03                     | 0.00                          |
| 70                     | A101                            | B5:H1                      | D1    | 41%                                      | 0.40                            | 0.85                                | 0.03              | 0.03                     | 0.00                          |
| 71                     | A101                            | B7:H1                      | D1    | 41%                                      | 0.40                            | 0.85                                | 0.03              | 0.03                     | 0.00                          |
| 72                     | A101                            | B12:H1                     | D1    | 41%                                      | 0.40                            | 0.85                                | 0.03              | 0.03                     | 0.00                          |
| 73                     | A101                            | C1-1                       | D1    | 57%                                      | 0.35                            | 0.75                                | 0.02              | 0.02                     | 0.00                          |
| 74                     | A101                            | C1-7                       | D1    | 57%                                      | 0.35                            | 0.75                                | 0.02              | 0.02                     | 0.00                          |
| 75                     | A101                            | C1-9                       | D1    | 41%                                      | 0.35                            | 0.75                                | 0.02              | 0.02                     | 0.00                          |
| 76                     | A101                            | C2-1                       | D1    | 41%                                      | 0.35                            | 0.75                                | 0.02              | 0.02                     | 0.00                          |
| 77                     | A101                            | C3-3                       | D1    | 41%                                      | 0.35                            | 0.75                                | 0.02              | 0.02                     | 0.00                          |
| 78                     | A101                            | B1:H1                      | D3    | 41%                                      | 0.26                            | 0.85                                | 0.03              | 0.03                     | 0.00                          |
| 79                     | A101                            | B1:H1                      | D5    | 41%                                      | 0.26                            | 0.85                                | 0.03              | 0.03                     | 0.00                          |
| 80                     | A101                            | B1:H1                      | D19   | 41%                                      | 0.26                            | 0.85                                | 0.03              | 0.03                     | 0.00                          |
| 81                     | A101                            | B1:H1                      | D20   | 41%                                      | 0.26                            | 0.85                                | 0.03              | 0.03                     | 0.00                          |
| 82                     | A124                            | C1-3                       | D1    | 65%                                      | 0.45                            | 0.65                                | 0.01              | 0.01                     | 0.00                          |
| 83                     | A130                            | C1-3                       | D1    | 65%                                      | 0.45                            | 0.65                                | 0.01              | 0.01                     | 0.00                          |
| 84                     | A156                            | C1-3                       | D1    | 65%                                      | 0.45                            | 0.65                                | 0.01              | 0.01                     | 0.00                          |
| 85                     | A125                            | C1-3                       | D1    | 70%                                      | 0.49                            | 0.65                                | 0.01              | 0.01                     | 0.00                          |
| 86                     | A125                            | C1-3                       | D1    | 72%                                      | 0.49                            | 0.75                                | 0.02              | 0.02                     | 0.00                          |
| 87                     | A125                            | C1-3                       | D1    | 70%                                      | 0.70                            | 0.75                                | 0.02              | 0.02                     | 0.00                          |
| 88                     | A125                            | C1-3                       | D1    | 70%                                      | 0.95                            | 0.75                                | 0.02              | 0.02                     | 0.00                          |
| 89                     | A125                            | C1-3                       | D1    | 70%                                      | 1.24                            | 0.80                                | 0.03              | 0.03                     | 0.00                          |
| 90                     | A101                            | B1:H1                      | D1    | 30%                                      | 0.53                            | 0.95                                | 0.04              | 0.05                     | 0.01                          |
| 91                     | A101                            | B1:H1                      | D1    | 33%                                      | 0.15                            | 0.85                                | 0.03              | 0.03                     | 0.00                          |
| 92                     | A101                            | B1:H1                      | D1    | 33%                                      | 0.53                            | 0.95                                | 0.04              | 0.05                     | 0.01                          |
| 93                     | A101                            | B1:H1                      | D1    | 33%                                      | 0.53                            | 0.85                                | 0.03              | 0.03                     | 0.00                          |
| Comparative Example 1  | A101                            | B1:H1                      | D1    | 20%                                      | 0.53                            | 0.99                                | 0.1               | 0.13                     | 0.03                          |
| Comparative Example 2  | A101                            | B1:H1                      | D1    | 25%                                      | 0.53                            | 0.98                                | 0.07              | 0.10                     | 0.03                          |
| Comparative Example 3  | A101                            | B1:H1                      | D1    | 25%                                      | 0.40                            | 0.98                                | 0.07              | 0.10                     | 0.03                          |
| Comparative Example 4  | A101                            | B1:H1                      | D1    | 25%                                      | 0.32                            | 0.97                                | 0.07              | 0.09                     | 0.02                          |
| Comparative Example 5  | A101                            | B1:H1                      | D1    | 33%                                      | 0.78                            | 0.98                                | 0.06              | 0.09                     | 0.03                          |
| Comparative Example 6  | A101                            | B1:H1                      | D1    | 33%                                      | 1.03                            | 0.99                                | 0.07              | 0.10                     | 0.03                          |
| Comparative Example 7  | A101                            | B1:H1                      | D1    | 33%                                      | 1.48                            | 1                                   | 0.09              | 0.13                     | 0.04                          |
| Comparative Example 8  | A101                            | hexamethylene diisocyanate | D1    | 36%                                      | 1.00                            | 0.99                                | 0.07              | 0.10                     | 0.03                          |
| Comparative Example 9  | A225                            | 2,4-toluene diisocyanate   | D1    | 50%                                      | 0.40                            | 0.99                                | 0.07              | 0.10                     | 0.03                          |
| Comparative Example 10 | A124                            | poly(p-hydroxystyrene)     |       |                                          |                                 |                                     |                   |                          |                               |

TABLE 12-continued

| Example                | Electron Transporting Substance | Crosslinking Agent       | Resin                  | Ratio of Electron Transporting Substance | Thickness of Undercoating Layer | R <sub>opt</sub> /R <sub>dark</sub> | Early-Stage Ghost | Ghost After 1,000 Sheets | Difference Between the Ghosts |
|------------------------|---------------------------------|--------------------------|------------------------|------------------------------------------|---------------------------------|-------------------------------------|-------------------|--------------------------|-------------------------------|
| Comparative Example 11 | A124                            | 2,4-toluene diisocyanate | poly(p-hydroxystyrene) | 70%                                      | 0.40                            | 0.98                                | 0.06              | 0.09                     | 0.03                          |

TABLE 13

| Example | Electron Transporting Substance | Crosslinking Agent | Resin | Ratio of Electron Transporting Substance | Thickness of Undercoating Layer | R <sub>opt</sub> /R <sub>dark</sub> | Early-Stage Ghost | Ghost After 1,000 Sheets | Difference Between the Ghosts |
|---------|---------------------------------|--------------------|-------|------------------------------------------|---------------------------------|-------------------------------------|-------------------|--------------------------|-------------------------------|
| 94      | A101                            | B1:H1              | D1    | 33%                                      | 0.53                            | 0.85                                | 0.03              | 0.03                     | 0.00                          |
| 95      | A106                            | B1:H6              | D14   | 33%                                      | 0.53                            | 0.85                                | 0.03              | 0.03                     | 0.00                          |
| 96      | A107                            | B1:H7              | D15   | 33%                                      | 0.53                            | 0.85                                | 0.04              | 0.04                     | 0.00                          |
| 97      | A157                            | B1:H5              | D25   | 41%                                      | 0.47                            | 0.80                                | 0.03              | 0.03                     | 0.00                          |
| 98      | A157                            | B1:H5              | D25   | 41%                                      | 0.47                            | 0.80                                | 0.03              | 0.03                     | 0.00                          |
| 99      | A157                            | B1:H5              | D25   | 41%                                      | 0.47                            | 0.80                                | 0.03              | 0.03                     | 0.00                          |
| 100     | A157                            | B1:H5              | D25   | 41%                                      | 0.47                            | 0.80                                | 0.04              | 0.04                     | 0.00                          |
| 101     | A124                            | B1:H5              | D25   | 41%                                      | 0.47                            | 0.80                                | 0.04              | 0.04                     | 0.00                          |
| 102     | A125                            | B1:H5              | D25   | 41%                                      | 0.47                            | 0.70                                | 0.03              | 0.03                     | 0.00                          |
| 103     | A152                            | B1:H5              | D25   | 41%                                      | 0.47                            | 0.85                                | 0.04              | 0.04                     | 0.00                          |
| 104     | A159                            | B1:H5              | D25   | 41%                                      | 0.47                            | 0.70                                | 0.03              | 0.03                     | 0.00                          |
| 105     | A164                            | B1:H5              | D25   | 41%                                      | 0.47                            | 0.65                                | 0.03              | 0.03                     | 0.00                          |
| 106     | A166                            | B1:H5              | D25   | 41%                                      | 0.47                            | 0.85                                | 0.04              | 0.04                     | 0.00                          |
| 107     | A167                            | B1:H5              | D25   | 41%                                      | 0.47                            | 0.80                                | 0.04              | 0.04                     | 0.00                          |
| 108     | A168                            | B1:H5              | D25   | 41%                                      | 0.47                            | 0.70                                | 0.03              | 0.03                     | 0.00                          |
| 109     | A172                            | B1:H5              | D25   | 41%                                      | 0.47                            | 0.75                                | 0.03              | 0.03                     | 0.00                          |
| 110     | A177                            | B1:H5              | D25   | 41%                                      | 0.47                            | 0.65                                | 0.03              | 0.03                     | 0.00                          |
| 111     | A178                            | B1:H5              | D25   | 41%                                      | 0.47                            | 0.65                                | 0.03              | 0.03                     | 0.00                          |
| 112     | A207                            | B1:H5              | D25   | 41%                                      | 0.47                            | 0.85                                | 0.04              | 0.04                     | 0.00                          |
| 113     | A315                            | B1:H5              | D25   | 41%                                      | 0.47                            | 0.85                                | 0.04              | 0.04                     | 0.00                          |
| 114     | A402                            | B1:H5              | D25   | 41%                                      | 0.47                            | 0.70                                | 0.03              | 0.03                     | 0.00                          |
| 115     | A509                            | B1:H5              | D25   | 41%                                      | 0.47                            | 0.70                                | 0.03              | 0.03                     | 0.00                          |
| 116     | A602                            | B1:H5              | D25   | 41%                                      | 0.47                            | 0.80                                | 0.04              | 0.04                     | 0.00                          |
| 117     | A707                            | B1:H5              | D25   | 41%                                      | 0.47                            | 0.65                                | 0.03              | 0.03                     | 0.00                          |
| 118     | A819                            | B1:H5              | D25   | 41%                                      | 0.47                            | 0.65                                | 0.03              | 0.03                     | 0.00                          |
| 119     | A908                            | B1:H5              | D25   | 41%                                      | 0.47                            | 0.70                                | 0.03              | 0.03                     | 0.00                          |

40

## Comparative Example 12

An electrophotographic photosensitive member was manufactured and evaluated as in Example 1, except for forming an electron transporting layer as follows. The results are shown in Table 14.

5 parts of the electron transporting substance (A922), 13.5 parts of an isocyanate compound (Sumidure 3173, made by Sumitomo Bayer Urethane Co., Ltd.), 10 parts of a butyral resin (BM-1, made by Sekisui Chemical Co., Ltd.) and 0.005 part of diocetyltin laurate as a catalyst were dissolved in a solvent of 120 parts of methyl ethyl ketone to thereby prepare a coating liquid for an electron transporting layer. The coating liquid for an electron transporting layer was immersion coated on the conductive layer, and the obtained coating film was heated for 60 min at 150° C. to be polymerized to thereby form an electron transporting layer having a thickness of 1.00  $\mu$ m.

## Comparative Example 13

An electrophotographic photosensitive member was manufactured and evaluated as in Example 1, except for forming an electron transporting layer as follows. The results are shown in Table 14.

5 parts of the electron transporting substance (A101) and 2.4 parts of a melamine resin (Yuban 20HS, made by Mitsui

Chemicals Inc.) were dissolved in a mixed solvent of 50 parts of tetrahydrofuran and 50 parts of methoxypropanol to thereby prepare a coating liquid for an electron transporting layer. The coating liquid for an electron transporting layer was immersion coated on the conductive layer, and the obtained coating film was heated for 60 min at 150° C. to be polymerized to thereby form an electron transporting layer having a thickness of 1.00  $\mu$ m.

50

## Comparative Example 14

An electrophotographic photosensitive member was manufactured and evaluated as in Comparative Example 12, except for altering the thickness of the electron transporting layer from 1.00  $\mu$ m to 0.50  $\mu$ m. The results are shown in Table 14.

## Comparative Example 15

An electrophotographic photosensitive member was manufactured and evaluated as in Comparative Example 12, except for altering the melamine resin (Yuban 20HS, made by Mitsui Chemicals Inc.) of the electron transporting layer to the phenol resin (Plyophen J-325, made by DIC Corporation). The results are shown in Table 14.

117

## Comparative Example 16

An electrophotographic photosensitive member was manufactured and evaluated as in Example 1, except for forming an electron transporting layer as follows. The results are shown in Table 14.

10 parts of a mixture of a compound having a structure represented by the following formula (12-1) and a compound having a structure represented by the following formula (12-2) was dissolved in a mixed solvent of 30 parts of N-methyl-2-pyrrolidone and 60 parts of cyclohexanone to thereby prepare a coating liquid for an electron transporting layer. The coating liquid for an electron transporting layer was immersion coated on the conductive layer, and the obtained coating film was heated for 30 min at 150° C. to be polymerized to thereby form an electron transporting layer having a structure represented by the following formula (12-3) and having a thickness of 0.20 μm.



## Comparative Examples 17 and 18

Electrophotographic photosensitive members were manufactured and evaluated as in Comparative Example 16, except for altering the thickness of the electron transporting layer from 0.20 μm to 0.30 μm and 0.60 μm. The results are shown in Table 14.

## Comparative Example 19

An electrophotographic photosensitive member was manufactured and evaluated as in Example 1, except for forming an electron transporting layer as follows. The results are shown in Table 14.

10 parts of an electron transporting substance represented by the following formula (13) was dissolved in 60 parts of toluene to thereby prepare a coating liquid for an electron transporting layer. The coating liquid for an electron transporting layer was immersion coated on the conductive layer, and the obtained coating film was irradiated with electron beams under the conditions of an acceleration voltage of 150

118

kV and an irradiation dose of 10 Mrad to be polymerized to thereby form an electron transporting layer having a thickness of 1.00 μm.



## Comparative Example 20

An electrophotographic photosensitive member was manufactured and evaluated as in Example 1, except for forming an electron transporting layer as follows. The results are shown in Table 14.

5 parts of the electron transporting substance represented by the above formula (13), 5 parts of trimethylolpropane triacrylate (Kayarad TMPTA, Nippon Kayaku Co., Ltd.) and 0.1 part of AIBN (2,2-azobisisobutyronitrile) were dissolved in 190 parts of tetrahydrofuran (THF) to thereby prepare a coating liquid for an electron transporting layer. The coating liquid for an electron transporting layer was immersion coated on the conductive layer, and the obtained coating film was heated for 30 min at 150° C. to be polymerized to thereby form an electron transporting layer having a thickness of 0.80 μm.

## Comparative Example 21

An electrophotographic photosensitive member was manufactured and evaluated as in Example 1, except for forming an electron transporting layer as follows. The results are shown in Table 14.

5 parts of the electron transporting substance represented by the above formula (13) and 5 parts of a compound represented by the following formula (14) were dissolved in 60 parts of toluene to thereby prepare a coating liquid for an electron transporting layer. The coating liquid for an electron transporting layer was immersion coated on the conductive layer, and the obtained coating film was irradiated with electron beams under the conditions of an acceleration voltage of 150 kV and an irradiation dose of 10 Mrad to be polymerized to thereby form an electron transporting layer having a thickness of 1.00 μm.

(14)



## Comparative Example 22

An electrophotographic photosensitive member was manufactured and evaluated as in Example 1, except for forming an electron transporting layer as follows. The results are shown in Table 14.

119

An electron transporting layer (a constitution of example 1 of National Publication of International Patent Application No. 2009-505156) was formed using a block copolymer represented by the following structure, blocked isocyanate and a vinyl chloride-vinyl acetate copolymer to thereby form an electron transporting layer having a thickness of 0.32  $\mu\text{m}$ .



## Comparative Example 23

An electrophotographic photosensitive member was manufactured and evaluated as in Example 1, except for forming an electron transporting layer as follows. The results are shown in Table 14.



5 parts of the electron transporting substance (A101) and 5 parts of a polycarbonate resin (Z200, made by Mitsubishi Gas Chemical Co., Inc.) were dissolved in a mixed solvent of 50 parts of dimethylacetamide and 50 parts of chlorobenzene to thereby prepare a coating liquid for an electron transporting layer. The coating liquid for an electron transporting layer was immersion coated on the conductive layer, and the obtained coating film was heated for 30 min at 120° C. to be polymerized to thereby form an electron transporting layer having a thickness of 1.00  $\mu\text{m}$ .

## Comparative Example 24

An electrophotographic photosensitive member was manufactured and evaluated as in Example 1, except for forming an electron transporting layer as follows. The results are shown in Table 14.

5 parts of an electron transporting substance (pigment) represented by the following structural formula (16) was added to a liquid in which 5 parts of the resin (D1) was dissolved in 200 parts of methyl ethyl ketone, and was subjected to a dispersion treatment for 3 hours using a sand mill

120

to thereby prepare a coating liquid for an electron transporting layer. The coating liquid for an electron transporting layer was immersion coated on the conductive layer, and the obtained coating film was heated for 10 min at 100° C. to thereby form an electron transporting layer having a thickness of 1.50  $\mu\text{m}$ .

(15)

## Comparative Example 25

An electrophotographic photosensitive member was manufactured and evaluated as in Example 1, except for forming an electron transporting layer as follows. The results are shown in Table 14.

An electron transporting layer was formed by using a coating liquid for an electron transporting layer in which a polymer of an electron transporting substance described in example 1 of Japanese Patent No. 4594444 was dissolved in a solvent, to thereby form an electron transporting layer having a thickness of 2.00  $\mu\text{m}$ .

## Comparative Example 26

An electrophotographic photosensitive member was manufactured and evaluated as in Example 1, except for forming an electron transporting layer as follows. The results are shown in Table 14.

An electron transporting layer was formed by using a particle of a copolymer containing an electron transporting substance described in example 1 of Japanese Patent No. 4,594,444, to thereby form an electron transporting layer having a thickness of 1.00  $\mu\text{m}$ .

## Comparative Example 27

An electrophotographic photosensitive member was manufactured and evaluated as in Example 1, except for forming an electron transporting layer as follows. The results are shown in Table 14.

An electron transporting layer (a constitution of example 1 of Japanese Patent Application Laid-Open No. 2006-030698) was formed by using a zinc oxide pigment having been subjected to a surface treatment with a silane coupling agent, alizarin (A922), a blocked isocyanate compound and a butyral resin, to thereby form an electron transporting layer of 25  $\mu\text{m}$ .

## Comparative Example 28

An electrophotographic photosensitive member was manufactured and evaluated as in Example 1, except for forming an electron transporting layer as follows. The results are shown in Table 14.

5 parts of a polyamide resin (N-methoxymethylated 6-nylon resin (trade name: Toresin EF-30T, made by Nagase ChemteX Corp., the degree of polymerization: 420, methoxymethylation ratio: 36.8%)) was dissolved in 100 parts of methanol and 100 parts of 1-butanol to thereby prepare a coating liquid for an undercoating layer. The coating liquid for an undercoating layer was immersion coated on the conductive layer, and the obtained coating film was dried at 100° C. for 10 min to thereby form an undercoating layer.

## Comparative Example 29

An electrophotographic photosensitive member was manufactured and evaluated as in Example 1, except for forming an electron transporting layer as follows. The results are shown in Table 14.

An electron transporting layer (undercoating layer using an electron transporting pigment, a polyvinyl butyral resin, and a curable electron transporting substance having an alkoxyisilyl group) described in example 25 of Japanese Patent Application Laid-Open No. H11-119458 was formed.

TABLE 14

|                           | Thickness of<br>Electron<br>Transporting<br>Layer | R <sub>opt</sub> /<br>R <sub>dark</sub> | Early-<br>Stage<br>Ghost | Ghost After<br>1,000 Sheets | Difference<br>Between<br>the Ghosts |
|---------------------------|---------------------------------------------------|-----------------------------------------|--------------------------|-----------------------------|-------------------------------------|
| Comparative<br>Example 12 | 1.00                                              | 0.99                                    | 0.10                     | 0.13                        | 0.03                                |
| Comparative<br>Example 13 | 1.00                                              | 1.00                                    | 0.07                     | 0.10                        | 0.03                                |
| Comparative<br>Example 14 | 0.50                                              | 1.00                                    | 0.06                     | 0.10                        | 0.04                                |
| Comparative<br>Example 15 | 1.00                                              | 1.01                                    | 0.08                     | 0.12                        | 0.04                                |
| Comparative<br>Example 16 | 0.20                                              | 0.99                                    | 0.07                     | 0.10                        | 0.03                                |
| Comparative<br>Example 17 | 0.30                                              | 0.99                                    | 0.07                     | 0.10                        | 0.03                                |
| Comparative<br>Example 18 | 0.60                                              | 1.00                                    | 0.08                     | 0.11                        | 0.03                                |
| Comparative<br>Example 19 | 1.00                                              | 0.99                                    | 0.09                     | 0.12                        | 0.03                                |
| Comparative<br>Example 20 | 0.80                                              | 0.99                                    | 0.09                     | 0.13                        | 0.04                                |
| Comparative<br>Example 21 | 1.00                                              | 0.99                                    | 0.10                     | 0.13                        | 0.03                                |
| Comparative<br>Example 22 | 0.32                                              | 0.99                                    | 0.07                     | 0.10                        | 0.03                                |

## TABLE 14-continued

|                           | Thickness of<br>Electron<br>Transporting<br>Layer | R <sub>opt</sub> /<br>R <sub>dark</sub> | Early-<br>Stage<br>Ghost | Ghost After<br>1,000 Sheets | Difference<br>Between<br>the Ghosts |
|---------------------------|---------------------------------------------------|-----------------------------------------|--------------------------|-----------------------------|-------------------------------------|
| Comparative<br>Example 23 | 1.00                                              | 0.99                                    | 0.09                     | 0.13                        | 0.04                                |
| Comparative<br>Example 24 | 1.50                                              | 1.00                                    | 0.10                     | 0.13                        | 0.03                                |
| Comparative<br>Example 25 | 2.00                                              | 1.02                                    | 0.10                     | 0.14                        | 0.04                                |
| Comparative<br>Example 26 | 1.00                                              | 1.10                                    | 0.11                     | 0.14                        | 0.03                                |
| Comparative<br>Example 27 | 25.00                                             | 1.05                                    | 0.11                     | 0.15                        | 0.04                                |
| Comparative<br>Example 28 | 0.80                                              | 1.10                                    | 0.05                     | 0.12                        | 0.07                                |
| Comparative<br>Example 29 | 3.00                                              | 0.99                                    | 0.06                     | 0.09                        | 0.03                                |

While the present invention has been described with reference to exemplary embodiments, it is to be understood that the invention is not limited to the disclosed exemplary embodiments. The scope of the following claims is to be accorded the broadest interpretation so as to encompass all such modifications and equivalent structures and functions.

This application claims the benefit of Japanese Patent Application No. 2012-147158, filed Jun. 29, 2012, Japanese Patent Application No. 2013-093091, filed Apr. 25, 2013, and Japanese Patent Application No. 2013-130014, filed Jun. 20, 2013, which are hereby incorporated by reference herein in their entirety.

What is claimed is:

- An electrophotographic photosensitive member comprising:  
a laminated body, and  
a hole transporting layer formed on the laminated body,  
wherein the laminated body comprises:  
a conductive support,  
an electron transporting layer formed on the support, and  
a charge generating layer formed on the electron transporting layer,  
wherein the electron transporting layer comprises a polymerized product of a composition comprising:  
an electron transporting substance having a polymerizable functional group,  
a crosslinking agent, and  
a thermoplastic resin having a polymerizable functional group,  
wherein the polymerizable functional group is a hydroxy group, a thiol group, an amino group, a carboxyl group, or a methoxy group,  
wherein a content of the electron transporting substance in the composition is 30% by mass or more and 70% by mass or less with respect to the total mass of the composition, and  
wherein the laminated body satisfies the following expression (1):  
$$R_{opt}/R_{dark} \leq 0.95 \quad (1)$$
  
where, in the expression (1),  
R<sub>opt</sub> represents impedance of the laminated body measured by the steps of:  
forming, on a surface of the charge generating layer, a circular-shaped gold electrode having a thickness of 300 nm and a diameter of 10 mm by sputtering, and  
applying, between the conductive support and the circular-shaped gold electrode, an alternating electric field hav-

## 123

ing a voltage of 100 mV and a frequency of 0.1 Hz while irradiating the surface of the charge generating layer with light having intensity of 30  $\mu\text{J}/\text{cm}^2\cdot\text{s}$ , and measuring the impedance,

and

R\_dark represents impedance of the laminated body measured by the steps of:

forming, on a surface of the charge generating layer, a circular-shaped gold electrode having a thickness of 300 nm and a diameter of 10 mm by sputtering, and applying, between the conductive support and the circular-shaped gold electrode, an alternating electric field having a voltage of 100 mV and a frequency of 0.1 Hz without irradiating the surface of the charge generating layer with light, and measuring the impedance.

2. The electrophotographic photosensitive member according to claim 1, wherein the laminated body satisfies the following expression (2):

$$0 < R_{\text{opt}}/R_{\text{dark}} \leq 0.85 \quad (2).$$

3. The electrophotographic photosensitive member according to claim 1, wherein the electron transporting layer has a thickness of 0.2  $\mu\text{m}$  or more and 0.7  $\mu\text{m}$  or less.

4. The electrophotographic photosensitive member according to claim 1, wherein the crosslinking agent is a compound having 3 to 6 groups of an isocyanate group, a

## 124

compound having 3 to 6 groups of a blocked isocyanate group or a compound having 3 to 6 groups of a monovalent group represented by  $-\text{CH}_2-\text{OR}^1$  ( $\text{R}^1$  represents an alkyl group).

5. The electrophotographic photosensitive member according to claim 1, wherein the charge generating layer comprises at least one charge generating substance selected from the group consisting of phthalocyanine pigments and azo pigments.

6. The electrophotographic photosensitive member according to claim 1, wherein the hole transporting layer comprises at least one hole transporting substance selected from the group consisting of triarylamine compounds, benzidine compounds and styryl compounds.

7. A process cartridge detachably attachable to a main body of an electrophotographic apparatus, wherein the process cartridge integrally supports:

the electrophotographic photosensitive member according to claim 1, and at least one unit selected from the group consisting of a charging unit, a developing unit, a transfer unit and a cleaning unit.

8. An electrophotographic apparatus comprising an electrophotographic photosensitive member according to claim 1, and a charging unit, a light irradiation unit, a developing unit and a transfer unit.

\* \* \* \* \*